

# United States Patent [19]

Ma et al.

[11] Patent Number: 4,902,360

[45] Date of Patent: Feb. 20, 1990

[54] PERMANENT MAGNET ALLOY FOR  
ELEVATED TEMPERATURE  
APPLICATIONS

[75] Inventors: Bao-Min Ma, Pittsburgh; Kalathur S. V. L. Narasimhan, Monroeville, both of Pa.

[73] Assignee: Crucible Materials Corporation, Pittsburgh, Pa.

[21] Appl. No.: 266,226

[22] Filed: Oct. 28, 1988

## Related U.S. Application Data

[63] Continuation of Ser. No. 10,738, Feb. 4, 1987, abandoned.

[51] Int. Cl.<sup>4</sup> ..... H01F 1/04

[52] U.S. Cl. ..... 148/302; 420/83;  
420/121

[58] Field of Search ..... 148/302; 420/83, 121

[56]

## References Cited

### U.S. PATENT DOCUMENTS

4,533,408 8/1985 Koon ..... 148/108

### FOREIGN PATENT DOCUMENTS

0101552 2/1984 European Pat. Off. ..... 148/302

0106948 5/1984 European Pat. Off. ..... 148/302

0108474 5/1984 European Pat. Off. ..... 148/302

0126179 11/1984 European Pat. Off. ..... 148/302

Primary Examiner—John P. Sheehan

Attorney, Agent, or Firm—Finnegan, Henderson, Farabow, Garrett & Dunner

[57]

## ABSTRACT

A permanent magnet alloy consisting essentially of R<sub>2</sub>Fe<sub>14</sub>B, wherein, R is a combination of rare earth elements consisting essentially of, in atomic percent, neodymium 3 to 11 and balance holmium. The alloy may include optional additions of the rare earth elements gadolinium up to 10%, terbium up to 15%, dysprosium up to 16%, erbium up to 18% and thulium up to 12%.

18 Claims, No Drawings

## PERMANENT MAGNET ALLOY FOR ELEVATED TEMPERATURE APPLICATIONS

This application is a continuation of application Ser. No. 010,738, filed February 4, 1987, abandoned.

### BACKGROUND OF THE INVENTION

It is known to use permanent magnet alloys, and particularly permanent magnet alloys embodying one or more rare earth elements with a transition element iron and boron, for applications requiring permanent magnet properties at elevated temperatures. Specifically in this regard, permanent magnets used in electric motors may encounter motor operating temperatures in excess of 150° C. The permanent magnet alloy R<sub>2</sub>Fe<sub>14</sub>B has a temperature dependence of magnetization of -0.08% to -0.12% per °C. over the temperature range of -50° C. to 150° C. Accordingly, this permanent magnet alloy is limited with respect to high-temperature applications, and particularly use in electric motors operating at temperatures in excess of 150° C. For practical applications, it is necessary that permanent magnet alloys at the maximum operating temperature exhibit a magnetization of 8000 Gauss.

### OBJECTS OF THE INVENTION

It is accordingly an object of the present invention to provide a permanent magnet alloy of a combination of rare earth elements, the transition element iron and boron with the alloy having improved magnetization at elevated temperatures.

A more specific object of the invention is to provide a permanent magnet alloy of a composition wherein the alloy is characterized by a low temperature coefficient of magnetization, e.g.,  $\alpha$  less than -0.01% over °C. over a temperature range of over -50° C. to 250° C., with a magnetization greater than 7500 Gauss at room temperature, e.g., 23 ± 2° C.

### SUMMARY OF THE INVENTION

The alloy composition is a combination of rare earth elements (R), in atomic percent, in combination with the base composition R<sub>2</sub>Fe<sub>14</sub>B. R is neodymium 3 to 11% and balance holmium. The following are preferred limits for Nd and Ho and also preferred additional and optional rare earth elements.

| Nd | 4-10  | 5-11  | 7-11  | 7-11  | 7-11  |
|----|-------|-------|-------|-------|-------|
| Ho | 83-96 | 76-94 | 78-90 | 75-95 | 82-92 |
| Tm | 0-13  | —     | —     | —     | —     |
| Er | —     | 0-18  | —     | —     | —     |
| Tb | —     | —     | 0-12  | —     | —     |
| Dy | —     | —     | —     | 0-15  | —     |
| Gd | —     | —     | —     | —     | 0-10  |
| Nd | 1-10  | 6-10  | 3-11  | 9-11  | 8-12  |
| Ho | 80-90 | 76-96 | 76-92 | 75-88 | 72-88 |
| Tb | 0-10  | —     | —     | 0-12  | —     |
| Gd | 0-4   | —     | —     | —     | 0-8   |
| Dy | —     | 0-8   | —     | 0-15  | 0-15  |
| Er | —     | 0-14  | 0-18  | —     | —     |
| Tm | —     | —     | 0-12  | —     | —     |

The permanent magnet alloy of the invention including optional additional rare earth elements satisfies the above-stated properties with respect to a low temperature coefficient of magnetization in combination with magnetization at room temperature sufficient to enable the permanent magnets made from the alloy to retain

sufficient magnetization for use at elevated temperatures.

This is achieved by combining the light rare earth element neodymium (Nd) with the heavy rare earth element holmium (Ho) with the transition element iron and boron. The heavy rare earth element provides the desired low temperature coefficient of magnetization ( $\alpha$ ) and neodymium provides the required high magnetization (M<sub>s</sub>). In this manner, as the operating temperature of the permanent magnet made from alloy is increased the base magnetization being at a relatively high level in combination with the temperature dependence or the temperature coefficient of magnetization, being low, permanent magnet properties are retained, specifically magnetization, at relatively high operating temperatures.

The permanent magnet alloy of the invention consists essentially of R<sub>2</sub>Fe<sub>14</sub>B wherein R is a combination of rare earth elements consisting essentially of, in atomic percent, Nd 3 to 11 and balance Ho.

The alloy may optionally contain the additional rare earth elements gadolinium (Gd) up to 10%; terbium (Tb) up to 15%; dysprosium (Dy) up to 16%; erbium (Er) up to 18%, and thulium (Tm) up to 12%. Ho is preferably within the range of 72 to 92%.

The temperature coefficient of magnetization or the temperature dependence of magnetization in alloys of neodymium and iron result from the thermal effects on the ordered magnetic moment of the Nd sublattice and the iron sublattice. The magnetic moment of the Nd sublattice decreases much more rapidly than that of the iron sublattice. This results in a strong temperature dependence of the combined magnetic moment of Nd and iron. Consequently, as is well recognized, this alloy is not suitable to provide a constant flux in the presence of temperature variations. Although with heavy rare earth elements, such as Gd, Tb, Dy, Ho, Er, Tm, and Yb, the rare earth sublattice likewise exhibits a decrease in magnetic moment with increased temperature. It has been found, however, in accordance with the present invention, that these moments oppose the larger moment of iron sublattices to result in enhancing the net moment of the alloy in the presence of temperature increases. It has further been found with respect to these alloys in accordance with the invention, that although this net improvement in magnetic moment is observed and achieved, the magnetization of these alloys is less than required for high temperature application. It is further been found in accordance with the invention that the magnetic moment may be increased by substituting part of the heavy rare earth element content with heavy rare earth-iron-boron alloys with neodymium alone or with one or more additional heavy rare earth elements. In this manner, the required combination of high magnetization and low temperature coefficient of magnetization is achieved. It is this combination of properties that is necessary for the production of useful permanent magnets for applications requiring the retention of magnetization at increased temperatures during application.

### DESCRIPTION OF THE PREFERRED EMBODIMENTS AND SPECIFIC EXAMPLES

The temperature dependence of magnetization ( $\alpha$ ) of the heavy rare earth-iron-boron alloys are shown in Table I.

TABLE I

| Alloy                              | Magnetization $M_s$ and Temperature Coefficient of Heavy Rare Earth $R_2Fe_{14}B$ Alloys* |                            | 5  |
|------------------------------------|-------------------------------------------------------------------------------------------|----------------------------|----|
|                                    | $M_s$<br>Bohr magneton/formula unit                                                       | (-50-200° C.)<br>% per °C. |    |
| Ho <sub>2</sub> Fe <sub>14</sub> B | 15.69                                                                                     | +0.016                     |    |
| Tb <sub>2</sub> Fe <sub>14</sub> B | 13.27                                                                                     | -0.007                     |    |
| Dy <sub>2</sub> Fe <sub>14</sub> B | 13.70                                                                                     | +0.007                     |    |
| Gd <sub>2</sub> Fe <sub>14</sub> B | 16.56                                                                                     | -0.053                     |    |
| Er <sub>2</sub> Fe <sub>14</sub> B | 17.54                                                                                     | -0.042                     | 10 |
| Tm <sub>2</sub> Fe <sub>14</sub> B | 21.80                                                                                     | -0.078                     |    |

\* $\alpha = (MT_2 - MT_1)/M_{T_1} \times (T_2 - T_1)$  in percent,  $M_{T_1}$  and  $M_{T_2}$  are the magnetizations at temperatures  $T_1$  and  $T_2$  respectively.

As may be seen from the data presented Table I, the alpha values for the alloys are in the desired range; however, magnetization ( $M_s$ ) is lower than required. This is the case with respect to the alloys containing the heavy rare earth elements Ho, Tb and Dy. For the alloys of Table I having the heavy rare earth elements Gd, Er and Tm, the  $M_s$  values are at acceptable levels but  $\alpha$  is not within the required range.

In accordance with the invention and to demonstrate the effect of Nd with respect to increasing  $M_s$ , Nd was added to the heavy rare earth element containing alloys of Table I. The results from the standpoint of the combination of  $M_s$  and alpha by the addition of Nd is shown by the data presented in Tables II through Tables VII.

TABLE II

| COMPO-<br>SITION | Magnetization and Temperature Coefficient of<br>(Nd <sub>1-x</sub> Tb <sub>x</sub> ) <sub>2</sub> Fe <sub>14</sub> B Alloys Where x = 0<br>to 100% |       |                 |                 | 30               |          |
|------------------|----------------------------------------------------------------------------------------------------------------------------------------------------|-------|-----------------|-----------------|------------------|----------|
|                  | W                                                                                                                                                  | X     | M(25C)<br>MB/FU | M(25C)<br>GAUSS | ALPHA<br>-50-200 | R SQUARE |
| 100              | 0                                                                                                                                                  | 32.60 | 14670           | -.099           | .967             |          |
| 98               | 2                                                                                                                                                  | 32.21 | 14496           | -.099           | .967             |          |
| 96               | 4                                                                                                                                                  | 31.83 | 14322           | -.098           | .967             |          |
| 94               | 6                                                                                                                                                  | 31.44 | 14148           | -.097           | .966             | 40       |
| 92               | 8                                                                                                                                                  | 31.05 | 13974           | -.097           | .966             |          |
| 90               | 10                                                                                                                                                 | 30.67 | 13800           | -.096           | .965             |          |
| 88               | 12                                                                                                                                                 | 30.28 | 13626           | -.095           | .965             |          |
| 86               | 14                                                                                                                                                 | 29.89 | 13452           | -.094           | .964             |          |
| 84               | 16                                                                                                                                                 | 29.51 | 13278           | -.093           | .964             |          |
| 82               | 18                                                                                                                                                 | 29.12 | 13104           | -.092           | .963             | 45       |
| 80               | 20                                                                                                                                                 | 28.73 | 12930           | -.091           | .963             |          |
| 78               | 22                                                                                                                                                 | 28.35 | 12756           | -.091           | .962             |          |
| 76               | 24                                                                                                                                                 | 27.96 | 12582           | -.090           | .961             |          |
| 74               | 26                                                                                                                                                 | 27.57 | 12408           | -.089           | .961             |          |
| 72               | 28                                                                                                                                                 | 27.19 | 12234           | -.088           | .960             |          |
| 70               | 30                                                                                                                                                 | 26.80 | 12060           | -.087           | .959             | 50       |
| 68               | 32                                                                                                                                                 | 26.41 | 11886           | -.085           | .958             |          |
| 66               | 34                                                                                                                                                 | 26.03 | 11713           | -.084           | .957             |          |
| 64               | 36                                                                                                                                                 | 25.64 | 11539           | -.083           | .956             |          |
| 62               | 38                                                                                                                                                 | 25.25 | 11365           | -.082           | .955             |          |
| 60               | 40                                                                                                                                                 | 24.87 | 11191           | -.081           | .954             |          |
| 58               | 42                                                                                                                                                 | 24.48 | 11017           | -.080           | .953             |          |
| 56               | 44                                                                                                                                                 | 24.09 | 10843           | -.078           | .952             | 55       |
| 54               | 46                                                                                                                                                 | 23.71 | 10669           | -.077           | .950             |          |
| 52               | 48                                                                                                                                                 | 23.32 | 10495           | -.075           | .949             |          |
| 50               | 50                                                                                                                                                 | 22.94 | 10321           | -.074           | .947             |          |
| 48               | 52                                                                                                                                                 | 22.55 | 10147           | -.073           | .945             |          |
| 46               | 54                                                                                                                                                 | 22.16 | 9973            | -.071           | .943             |          |
| 44               | 56                                                                                                                                                 | 21.78 | 9799            | -.069           | .941             | 60       |
| 42               | 58                                                                                                                                                 | 21.39 | 9625            | -.068           | .939             |          |
| 40               | 60                                                                                                                                                 | 21.00 | 9451            | -.066           | .936             |          |
| 38               | 62                                                                                                                                                 | 20.62 | 9277            | -.064           | .933             |          |
| 36               | 64                                                                                                                                                 | 20.23 | 9103            | -.062           | .929             |          |
| 34               | 66                                                                                                                                                 | 19.84 | 8929            | -.060           | .926             |          |
| 32               | 68                                                                                                                                                 | 19.46 | 8755            | -.058           | .921             | 65       |
| 30               | 70                                                                                                                                                 | 19.07 | 8581            | -.056           | .916             |          |
| 28               | 72                                                                                                                                                 | 18.68 | 8407            | -.054           | .910             |          |
| 26               | 74                                                                                                                                                 | 18.30 | 8233            | -.051           | .903             |          |
| 24               | 76                                                                                                                                                 | 17.91 | 8059            | -.049           | .895             |          |

TABLE II-continued

| Magnetization and Temperature Coefficient of<br>(Nd <sub>1-x</sub> Tb <sub>x</sub> ) <sub>2</sub> Fe <sub>14</sub> B Alloys Where x = 0<br>to 100% |     |     |        |        |         |      |
|----------------------------------------------------------------------------------------------------------------------------------------------------|-----|-----|--------|--------|---------|------|
| W % Nd <sub>2</sub> Fe <sub>14</sub> B + X % Tb <sub>2</sub> Fe <sub>14</sub> B                                                                    |     |     |        |        |         |      |
| COMPO-<br>SITION                                                                                                                                   | W   | X   | M(25C) | M(25C) | ALPHA   |      |
|                                                                                                                                                    |     |     | MB/FU  | GAUSS  | -50-200 |      |
| 10                                                                                                                                                 | 22  | 78  | 17.52  | 7885   | -.046   | .885 |
|                                                                                                                                                    | 20  | 80  | 17.14  | 7711   | -.044   | .873 |
|                                                                                                                                                    | 18  | 82  | 16.75  | 7537   | -.041   | .858 |
|                                                                                                                                                    | 16  | 84  | 16.36  | 7363   | -.038   | .839 |
|                                                                                                                                                    | 14  | 86  | 15.98  | 7189   | -.035   | .816 |
|                                                                                                                                                    | 12  | 88  | 15.59  | 7015   | -.032   | .785 |
|                                                                                                                                                    | 10  | 90  | 15.20  | 6841   | -.028   | .744 |
|                                                                                                                                                    | 8   | 92  | 14.82  | 6667   | -.024   | .689 |
|                                                                                                                                                    | 6   | 94  | 14.43  | 6493   | -.020   | .611 |
|                                                                                                                                                    | 4   | 96  | 14.04  | 6319   | -.016   | .501 |
| 15                                                                                                                                                 | 2   | 98  | 13.66  | 6145   | -.012   | .351 |
|                                                                                                                                                    | 0   | 100 | 13.27  | 5972   | -.007   | .167 |
| 20                                                                                                                                                 | 100 | 0   | 32.60  | 14670  | -.099   | .967 |
|                                                                                                                                                    | 98  | 2   | 32.28  | 14526  | -.099   | .967 |
|                                                                                                                                                    | 96  | 4   | 31.96  | 14381  | -.099   | .966 |
|                                                                                                                                                    | 94  | 6   | 31.64  | 14237  | -.098   | .966 |
|                                                                                                                                                    | 92  | 8   | 31.32  | 14093  | -.098   | .965 |
|                                                                                                                                                    | 90  | 10  | 31.00  | 13498  | -.097   | .965 |
|                                                                                                                                                    | 88  | 12  | 30.68  | 13626  | -.097   | .965 |
|                                                                                                                                                    | 86  | 14  | 30.35  | 13452  | -.096   | .964 |
|                                                                                                                                                    | 84  | 16  | 30.03  | 13515  | -.096   | .964 |
|                                                                                                                                                    | 82  | 18  | 29.71  | 13371  | -.095   | .963 |
| 25                                                                                                                                                 | 80  | 20  | 29.39  | 13227  | -.094   | .963 |
|                                                                                                                                                    | 78  | 22  | 29.07  | 13082  | -.094   | .962 |
|                                                                                                                                                    | 76  | 24  | 28.75  | 12938  | -.093   | .961 |
|                                                                                                                                                    | 74  | 26  | 28.43  | 12794  | -.093   | .961 |
|                                                                                                                                                    | 72  | 28  | 28.11  | 12649  | -.092   | .960 |
|                                                                                                                                                    | 70  | 30  | 27.79  | 12505  | -.091   | .959 |
|                                                                                                                                                    | 68  | 32  | 27.47  | 12361  | -.091   | .958 |
|                                                                                                                                                    | 66  | 34  | 27.15  | 12216  | -.090   | .958 |
|                                                                                                                                                    | 64  | 36  | 26.83  | 12072  | -.089   | .957 |
|                                                                                                                                                    | 62  | 38  | 26.51  | 11928  | -.089   | .956 |
| 30                                                                                                                                                 | 60  | 40  | 26.19  | 11784  | -.088   | .955 |
|                                                                                                                                                    | 58  | 42  | 25.86  | 11639  | -.087   | .954 |
|                                                                                                                                                    | 56  | 44  | 25.54  | 11495  | -.087   | .953 |
|                                                                                                                                                    | 54  | 46  | 25.22  | 11351  | -.086   | .952 |
|                                                                                                                                                    | 52  | 48  | 24.90  | 11206  | -.085   | .951 |
|                                                                                                                                                    | 50  | 50  | 24.58  | 11062  | -.084   | .949 |
|                                                                                                                                                    | 48  | 52  | 24.26  | 10918  | -.083   | .948 |
|                                                                                                                                                    | 46  | 54  | 23.94  | 10773  | -.083   | .947 |
|                                                                                                                                                    | 44  | 56  | 23.62  | 10629  | -.082   | .945 |
|                                                                                                                                                    | 42  | 58  | 23.30  | 10485  | -.081   | .944 |
| 35                                                                                                                                                 | 40  | 60  | 22.98  | 10340  | -.080   | .942 |
|                                                                                                                                                    | 38  | 62  | 22.66  | 10196  | -.079   | .940 |
|                                                                                                                                                    | 36  | 64  | 22.34  | 10052  | -.078   | .938 |
|                                                                                                                                                    | 34  | 66  | 22.02  | 9907   | -.077   | .936 |
|                                                                                                                                                    | 32  | 68  | 21.70  | 9763   | -.076   | .934 |
|                                                                                                                                                    | 30  | 70  | 21.37  | 9619   | -.075   | .931 |
|                                                                                                                                                    | 28  | 72  | 21.05  | 9474   | -.074   | .928 |
|                                                                                                                                                    | 26  | 74  | 20.73  | 9330   | -.072   | .926 |
|                                                                                                                                                    | 24  | 76  | 20.41  | 9186   | -.071   | .922 |
|                                                                                                                                                    | 22  | 78  | 20.09  | 9041   | -.070   | .919 |
| 40                                                                                                                                                 | 20  | 80  | 19.77  | 8897   | -.069   | .915 |
|                                                                                                                                                    | 18  | 82  | 19.45  | 8753   | -.068   | .911 |
|                                                                                                                                                    | 16  | 84  | 19.13  | 8608   | -.066   | .907 |
|                                                                                                                                                    | 14  | 86  | 18.81  | 8464   | -.065   | .902 |
|                                                                                                                                                    | 12  | 88  | 18.49  | 8320   | -.063   | .896 |
|                                                                                                                                                    | 10  | 90  | 18.17  | 8175   | -.063   | .890 |
|                                                                                                                                                    | 8   | 92  | 17.85  | 8031   | -.060   | .883 |
|                                                                                                                                                    | 6   | 94  | 17.53  | 7887   | -.059   | .875 |
|                                                                                                                                                    | 4   | 96  | 17.21  | 7742   | -.057   | .867 |
|                                                                                                                                                    | 2   | 98  | 16.88  | 7598   | -.055   | .857 |

TABLE III-continued

| Magnetization and Temperature Coefficient of<br>(Nd <sub>1-x</sub> Gd <sub>x</sub> ) <sub>2</sub> Fe <sub>14</sub> B Alloys Where x = 0<br>to 100% |     |        |        |         |          |    |
|----------------------------------------------------------------------------------------------------------------------------------------------------|-----|--------|--------|---------|----------|----|
| W % Nd <sub>2</sub> Fe <sub>14</sub> B + X % Gd <sub>2</sub> Fe <sub>14</sub> B                                                                    |     |        |        |         |          |    |
| COMPO-<br>SITION                                                                                                                                   |     | M(25C) | M(25C) | ALPHA   |          |    |
| W                                                                                                                                                  | X   | MB/FU  | GAUSS  | -50-200 | R SQUARE |    |
| 0                                                                                                                                                  | 100 | 16.56  | 7454   | -.053   | .846     | 10 |

TABLE IV

| Magnetization and Temperature Coefficient of<br>(Nd <sub>1-x</sub> Dy <sub>x</sub> ) <sub>2</sub> Fe <sub>14</sub> B Alloys Where x = 0<br>to 100% |     |        |        |         |          |    |
|----------------------------------------------------------------------------------------------------------------------------------------------------|-----|--------|--------|---------|----------|----|
| W % Nd <sub>2</sub> Fe <sub>14</sub> B + X % Dy <sub>2</sub> Fe <sub>14</sub> B                                                                    |     |        |        |         |          |    |
| COMPO-<br>SITION                                                                                                                                   |     | M(25C) | M(25C) | ALPHA   |          |    |
| W                                                                                                                                                  | X   | MB/FU  | GAUSS  | -50-200 | R SQUARE |    |
| 100                                                                                                                                                | 0   | 32.60  | 14670  | -.099   | .967     |    |
| 98                                                                                                                                                 | 2   | 32.21  | 14496  | -.099   | .966     |    |
| 96                                                                                                                                                 | 4   | 31.83  | 14322  | -.098   | .966     |    |
| 94                                                                                                                                                 | 6   | 31.44  | 14148  | -.097   | .965     |    |
| 92                                                                                                                                                 | 8   | 31.05  | 13974  | -.096   | .964     | 20 |
| 90                                                                                                                                                 | 10  | 30.67  | 13800  | -.095   | .963     |    |
| 88                                                                                                                                                 | 12  | 30.28  | 13626  | -.094   | .962     |    |
| 86                                                                                                                                                 | 14  | 29.89  | 13452  | -.093   | .961     |    |
| 84                                                                                                                                                 | 16  | 29.51  | 13278  | -.092   | .960     |    |
| 82                                                                                                                                                 | 18  | 29.12  | 13104  | -.091   | .958     |    |
| 80                                                                                                                                                 | 20  | 28.73  | 12930  | -.090   | .957     | 30 |
| 78                                                                                                                                                 | 22  | 28.35  | 12756  | -.089   | .956     |    |
| 76                                                                                                                                                 | 24  | 27.96  | 12582  | -.087   | .954     |    |
| 74                                                                                                                                                 | 26  | 27.57  | 12408  | -.086   | .953     |    |
| 72                                                                                                                                                 | 28  | 27.19  | 12234  | -.085   | .951     |    |
| 70                                                                                                                                                 | 30  | 26.80  | 12060  | -.084   | .949     | 35 |
| 68                                                                                                                                                 | 32  | 26.41  | 11886  | -.082   | .947     |    |
| 66                                                                                                                                                 | 34  | 26.03  | 11713  | -.081   | .945     |    |
| 64                                                                                                                                                 | 36  | 25.64  | 11539  | -.080   | .942     |    |
| 62                                                                                                                                                 | 38  | 25.25  | 11365  | -.078   | .940     |    |
| 60                                                                                                                                                 | 40  | 24.87  | 11191  | -.077   | .937     | 40 |
| 58                                                                                                                                                 | 42  | 24.48  | 11017  | -.075   | .934     |    |
| 56                                                                                                                                                 | 44  | 24.09  | 10843  | -.073   | .930     |    |
| 54                                                                                                                                                 | 46  | 23.71  | 10669  | -.072   | .926     |    |
| 52                                                                                                                                                 | 48  | 23.32  | 10495  | -.070   | .922     |    |
| 50                                                                                                                                                 | 50  | 22.94  | 10321  | -.068   | .917     |    |
| 48                                                                                                                                                 | 52  | 22.55  | 10147  | -.066   | .912     | 45 |
| 46                                                                                                                                                 | 54  | 22.16  | 9973   | -.064   | .906     |    |
| 44                                                                                                                                                 | 56  | 21.78  | 9799   | -.062   | .899     |    |
| 42                                                                                                                                                 | 58  | 21.39  | 9625   | -.060   | .892     |    |
| 40                                                                                                                                                 | 60  | 21.00  | 9421   | -.058   | .883     |    |
| 38                                                                                                                                                 | 62  | 20.62  | 9277   | -.056   | .873     |    |
| 36                                                                                                                                                 | 64  | 20.23  | 9103   | -.054   | .861     | 50 |
| 34                                                                                                                                                 | 66  | 19.84  | 8929   | -.051   | .847     |    |
| 32                                                                                                                                                 | 68  | 19.46  | 8755   | -.049   | .831     |    |
| 30                                                                                                                                                 | 70  | 19.07  | 8581   | -.046   | .812     |    |
| 28                                                                                                                                                 | 72  | 18.68  | 8407   | -.043   | .789     |    |
| 26                                                                                                                                                 | 74  | 18.30  | 8233   | -.040   | .761     | 55 |
| 24                                                                                                                                                 | 76  | 17.91  | 8059   | -.037   | .728     |    |
| 22                                                                                                                                                 | 78  | 17.52  | 7885   | -.034   | .686     |    |
| 20                                                                                                                                                 | 80  | 17.14  | 7711   | -.031   | .634     |    |
| 18                                                                                                                                                 | 82  | 16.75  | 7537   | -.027   | .570     |    |
| 16                                                                                                                                                 | 84  | 16.36  | 7363   | -.023   | .491     |    |
| 14                                                                                                                                                 | 86  | 15.98  | 7189   | -.020   | .395     |    |
| 12                                                                                                                                                 | 88  | 15.59  | 7015   | -.015   | .283     |    |
| 10                                                                                                                                                 | 90  | 15.20  | 6841   | -.011   | .164     |    |
| 8                                                                                                                                                  | 92  | 14.82  | 6667   | -.006   | .060     |    |
| 6                                                                                                                                                  | 94  | 14.43  | 6493   | -.001   | .003     |    |
| 4                                                                                                                                                  | 96  | 14.04  | 6319   | -.004   | .021     | 65 |
| 2                                                                                                                                                  | 98  | 13.66  | 6145   | -.009   | .110     |    |
| 0                                                                                                                                                  | 100 | 13.27  | 5972   | -.015   | .243     |    |

TABLE V

| Magnetization and Temperature Coefficient of<br>(Nd <sub>1-x</sub> Tm <sub>x</sub> ) <sub>2</sub> Fe <sub>14</sub> B Alloys Where x = 0<br>to 100% |     |        |        |         |          |  |
|----------------------------------------------------------------------------------------------------------------------------------------------------|-----|--------|--------|---------|----------|--|
| W % Nd <sub>2</sub> Fe <sub>14</sub> B + X % Tm <sub>2</sub> Fe <sub>14</sub> B                                                                    |     |        |        |         |          |  |
| COMPO-<br>SITION                                                                                                                                   |     | M(25C) | M(25C) | ALPHA   |          |  |
| W                                                                                                                                                  | X   | MB/FU  | GAUSS  | -50-200 | R SQUARE |  |
| 100                                                                                                                                                | 0   | 32.60  | 14670  | -.099   | .967     |  |
| 98                                                                                                                                                 | 2   | 32.38  | 14573  | -.099   | .965     |  |
| 96                                                                                                                                                 | 4   | 32.17  | 14476  | -.099   | .963     |  |
| 94                                                                                                                                                 | 6   | 31.95  | 14378  | -.099   | .961     |  |
| 92                                                                                                                                                 | 8   | 31.74  | 14281  | -.098   | .958     |  |
| 90                                                                                                                                                 | 10  | 31.52  | 14184  | -.098   | .955     |  |
| 88                                                                                                                                                 | 12  | 31.30  | 14087  | -.098   | .952     |  |
| 86                                                                                                                                                 | 14  | 31.09  | 13990  | -.097   | .949     |  |
| 84                                                                                                                                                 | 16  | 30.87  | 13892  | -.097   | .946     |  |
| 82                                                                                                                                                 | 18  | 30.66  | 13795  | -.097   | .943     |  |
| 80                                                                                                                                                 | 20  | 30.44  | 13698  | -.096   | .940     |  |
| 78                                                                                                                                                 | 22  | 30.22  | 13601  | -.096   | .936     |  |
| 76                                                                                                                                                 | 24  | 30.01  | 13504  | -.096   | .932     |  |
| 74                                                                                                                                                 | 26  | 29.79  | 13407  | -.095   | .928     |  |
| 72                                                                                                                                                 | 28  | 29.58  | 13309  | -.095   | .924     |  |
| 70                                                                                                                                                 | 30  | 29.36  | 13212  | -.095   | .919     |  |
| 68                                                                                                                                                 | 32  | 29.14  | 13115  | -.094   | .914     |  |
| 66                                                                                                                                                 | 34  | 28.93  | 13018  | -.094   | .910     |  |
| 64                                                                                                                                                 | 36  | 28.71  | 12921  | -.094   | .904     |  |
| 62                                                                                                                                                 | 38  | 28.50  | 12823  | -.093   | .899     |  |
| 60                                                                                                                                                 | 40  | 28.28  | 12726  | -.093   | .893     |  |
| 58                                                                                                                                                 | 42  | 28.06  | 12629  | -.093   | .887     |  |
| 56                                                                                                                                                 | 44  | 27.85  | 12535  | -.092   | .881     |  |
| 54                                                                                                                                                 | 46  | 27.63  | 12435  | -.092   | .875     |  |
| 52                                                                                                                                                 | 48  | 27.42  | 12337  | -.091   | .868     |  |
| 50                                                                                                                                                 | 50  | 27.20  | 12240  | -.091   | .861     |  |
| 48                                                                                                                                                 | 52  | 26.98  | 12143  | -.091   | .854     |  |
| 46                                                                                                                                                 | 54  | 26.77  | 12046  | -.090   | .847     |  |
| 44                                                                                                                                                 | 56  | 26.55  | 11949  | -.090   | .839     |  |
| 42                                                                                                                                                 | 58  | 26.34  | 11851  | -.089   | .831     |  |
| 40                                                                                                                                                 | 60  | 26.12  | 11754  | -.089   | .822     |  |
| 38                                                                                                                                                 | 62  | 25.90  | 11657  | -.088   | .813     |  |
| 36                                                                                                                                                 | 64  | 25.69  | 11650  | -.088   | .804     |  |
| 34                                                                                                                                                 | 66  | 25.47  | 11463  | -.088   | .795     |  |
| 32                                                                                                                                                 | 68  | 25.26  | 11366  | -.087   | .785     |  |
| 30                                                                                                                                                 | 70  | 25.04  | 11268  | -.087   | .775     |  |
| 28                                                                                                                                                 | 72  | 24.82  | 11171  | -.086   | .765     |  |
| 26                                                                                                                                                 | 74  | 24.61  | 11074  | -.086   | .754     |  |
| 24                                                                                                                                                 | 76  | 24.39  | 10977  | -.085   | .743     |  |
| 22                                                                                                                                                 | 78  | 24.18  | 10880  | -.085   | .732     |  |
| 20                                                                                                                                                 | 80  | 23.96  | 10782  | -.084   | .720     |  |
| 18                                                                                                                                                 | 82  | 23.74  | 10685  | -.084   | .708     |  |
| 16                                                                                                                                                 | 84  | 23.53  | 10588  | -.083   | .695     |  |
| 14                                                                                                                                                 | 86  | 23.31  | 10491  | -.082   | .683     |  |
| 12                                                                                                                                                 | 88  | 23.10  | 10394  | -.082   | .670     |  |
| 10                                                                                                                                                 | 90  | 22.88  | 10296  | -.081   | .656     |  |
| 8                                                                                                                                                  | 92  | 22.66  | 10199  | -.081   | .643     |  |
| 6                                                                                                                                                  | 94  | 22.45  | 10102  | -.080   | .629     |  |
| 4                                                                                                                                                  | 96  | 22.23  | 10005  | -.080   | .614     |  |
| 2                                                                                                                                                  | 98  | 22.02  | 9908   | -.079   | .600     |  |
| 0                                                                                                                                                  | 100 | 21.80  | 9810   | -.078   | .585     |  |

TABLE VI

| Magnetization and Temperature Coefficient of<br>(Nd <sub>1-x</sub> Er <sub>x</sub> ) <sub>2</sub> Fe <sub>14</sub> B Alloys Where x = 0<br>to 100% |    |        |        |         |          |  |
|----------------------------------------------------------------------------------------------------------------------------------------------------|----|--------|--------|---------|----------|--|
| W % Nd <sub>2</sub> Fe <sub>14</sub> B + X % Er <sub>2</sub> Fe <sub>14</sub> B                                                                    |    |        |        |         |          |  |
| COMPO-<br>SITION                                                                                                                                   |    | M(25C) | M(25C) | ALPHA   |          |  |
| W                                                                                                                                                  | X  | MB/FU  | GAUSS  | -50-200 | R SQUARE |  |
| 100                                                                                                                                                | 0  | 32.60  | 14670  | -.099   | .967     |  |
| 98                                                                                                                                                 | 2  | 32.30  | 14534  | -.099   | .965     |  |
| 96                                                                                                                                                 | 4  | 32.00  | 14399  | -.098   | .963     |  |
| 94                                                                                                                                                 | 6  | 31.70  | 14263  | -.098   | .961     |  |
| 92                                                                                                                                                 | 8  | 31.39  | 14128  | -.097   | .958     |  |
| 90                                                                                                                                                 | 10 | 31.09  | 13992  | -.096   | .956     |  |
| 88                                                                                                                                                 | 12 | 30.79  | 13857  | -.096   | .953     |  |
| 86                                                                                                                                                 | 14 | 30.49  | 13721  | -.095   | .950     |  |
| 84                                                                                                                                                 | 16 | 30.19  | 13585  | -.094   | .947     |  |
| 82                                                                                                                                                 | 18 | 29.89  | 13450  | -.094   | .943     |  |
| 80                                                                                                                                                 | 20 | 29.59  | 13314  | -.093   | .940     |  |

TABLE VI-continued

| Magnetization and Temperature Coefficient of<br>(Nd <sub>1-x</sub> Er <sub>x</sub> ) <sub>2</sub> Fe <sub>14</sub> B Alloys Where x = 0<br>to 100% |        |       |        |       |         |          |
|----------------------------------------------------------------------------------------------------------------------------------------------------|--------|-------|--------|-------|---------|----------|
| W % Nd <sub>2</sub> Fe <sub>14</sub> B + X % Er <sub>2</sub> Fe <sub>14</sub> B                                                                    |        |       |        |       |         |          |
| COMPO-<br>SITION                                                                                                                                   | M(25C) |       | M(25C) |       | ALPHA   |          |
|                                                                                                                                                    | W      | X     | MB/FU  | GAUSS | -50-200 | R SQUARE |
| 78                                                                                                                                                 | 22     | 29.29 | 13179  | -.092 | .936    |          |
| 76                                                                                                                                                 | 24     | 28.98 | 13043  | -.091 | .932    |          |
| 74                                                                                                                                                 | 26     | 28.68 | 12908  | -.091 | .927    |          |
| 72                                                                                                                                                 | 28     | 28.38 | 12772  | -.090 | .923    |          |
| 70                                                                                                                                                 | 30     | 28.08 | 12636  | -.089 | .918    |          |
| 68                                                                                                                                                 | 32     | 27.78 | 12501  | -.088 | .912    |          |
| 66                                                                                                                                                 | 34     | 27.48 | 12365  | -.087 | .906    |          |
| 64                                                                                                                                                 | 36     | 27.18 | 12230  | -.087 | .900    |          |
| 62                                                                                                                                                 | 38     | 26.88 | 12094  | -.086 | .893    |          |
| 60                                                                                                                                                 | 40     | 26.57 | 11958  | -.085 | .886    |          |
| 58                                                                                                                                                 | 42     | 26.27 | 11823  | -.084 | .879    |          |
| 56                                                                                                                                                 | 44     | 25.97 | 11867  | -.083 | .871    |          |
| 54                                                                                                                                                 | 46     | 25.67 | 11552  | -.082 | .862    |          |
| 52                                                                                                                                                 | 48     | 25.37 | 11416  | -.081 | .853    |          |
| 50                                                                                                                                                 | 50     | 25.07 | 11281  | -.080 | .843    |          |
| 48                                                                                                                                                 | 52     | 24.77 | 11145  | -.079 | .832    |          |
| 46                                                                                                                                                 | 54     | 24.47 | 11009  | -.078 | .821    |          |
| 44                                                                                                                                                 | 56     | 24.16 | 10874  | -.077 | .809    |          |
| 42                                                                                                                                                 | 58     | 23.86 | 10738  | -.076 | .796    |          |
| 40                                                                                                                                                 | 60     | 23.56 | 10603  | -.075 | .782    |          |
| 38                                                                                                                                                 | 62     | 23.26 | 10467  | -.073 | .767    |          |
| 36                                                                                                                                                 | 64     | 22.96 | 10332  | -.072 | .751    |          |
| 34                                                                                                                                                 | 66     | 22.66 | 10196  | -.071 | .735    |          |
| 32                                                                                                                                                 | 68     | 22.36 | 10060  | -.070 | .717    |          |
| 30                                                                                                                                                 | 70     | 22.06 | 9925   | -.068 | .698    |          |
| 28                                                                                                                                                 | 72     | 21.75 | 9789   | -.067 | .678    |          |
| 26                                                                                                                                                 | 74     | 21.45 | 9654   | -.066 | .656    |          |
| 24                                                                                                                                                 | 76     | 21.15 | 9518   | -.064 | .634    |          |
| 22                                                                                                                                                 | 78     | 20.85 | 9383   | -.063 | .610    |          |
| 20                                                                                                                                                 | 80     | 20.55 | 9247   | -.061 | .585    |          |
| 18                                                                                                                                                 | 82     | 20.25 | 9111   | -.059 | .559    |          |
| 16                                                                                                                                                 | 84     | 19.95 | 8976   | -.058 | .531    |          |
| 14                                                                                                                                                 | 86     | 19.64 | 8840   | -.056 | .502    |          |
| 12                                                                                                                                                 | 88     | 19.34 | 8705   | -.054 | .473    |          |
| 10                                                                                                                                                 | 90     | 19.04 | 8569   | -.053 | .442    |          |
| 8                                                                                                                                                  | 92     | 18.74 | 8434   | -.051 | .410    |          |
| 6                                                                                                                                                  | 94     | 18.44 | 8298   | -.049 | .378    |          |
| 4                                                                                                                                                  | 96     | 18.14 | 8162   | -.047 | .345    |          |
| 2                                                                                                                                                  | 98     | 17.84 | 8027   | -.045 | .312    |          |
| 0                                                                                                                                                  | 100    | 17.54 | 7891   | -.042 | .280    |          |

TABLE VII

| Magnetization and Temperature Coefficient of<br>(Nd <sub>1-x</sub> Ho <sub>x</sub> ) <sub>2</sub> Fe <sub>14</sub> B Alloys Where x = 0<br>to 100% |        |       |        |       |         |          |
|----------------------------------------------------------------------------------------------------------------------------------------------------|--------|-------|--------|-------|---------|----------|
| W % Nd <sub>2</sub> Fe <sub>14</sub> B + X % Ho <sub>2</sub> Fe <sub>14</sub> B                                                                    |        |       |        |       |         |          |
| COMPOSITION                                                                                                                                        | M(25C) |       | M(25C) |       | ALPHA   |          |
|                                                                                                                                                    | W      | X     | MB/FU  | GAUSS | -50-200 | R SQUARE |
| 100                                                                                                                                                | 0      | 32.60 | 14670  | -.099 | .967    |          |
| 98                                                                                                                                                 | 2      | 32.26 | 14518  | -.098 | .966    |          |
| 96                                                                                                                                                 | 4      | 31.92 | 14366  | -.097 | .965    |          |
| 94                                                                                                                                                 | 6      | 31.59 | 14213  | -.096 | .963    |          |
| 92                                                                                                                                                 | 8      | 31.25 | 14061  | -.095 | .962    |          |
| 90                                                                                                                                                 | 10     | 30.91 | 13909  | -.094 | .960    |          |
| 88                                                                                                                                                 | 12     | 30.57 | 13757  | -.093 | .959    |          |
| 86                                                                                                                                                 | 14     | 30.23 | 13604  | -.092 | .957    |          |
| 84                                                                                                                                                 | 16     | 29.89 | 13452  | -.091 | .955    |          |
| 82                                                                                                                                                 | 18     | 29.56 | 13300  | -.089 | .953    |          |
| 80                                                                                                                                                 | 20     | 29.22 | 13148  | -.088 | .951    |          |
| 78                                                                                                                                                 | 22     | 28.88 | 12996  | -.087 | .948    |          |
| 76                                                                                                                                                 | 24     | 28.54 | 12843  | -.085 | .946    |          |
| 74                                                                                                                                                 | 26     | 28.20 | 12691  | -.084 | .943    |          |
| 72                                                                                                                                                 | 28     | 27.86 | 12539  | -.083 | .940    |          |
| 70                                                                                                                                                 | 30     | 27.53 | 12387  | -.081 | .936    |          |
| 68                                                                                                                                                 | 32     | 27.19 | 12235  | -.080 | .933    |          |
| 66                                                                                                                                                 | 34     | 26.85 | 12082  | -.078 | .929    |          |
| 64                                                                                                                                                 | 36     | 26.51 | 11930  | -.077 | .924    |          |
| 62                                                                                                                                                 | 38     | 26.17 | 11778  | -.075 | .920    |          |
| 60                                                                                                                                                 | 40     | 25.83 | 11626  | -.073 | .914    |          |
| 58                                                                                                                                                 | 42     | 25.50 | 11473  | -.072 | .909    |          |
| 56                                                                                                                                                 | 44     | 25.16 | 11321  | -.070 | .902    |          |

TABLE VII-continued

| Magnetization and Temperature Coefficient of<br>(Nd <sub>1-x</sub> Ho <sub>x</sub> ) <sub>2</sub> Fe <sub>14</sub> B Alloys Where x = 0<br>to 100% |                                                                                 |   |        |       |         |          |       |
|----------------------------------------------------------------------------------------------------------------------------------------------------|---------------------------------------------------------------------------------|---|--------|-------|---------|----------|-------|
| 5                                                                                                                                                  | W % Nd <sub>2</sub> Fe <sub>14</sub> B + X % Ho <sub>2</sub> Fe <sub>14</sub> B |   |        |       |         |          |       |
|                                                                                                                                                    | COMPOSITION                                                                     |   | M(25C) |       | M(25C)  |          | ALPHA |
|                                                                                                                                                    | W                                                                               | X | MB/FU  | GAUSS | -50-200 | R SQUARE |       |
| 54                                                                                                                                                 | 46                                                                              |   | 24.82  | 11169 | -.068   | .895     |       |
| 52                                                                                                                                                 | 48                                                                              |   | 24.48  | 11017 | -.066   | .887     |       |
| 50                                                                                                                                                 | 50                                                                              |   | 24.14  | 10865 | -.064   | .878     |       |
| 48                                                                                                                                                 | 52                                                                              |   | 23.81  | 10712 | -.062   | .868     |       |
| 46                                                                                                                                                 | 54                                                                              |   | 23.47  | 10560 | -.060   | .857     |       |
| 44                                                                                                                                                 | 56                                                                              |   | 23.13  | 10408 | -.058   | .844     |       |
| 42                                                                                                                                                 | 58                                                                              |   | 22.79  | 10256 | -.056   | .830     |       |
| 40                                                                                                                                                 | 60                                                                              |   | 22.45  | 10103 | -.054   | .814     |       |
| 38                                                                                                                                                 | 62                                                                              |   | 22.11  | 9951  | -.051   | .795     |       |
| 36                                                                                                                                                 | 64                                                                              |   | 21.78  | 9799  | -.049   | .773     |       |
| 34                                                                                                                                                 | 66                                                                              |   | 21.44  | 9647  | -.047   | .748     |       |
| 32                                                                                                                                                 | 68                                                                              |   | 21.10  | 9495  | -.044   | .720     |       |
| 30                                                                                                                                                 | 70                                                                              |   | 20.76  | 9342  | -.041   | .686     |       |
| 28                                                                                                                                                 | 72                                                                              |   | 20.42  | 9190  | -.038   | .648     |       |
| 26                                                                                                                                                 | 74                                                                              |   | 20.08  | 9038  | -.036   | .603     |       |
| 24                                                                                                                                                 | 76                                                                              |   | 19.75  | 8886  | -.033   | .551     |       |
| 22                                                                                                                                                 | 78                                                                              |   | 19.41  | 8734  | -.029   | .491     |       |
| 20                                                                                                                                                 | 80                                                                              |   | 19.07  | 8581  | -.026   | .424     |       |
| 18                                                                                                                                                 | 82                                                                              |   | 18.73  | 8429  | -.023   | .349     |       |
| 16                                                                                                                                                 | 84                                                                              |   | 18.39  | 8277  | -.019   | .269     |       |
| 14                                                                                                                                                 | 86                                                                              |   | 18.05  | 8125  | -.016   | .187     |       |
| 12                                                                                                                                                 | 88                                                                              |   | 17.72  | 7972  | -.012   | .111     |       |
| 10                                                                                                                                                 | 90                                                                              |   | 17.38  | 7820  | -.008   | .049     |       |
| 8                                                                                                                                                  | 92                                                                              |   | 17.04  | 7668  | -.003   | .010     |       |
| 6                                                                                                                                                  | 94                                                                              |   | 16.70  | 7516  | .001    | .001     |       |
| 4                                                                                                                                                  | 96                                                                              |   | 16.36  | 7364  | .006    | .024     |       |
| 2                                                                                                                                                  | 98                                                                              |   | 16.03  | 7211  | .011    | .075     |       |
| 0                                                                                                                                                  | 100                                                                             |   | 15.69  | 7059  | .016    | .146     |       |

In Tables II through Tables VII it may be seen that complete replacement of the heavy rare earth element with Nd is not desirable as the resulting values are not within the required range. In addition, the values are not improved by the addition of Nd except for the relatively narrow ranges of Nd in combination with Ho in accordance with the composition limits of the invention.

It was additionally determined from an analysis of the magnetization curve as a function of temperature that a combination of two or more heavy rare earth elements with neodymium-iron-boron may provide optimum properties in accordance with the invention.

TABLE VIII

| Magnetization and Temperature Coefficient<br>of (NdDyHo) <sub>2</sub> Fe <sub>14</sub> B Alloys |                                                                                                                         |    |        |       |        |         |          |
|-------------------------------------------------------------------------------------------------|-------------------------------------------------------------------------------------------------------------------------|----|--------|-------|--------|---------|----------|
| 50                                                                                              | W % Dy <sub>2</sub> F <sub>14</sub> B + X % Nd <sub>2</sub> Fe <sub>14</sub> B + Y % Ho <sub>2</sub> FE <sub>14</sub> B |    |        |       |        |         |          |
|                                                                                                 | COMPOSITION                                                                                                             |    | M(25C) |       | M(25C) |         | ALPHA    |
|                                                                                                 | W                                                                                                                       | X  | Y      | MB/FU | GAUSS. | -50-200 | R SQUARE |
| 96                                                                                              | 4                                                                                                                       | 0  | 14.04  | 6319  | .004   | .021    |          |
| 86                                                                                              | 4                                                                                                                       | 10 | 14.28  | 6428  | .004   | .021    |          |
| 76                                                                                              | 4                                                                                                                       | 20 | 14.53  | 6537  | .004   | .022    |          |
| 66                                                                                              | 4                                                                                                                       | 30 | 14.77  | 6646  | .004   | .022    |          |
| 56                                                                                              | 4                                                                                                                       | 40 | 15.01  | 6755  | .005   | .022    |          |
| 46                                                                                              | 4                                                                                                                       | 50 | 15.25  | 6863  | .005   | .023    |          |
| 36                                                                                              | 4                                                                                                                       | 60 | 15.49  | 6972  | .005   | .023    |          |
| 26                                                                                              | 4                                                                                                                       | 70 | 15.74  | 7081  | .005   | .023    |          |
| 16                                                                                              | 4                                                                                                                       | 80 | 15.98  | 7190  | .005   | .024    |          |
| 6                                                                                               | 4                                                                                                                       | 90 | 16.22  | 7298  | .006   | .024    |          |
| 94                                                                                              | 6                                                                                                                       | 0  | 14.43  | 6493  | -.001  | .003    |          |
| 84                                                                                              | 6                                                                                                                       | 10 | 14.67  | 6602  | -.001  | .002    |          |
| 74                                                                                              | 6                                                                                                                       | 20 | 14.91  | 6711  | -.001  | .001    |          |
| 64                                                                                              | 6                                                                                                                       | 30 | 15.15  | 6820  | -.001  | .000    |          |
| 54                                                                                              | 6                                                                                                                       | 40 | 15.40  | 6928  | -.000  | .000    |          |
| 44                                                                                              | 6                                                                                                                       | 50 | 15.64  | 7037  | -.000  | .000    |          |
| 34                                                                                              | 6                                                                                                                       | 60 | 15.88  | 7146  | .000   | .000    |          |
| 24                                                                                              | 6                                                                                                                       | 70 | 16.12  | 7255  | .000   | .000    |          |
| 14                                                                                              | 6                                                                                                                       | 80 | 16.36  | 7364  | .001   | .000    |          |
| 4                                                                                               | 6                                                                                                                       | 90 | 16.61  | 7472  | .001   | .001    |          |
| 92                                                                                              | 8                                                                                                                       | 0  | 14.82  | 6667  | -.006  | .060    |          |
| 82                                                                                              | 8                                                                                                                       | 10 | 15.06  | 6776  | -.006  | .050    |          |

TABLE VIII-continued

| Magnetization and Temperature Coefficient of $(NdDyHo)_2Fe_{14}B$ Alloys |    |    |             |        |       |       |
|--------------------------------------------------------------------------|----|----|-------------|--------|-------|-------|
| W % $Dy_2Fe_{14}B$ + X % $Nd_2Fe_{14}B$ + Y % $Ho_2Fe_{14}B$             |    |    | COMPOSITION |        |       |       |
| W                                                                        | X  | Y  | M(25C)      | M(25C) | ALPHA |       |
|                                                                          |    |    | W           | X      | Y     | MB/FU |
|                                                                          |    |    |             |        |       | GAUSS |
| 72                                                                       | 8  | 20 | 15.30       | 6885   | -.006 | .041  |
| 62                                                                       | 8  | 30 | 15.54       | 6994   | -.005 | .034  |
| 52                                                                       | 8  | 40 | 15.78       | 7102   | -.005 | .028  |
| 42                                                                       | 8  | 50 | 16.02       | 7211   | -.005 | .023  |
| 32                                                                       | 8  | 60 | 16.27       | 7320   | -.004 | .019  |
| 22                                                                       | 8  | 70 | 16.51       | 7429   | -.004 | .015  |
| 12                                                                       | 8  | 80 | 16.75       | 7538   | -.004 | .013  |
| 2                                                                        | 8  | 90 | 16.99       | 7646   | -.003 | .010  |
| 90                                                                       | 10 | 0  | 15.20       | 6841   | -.011 | .164  |
| 80                                                                       | 10 | 10 | 15.44       | 6950   | -.011 | .143  |
| 70                                                                       | 10 | 20 | 15.69       | 7069   | -.010 | .125  |
| 60                                                                       | 10 | 30 | 15.93       | 7168   | -.010 | .109  |
| 50                                                                       | 10 | 40 | 16.17       | 7275   | -.009 | .095  |
| 40                                                                       | 10 | 50 | 16.41       | 7385   | -.009 | .083  |
| 30                                                                       | 10 | 60 | 16.65       | 7494   | -.009 | .073  |
| 20                                                                       | 10 | 70 | 17.14       | 7603   | -.008 | .064  |
| 10                                                                       | 10 | 80 | 17.14       | 7711   | -.008 | .056  |
| 0                                                                        | 10 | 90 | 17.38       | 7820   | -.008 | .049  |
| 88                                                                       | 12 | 0  | 15.59       | 7014   | -.015 | .283  |
| 78                                                                       | 12 | 10 | 15.83       | 7124   | -.015 | .254  |
| 68                                                                       | 12 | 20 | 16.07       | 7233   | -.014 | .228  |
| 58                                                                       | 12 | 30 | 16.31       | 7342   | -.014 | .205  |
| 48                                                                       | 12 | 40 | 16.56       | 7450   | -.014 | .184  |
| 38                                                                       | 12 | 50 | 16.80       | 7559   | -.013 | .166  |
| 28                                                                       | 12 | 60 | 17.04       | 7668   | -.013 | .149  |
| 18                                                                       | 12 | 70 | 17.28       | 7777   | -.012 | .134  |
| 8                                                                        | 12 | 80 | 17.52       | 7885   | -.012 | .121  |
| 86                                                                       | 14 | 0  | 15.98       | 7189   | -.020 | .395  |
| 76                                                                       | 14 | 10 | 16.22       | 7298   | -.019 | .363  |
| 66                                                                       | 14 | 20 | 16.46       | 7407   | -.019 | .333  |
| 56                                                                       | 14 | 30 | 16.70       | 7516   | -.018 | .305  |
| 46                                                                       | 14 | 40 | 16.94       | 7624   | -.018 | .280  |
| 36                                                                       | 14 | 50 | 17.18       | 7733   | -.017 | .256  |
| 26                                                                       | 14 | 60 | 17.43       | 7842   | -.017 | .235  |
| 16                                                                       | 14 | 70 | 17.67       | 7951   | -.016 | .215  |
| 6                                                                        | 14 | 80 | 17.91       | 8059   | -.016 | .197  |
| 84                                                                       | 16 | 0  | 16.36       | 7363   | -.023 | .491  |
| 74                                                                       | 16 | 10 | 16.60       | 7472   | -.023 | .459  |
| 64                                                                       | 16 | 20 | 16.85       | 7581   | -.022 | .428  |
| 54                                                                       | 16 | 30 | 17.09       | 7690   | -.022 | .399  |
| 44                                                                       | 16 | 40 | 17.33       | 7798   | -.021 | .371  |
| 34                                                                       | 16 | 50 | 17.57       | 7907   | -.021 | .345  |
| 24                                                                       | 16 | 60 | 17.81       | 8016   | -.020 | .321  |
| 14                                                                       | 16 | 70 | 18.05       | 8125   | -.020 | .298  |
| 4                                                                        | 16 | 80 | 18.30       | 8233   | -.019 | .277  |
| 82                                                                       | 18 | 0  | 16.75       | 7537   | -.027 | .570  |
| 72                                                                       | 18 | 10 | 16.99       | 7646   | -.027 | .539  |
| 62                                                                       | 18 | 20 | 17.23       | 7755   | -.026 | .509  |
| 52                                                                       | 18 | 30 | 17.47       | 7864   | -.025 | .480  |
| 42                                                                       | 18 | 40 | 17.72       | 7972   | -.025 | .453  |
| 32                                                                       | 18 | 50 | 17.96       | 8081   | -.024 | .426  |
| 22                                                                       | 18 | 60 | 18.20       | 8190   | -.024 | .401  |
| 12                                                                       | 18 | 70 | 18.44       | 8299   | -.023 | .376  |
| 2                                                                        | 18 | 80 | 18.68       | 8407   | -.023 | .354  |
| 80                                                                       | 20 | 0  | 17.14       | 7711   | -.031 | .634  |
| 70                                                                       | 20 | 10 | 17.38       | 7820   | -.030 | .606  |
| 60                                                                       | 20 | 20 | 17.62       | 7929   | -.029 | .578  |
| 50                                                                       | 20 | 30 | 17.86       | 8146   | -.029 | .550  |
| 40                                                                       | 20 | 40 | 18.10       | 8146   | -.028 | .523  |
| 30                                                                       | 20 | 50 | 18.34       | 8255   | -.028 | .497  |
| 20                                                                       | 20 | 60 | 18.59       | 8364   | -.027 | .472  |
| 10                                                                       | 20 | 70 | 18.83       | 8473   | -.027 | .447  |
| 0                                                                        | 20 | 80 | 19.07       | 8581   | -.026 | .424  |

As shown from Table VIII, by adding Nd to a combination of Ho and Dy in an iron-boron alloy both the alpha and  $M_s$  are achieved in combination only when Nd is within the range of 8 to 11%, Ho in the range of 75 to 92%, and Dy in the range of 0 to 15%.

TABLE IX

| Magnetization and Temperature Coefficient of $(NdDyTm)_2$ Alloys |    |    |             |        |       |       |
|------------------------------------------------------------------|----|----|-------------|--------|-------|-------|
| W % $Dy_2Fe_{14}B$ + X % $Nd_2Fe_{14}B$ + Y % $Tm_2Fe_{14}B$     |    |    | COMPOSITION |        |       |       |
| W                                                                | X  | Y  | M(25C)      | M(25C) | ALPHA |       |
|                                                                  |    |    | W           | X      | Y     | GAUSS |
| 96                                                               | 4  | 0  | 14.04       | 6319   | .004  | .021  |
| 86                                                               | 4  | 10 | 14.90       | 6703   | -.010 | .089  |
| 76                                                               | 4  | 20 | 15.75       | 7087   | -.022 | .259  |
| 10                                                               | 66 | 4  | 30          | 16.60  | 7471  | -.033 |
|                                                                  | 56 | 4  | 40          | 17.46  | 7855  | -.042 |
|                                                                  | 46 | 4  | 50          | 18.31  | 8239  | -.050 |
|                                                                  | 36 | 4  | 60          | 19.16  | 8623  | -.058 |
|                                                                  | 26 | 4  | 70          | 20.01  | 9007  | -.065 |
| 15                                                               | 16 | 4  | 80          | 20.87  | 9391  | -.071 |
|                                                                  | 94 | 6  | 90          | 21.72  | 9774  | -.076 |
|                                                                  | 84 | 6  | 10          | 21.43  | 6493  | -.001 |
|                                                                  | 74 | 6  | 20          | 22.11  | 6948  | -.014 |
|                                                                  | 64 | 6  | 30          | 22.84  | 7645  | -.036 |
| 20                                                               | 54 | 6  | 40          | 23.64  | 8029  | -.045 |
|                                                                  | 44 | 6  | 50          | 24.40  | 8413  | -.053 |
|                                                                  | 34 | 6  | 60          | 25.15  | 8797  | -.060 |
|                                                                  | 24 | 6  | 70          | 25.90  | 9181  | -.067 |
|                                                                  | 14 | 6  | 80          | 26.65  | 9565  | -.073 |
| 25                                                               | 62 | 8  | 90          | 27.40  | 7819  | -.039 |
|                                                                  | 52 | 8  | 10          | 28.11  | 8203  | -.048 |
|                                                                  | 42 | 8  | 20          | 28.84  | 9145  | -.065 |
|                                                                  | 32 | 8  | 30          | 29.59  | 9529  | -.071 |
|                                                                  | 22 | 8  | 40          | 30.34  | 9913  | -.076 |
| 30                                                               | 12 | 8  | 50          | 21.64  | 9739  | -.074 |
|                                                                  | 2  | 8  | 60          | 22.49  | 10122 | -.080 |
|                                                                  | 90 | 10 | 70          | 23.20  | 6841  | -.011 |
|                                                                  | 80 | 10 | 80          | 23.96  | 7225  | -.023 |
|                                                                  | 70 | 10 | 90          | 24.71  | 7609  | -.033 |
| 35                                                               | 60 | 10 | 10          | 25.46  | 7993  | -.042 |
|                                                                  | 50 | 10 | 20          | 26.21  | 8377  | -.050 |
|                                                                  | 40 | 10 | 30          | 26.97  | 8761  | -.058 |
|                                                                  | 30 | 10 | 40          | 27.72  | 9145  | -.065 |
|                                                                  | 20 | 10 | 50          | 28.47  | 9145  | -.065 |
| 40                                                               | 88 | 12 | 0           | 29.22  | 10296 | -.081 |
|                                                                  | 78 | 12 | 10          | 29.97  | 7015  | -.015 |
|                                                                  | 68 | 12 | 20          | 30.72  | 7399  | -.027 |
|                                                                  | 58 | 12 | 30          | 31.47  | 7783  | -.036 |
|                                                                  | 48 | 12 | 40          | 32.17  | 8167  | -.045 |
| 45                                                               | 38 | 12 | 50          | 32.87  | 8551  | -.053 |
|                                                                  | 28 | 12 | 60          | 33.57  | 8935  | -.060 |
|                                                                  | 18 | 12 | 70          | 34.27  | 9139  | -.067 |
|                                                                  | 8  | 12 | 80          | 34.97  | 9703  | -.073 |
|                                                                  | 78 | 12 | 90          | 35.67  | 10086 | -.078 |
| 50                                                               | 66 | 14 | 0           | 15.98  | 7189  | -.020 |
|                                                                  | 56 | 14 | 10          | 16.83  | 7573  | -.030 |
|                                                                  | 46 | 14 | 20          | 17.68  | 7957  | -.040 |
|                                                                  | 36 | 14 | 30          | 18.54  | 8341  | -.048 |
|                                                                  | 26 | 14 | 40          | 19.39  | 8725  | -.056 |
| 55                                                               | 56 | 14 | 50          | 20.24  | 9109  | -.062 |
|                                                                  | 46 | 14 | 60          | 21.09  | 9493  | -.069 |
|                                                                  | 36 | 14 | 70          | 21.95  | 9877  | -.074 |
|                                                                  | 26 | 14 | 80          | 22.80  | 10260 | -.080 |
|                                                                  | 16 | 14 | 90          | 23.55  | 10434 | -.081 |
| 60                                                               | 82 | 18 | 0           | 16.75  | 7537  | -.027 |
|                                                                  | 72 | 18 | 10          | 17.60  | 7921  | -.037 |
|                                                                  | 62 | 18 | 20          | 18.46  | 8305  | -.045 |
|                                                                  | 52 | 18 | 30          | 18.46  | 8689  | -.053 |
|                                                                  | 42 | 18 | 40          | 20.16  | 9073  | -.060 |
| 65                                                               | 32 | 18 | 50          | 21.01  | 9457  | -.067 |
|                                                                  | 22 | 18 | 60          | 21.87  | 9841  | -.072 |
|                                                                  | 12 | 18 | 70          | 22.72  | 10224 | -.078 |
|                                                                  | 2  | 18 | 80          | 23.57  | 10608 | -.083 |
|                                                                  | 72 | 18 | 90          | 24.32  | 10707 | -.087 |

TABLE IX-continued

| Magnetization and Temperature Coefficient of (NdDyTm) Alloys                                                             |    |    |             |       |         |          |
|--------------------------------------------------------------------------------------------------------------------------|----|----|-------------|-------|---------|----------|
| W % Dy <sub>2</sub> Fe <sub>14</sub> B + X % Nd <sub>2</sub> Fe <sub>14</sub> B + Y % Tm <sub>2</sub> Fe <sub>14</sub> B |    |    | COMPOSITION |       | M(25C)  | M(25C)   |
| W                                                                                                                        | X  | Y  | MB/FU       | GAUSS | -50-200 | R SQUARE |
| 80                                                                                                                       | 20 | 0  | 17.14       | 7711  | -.031   | .634     |
| 70                                                                                                                       | 20 | 10 | 17.99       | 8095  | -.040   | .668     |
| 60                                                                                                                       | 20 | 20 | 18.84       | 8479  | -.048   | .687     |
| 50                                                                                                                       | 20 | 30 | 19.70       | 8863  | -.056   | .698     |
| 40                                                                                                                       | 20 | 40 | 20.55       | 9247  | -.062   | .705     |
| 30                                                                                                                       | 20 | 50 | 21.40       | 9631  | -.069   | .710     |
| 20                                                                                                                       | 20 | 60 | 22.25       | 10015 | -.074   | .714     |
| 10                                                                                                                       | 20 | 70 | 23.11       | 10398 | -.079   | .717     |
| 0                                                                                                                        | 20 | 80 | 23.96       | 10782 | -.084   | .720     |

As may be seen from the data presented in Table IX where the Nd is alloyed with Dy and Tm within the cited ranges none of the alloys meet the desired combination of properties.

TABLE X

| Magnetization and Temperature Coefficient of (NdDyTb) <sub>2</sub> Fe <sub>14</sub> B Alloys                             |    |    |             |       |         |          |
|--------------------------------------------------------------------------------------------------------------------------|----|----|-------------|-------|---------|----------|
| W % Dy <sub>2</sub> Fe <sub>14</sub> B + X % Nd <sub>2</sub> Fe <sub>14</sub> B + Y % Tb <sub>2</sub> Fe <sub>14</sub> B |    |    | COMPOSITION |       | M(25C)  | M(25C)   |
| W                                                                                                                        | X  | Y  | MB/FU       | GAUSS | -50-200 | R SQUARE |
| 96                                                                                                                       | 4  | 0  | 14.04       | 6319  | .004    | .021     |
| 86                                                                                                                       | 4  | 10 | 14.04       | 6319  | -.002   | .004     |
| 76                                                                                                                       | 4  | 20 | 14.04       | 6319  | -.000   | .000     |
| 66                                                                                                                       | 4  | 30 | 14.04       | 6319  | -.003   | .013     |
| 56                                                                                                                       | 4  | 40 | 14.04       | 6319  | -.005   | .044     |
| 46                                                                                                                       | 4  | 50 | 14.04       | 6319  | -.007   | .097     |
| 36                                                                                                                       | 4  | 60 | 14.04       | 6319  | -.009   | .168     |
| 26                                                                                                                       | 4  | 70 | 14.04       | 6319  | -.011   | .254     |
| 16                                                                                                                       | 4  | 80 | 14.04       | 6319  | -.013   | .349     |
| 6                                                                                                                        | 4  | 90 | 14.04       | 6319  | -.015   | .445     |
| 94                                                                                                                       | 6  | 0  | 14.43       | 6493  | -.001   | .003     |
| 84                                                                                                                       | 6  | 10 | 14.43       | 6493  | -.004   | .020     |
| 74                                                                                                                       | 6  | 20 | 14.43       | 6493  | -.006   | .053     |
| 64                                                                                                                       | 6  | 30 | 14.43       | 6493  | -.008   | .102     |
| 54                                                                                                                       | 6  | 40 | 14.43       | 6493  | -.010   | .167     |
| 44                                                                                                                       | 6  | 50 | 14.43       | 6493  | -.012   | .244     |
| 34                                                                                                                       | 6  | 60 | 14.43       | 6493  | -.014   | .328     |
| 24                                                                                                                       | 6  | 70 | 14.43       | 6493  | -.016   | .416     |
| 14                                                                                                                       | 6  | 80 | 14.43       | 6493  | -.018   | .501     |
| 4                                                                                                                        | 6  | 90 | 14.43       | 6493  | -.020   | .581     |
| 92                                                                                                                       | 88 | 0  | 14.82       | 6667  | -.006   | .060     |
| 82                                                                                                                       | 8  | 10 | 14.82       | 6667  | -.008   | .106     |
| 72                                                                                                                       | 8  | 20 | 14.82       | 6667  | -.010   | .165     |
| 62                                                                                                                       | 8  | 30 | 14.82       | 6667  | -.012   | .235     |
| 52                                                                                                                       | 8  | 40 | 14.82       | 6667  | -.014   | .311     |
| 42                                                                                                                       | 8  | 50 | 14.82       | 6667  | -.016   | .390     |
| 32                                                                                                                       | 8  | 60 | 14.82       | 6667  | -.018   | .469     |
| 22                                                                                                                       | 8  | 70 | 14.82       | 6667  | -.020   | .545     |
| 12                                                                                                                       | 8  | 80 | 14.82       | 6667  | -.022   | .614     |
| 2                                                                                                                        | 8  | 90 | 14.82       | 6667  | -.024   | .677     |
| 90                                                                                                                       | 10 | 0  | 15.20       | 6841  | -.011   | .164     |
| 80                                                                                                                       | 10 | 10 | 15.20       | 6841  | -.013   | .227     |
| 70                                                                                                                       | 10 | 20 | 15.20       | 6841  | -.015   | .296     |
| 60                                                                                                                       | 10 | 30 | 15.20       | 6841  | -.017   | .368     |
| 50                                                                                                                       | 10 | 40 | 15.20       | 6841  | -.019   | .441     |
| 40                                                                                                                       | 10 | 50 | 15.20       | 6841  | -.021   | .512     |
| 30                                                                                                                       | 10 | 60 | 15.20       | 6841  | -.022   | .579     |
| 20                                                                                                                       | 10 | 70 | 15.20       | 6841  | -.024   | .640     |
| 10                                                                                                                       | 10 | 80 | 15.20       | 6841  | -.026   | .696     |
| 0                                                                                                                        | 10 | 90 | 15.20       | 6841  | -.028   | .744     |
| 88                                                                                                                       | 12 | 0  | 15.59       | 7015  | -.015   | .283     |
| 78                                                                                                                       | 12 | 10 | 15.59       | 7015  | -.017   | .349     |
| 68                                                                                                                       | 12 | 20 | 15.59       | 7015  | -.019   | .416     |
| 58                                                                                                                       | 12 | 30 | 15.59       | 7015  | -.021   | .483     |
| 48                                                                                                                       | 12 | 40 | 15.59       | 7015  | -.023   | .546     |
| 38                                                                                                                       | 12 | 50 | 15.59       | 7015  | -.025   | .606     |
| 28                                                                                                                       | 12 | 60 | 15.59       | 7015  | -.026   | .661     |
| 18                                                                                                                       | 12 | 70 | 15.59       | 7015  | -.028   | .710     |
| 8                                                                                                                        | 12 | 80 | 15.59       | 7015  | -.030   | .754     |
| 86                                                                                                                       | 14 | 0  | 15.98       | 7189  | -.020   | .395     |
| 76                                                                                                                       | 14 | 10 | 15.98       | 7189  | -.021   | .457     |
| 66                                                                                                                       | 14 | 20 | 15.98       | 7189  | -.023   | .517     |

TABLE X-continued

| Magnetization and Temperature Coefficient of (NdDyTb) <sub>2</sub> Fe <sub>14</sub> B Alloys                             |                                                                                     |    |             |       |         |          |
|--------------------------------------------------------------------------------------------------------------------------|-------------------------------------------------------------------------------------|----|-------------|-------|---------|----------|
| W % Dy <sub>2</sub> Fe <sub>14</sub> B + X % Nd <sub>2</sub> Fe <sub>14</sub> B + Y % Tb <sub>2</sub> Fe <sub>14</sub> B |                                                                                     |    | COMPOSITION |       | M(25C)  | M(25C)   |
| W                                                                                                                        | X                                                                                   | Y  | MB/FU       | GAUSS | -50-200 | R SQUARE |
| 56                                                                                                                       | 14                                                                                  | 30 | 15.98       | 7189  | -.025   | .575     |
| 46                                                                                                                       | 14                                                                                  | 40 | 15.98       | 7189  | -.027   | .628     |
| 36                                                                                                                       | 14                                                                                  | 50 | 15.98       | 7189  | -.028   | .677     |
| 10                                                                                                                       | 26                                                                                  | 14 | 60          | 15.98 | 7189    | -.030    |
| 16                                                                                                                       | 14                                                                                  | 70 | 15.98       | 7189  | -.032   | .762     |
| 6                                                                                                                        | 14                                                                                  | 80 | 15.98       | 7189  | -.034   | .797     |
| 84                                                                                                                       | 16                                                                                  | 0  | 16.36       | 7363  | -.023   | .491     |
| 74                                                                                                                       | 16                                                                                  | 10 | 16.36       | 7363  | -.025   | .546     |
| 64                                                                                                                       | 16                                                                                  | 20 | 16.36       | 7363  | -.027   | .598     |
| 54                                                                                                                       | 16                                                                                  | 30 | 16.36       | 7363  | -.029   | .647     |
| 44                                                                                                                       | 16                                                                                  | 40 | 16.36       | 7363  | -.030   | .691     |
| 34                                                                                                                       | 16                                                                                  | 50 | 16.36       | 7363  | -.032   | .732     |
| 24                                                                                                                       | 16                                                                                  | 60 | 16.36       | 7363  | -.034   | .768     |
| 14                                                                                                                       | 16                                                                                  | 70 | 16.36       | 7363  | -.036   | .800     |
| 4                                                                                                                        | 16                                                                                  | 80 | 16.36       | 7363  | -.037   | .829     |
| 82                                                                                                                       | 18                                                                                  | 0  | 16.75       | 7537  | -.027   | .570     |
| 72                                                                                                                       | 18                                                                                  | 10 | 16.75       | 7537  | -.029   | .618     |
| 62                                                                                                                       | 18                                                                                  | 20 | 16.75       | 7537  | -.031   | .662     |
| 52                                                                                                                       | 18                                                                                  | 30 | 16.75       | 7537  | -.032   | .703     |
| 42                                                                                                                       | 18                                                                                  | 40 | 16.75       | 7537  | -.034   | .740     |
| 32                                                                                                                       | 18                                                                                  | 50 | 16.75       | 7537  | -.036   | .773     |
| 22                                                                                                                       | 18                                                                                  | 60 | 16.75       | 7537  | -.037   | .803     |
| 12                                                                                                                       | 18                                                                                  | 70 | 16.75       | 7537  | -.039   | .830     |
| 2                                                                                                                        | 18                                                                                  | 80 | 16.75       | 7537  | -.041   | .854     |
| 80                                                                                                                       | 20                                                                                  | 0  | 17.14       | 7711  | -.031   | .634     |
| 70                                                                                                                       | 20                                                                                  | 10 | 17.14       | 7711  | -.032   | .675     |
| 60                                                                                                                       | 20                                                                                  | 20 | 17.14       | 7711  | -.034   | .712     |
| 50                                                                                                                       | 20                                                                                  | 30 | 17.14       | 7711  | -.036   | .746     |
| 40                                                                                                                       | 20                                                                                  | 40 | 17.14       | 7711  | -.037   | .777     |
| 30                                                                                                                       | 20                                                                                  | 50 | 17.14       | 7711  | -.039   | .805     |
| 20                                                                                                                       | 20                                                                                  | 60 | 17.14       | 7711  | -.041   | .831     |
| 10                                                                                                                       | 20                                                                                  | 70 | 17.14       | 7711  | -.042   | .853     |
| 0                                                                                                                        | 20                                                                                  | 80 | 17.14       | 7711  | -.044   | .873     |
| 35                                                                                                                       | This is also the case with respect to Table X wherein Nd is alloyed with Tb and Dy. |    |             |       |         |          |
| Magnetization and Temperature Coefficient of (NdDyGd) <sub>2</sub> Fe <sub>14</sub> B Alloys                             |                                                                                     |    |             |       |         |          |
| W % Dy <sub>2</sub> Fe <sub>14</sub> B + X % Nd <sub>2</sub> Fe <sub>14</sub> B + Y % Gd <sub>2</sub> Fe <sub>14</sub> B |                                                                                     |    | COMPOSITION |       | M(25C)  | M(25C)   |
| W                                                                                                                        | X                                                                                   | Y  | MB/FU       | GAUSS | -50-200 | R SQUARE |
| 96                                                                                                                       | 4                                                                                   | 0  | 14.04       | 6319  | .004    | .021     |
| 86                                                                                                                       | 4                                                                                   | 10 | 14.37       | 6468  | -.004   | .026     |
| 76                                                                                                                       | 4                                                                                   | 20 | 14.70       | 6616  | -.012   | .177     |
| 66                                                                                                                       | 4                                                                                   | 30 | 15.03       | 6764  | -.019   | .365     |
| 56                                                                                                                       | 4                                                                                   | 40 | 15.36       | 6912  | -.025   | .523     |
| 46                                                                                                                       | 4                                                                                   | 50 | 15.69       | 7061  | -.032   | .639     |
| 36                                                                                                                       | 4                                                                                   | 60 | 16.02       | 7209  | -.038   | .721     |
| 26                                                                                                                       | 4                                                                                   | 70 | 16.35       | 7357  | -.043   | .779     |
| 16                                                                                                                       | 4                                                                                   | 80 | 16.68       | 7505  | -.049   | .821     |
| 6                                                                                                                        | 4                                                                                   | 90 | 17.01       | 7654  | -.054   | .852     |
| 94                                                                                                                       | 6                                                                                   | 0  | 14.43       | 6493  | -.001   | .003     |
| 84                                                                                                                       | 6                                                                                   | 10 | 14.76       | 6642  | -.009   | .113     |
| 74                                                                                                                       | 6                                                                                   | 20 | 14.76       | 6642  | -.016   | .299     |
| 64                                                                                                                       | 6                                                                                   | 30 | 15.42       | 6938  | -.023   | .470     |
| 54                                                                                                                       | 6                                                                                   | 40 | 15.75       | 7086  | -.029   | .600     |
| 44                                                                                                                       | 6                                                                                   | 50 | 16.08       | 7235  | -.035   | .693     |
| 34                                                                                                                       | 6                                                                                   | 60 | 16.41       | 7383  | -.041   | .759     |
| 24                                                                                                                       | 6                                                                                   | 70 | 16.74       | 7531  | -.046   | .806     |
| 14                                                                                                                       | 6                                                                                   | 80 | 17.07       | 7679  | -.052   | .841     |
| 4                                                                                                                        | 6                                                                                   | 90 | 17.39       | 7827  | -.057   | .867     |
| 60                                                                                                                       | 92                                                                                  | 8  | 0           | 14.82 | 6667    | -.006    |
| 52                                                                                                                       | 8                                                                                   | 40 | 14.82       | 7260  | -.033   | .662     |
| 42                                                                                                                       | 8                                                                                   | 50 | 16.13       | 7409  | -.039   | .736     |
| 32                                                                                                                       | 8                                                                                   | 60 | 16.46       | 7557  | -.044   | .789     |
| 22                                                                                                                       | 8                                                                                   | 70 | 16.79       | 7705  | -.049   | .828     |
| 12                                                                                                                       | 8                                                                                   | 80 | 17.12       | 7853  | -.054   | .857     |
| 2                                                                                                                        | 8                                                                                   | 90 | 17.45       | 8001  | -.059   | .879     |
| 90                                                                                                                       | 10                                                                                  | 0  | 17.78       | 6841  | -.011   | .164     |

TABLE XI-continued

| Magnetization and Temperature Coefficient of $(NdDyGd)_2Fe_{14}B$ Alloys                                            |    |    |        |        |         |          |  |  |
|---------------------------------------------------------------------------------------------------------------------|----|----|--------|--------|---------|----------|--|--|
| <u>W % Dy<sub>2</sub>Fe<sub>14</sub>B + X % Nd<sub>2</sub>Fe<sub>14</sub>B + Y % Gd<sub>2</sub>Fe<sub>14</sub>B</u> |    |    |        |        |         |          |  |  |
| COMPOSITION                                                                                                         |    |    | M(25C) | M(25C) | ALPHA   |          |  |  |
| W                                                                                                                   | X  | Y  | MB/FU  | GAUSS  | -50-200 | R SQUARE |  |  |
| 80                                                                                                                  | 10 | 10 | 15.20  | 6990   | -.018   | .349     |  |  |
| 70                                                                                                                  | 10 | 20 | 15.53  | 7138   | -.024   | .508     |  |  |
| 60                                                                                                                  | 10 | 30 | 15.86  | 7286   | -.031   | .626     |  |  |
| 50                                                                                                                  | 10 | 40 | 16.19  | 7434   | -.036   | .710     |  |  |
| 40                                                                                                                  | 10 | 50 | 16.52  | 7583   | -.042   | .771     |  |  |
| 30                                                                                                                  | 10 | 60 | 16.85  | 7731   | -.047   | .814     |  |  |
| 20                                                                                                                  | 10 | 70 | 17.18  | 7879   | -.052   | .847     |  |  |
| 10                                                                                                                  | 10 | 80 | 17.51  | 8027   | -.057   | .871     |  |  |
| 0                                                                                                                   | 10 | 90 | 17.84  | 8175   | -.062   | .890     |  |  |
| 88                                                                                                                  | 12 | 0  | 18.17  | 7015   | -.015   | .283     |  |  |
| 78                                                                                                                  | 12 | 10 | 15.59  | 7164   | -.022   | .454     |  |  |
| 68                                                                                                                  | 12 | 20 | 15.92  | 7312   | -.028   | .586     |  |  |
| 58                                                                                                                  | 12 | 30 | 16.25  | 7460   | -.034   | .681     |  |  |
| 48                                                                                                                  | 12 | 40 | 16.58  | 7608   | -.040   | .749     |  |  |
| 38                                                                                                                  | 12 | 50 | 16.91  | 7756   | -.045   | .799     |  |  |
| 28                                                                                                                  | 12 | 60 | 17.24  | 7905   | -.050   | .835     |  |  |
| 18                                                                                                                  | 12 | 70 | 17.57  | 8053   | -.055   | .862     |  |  |
| 8                                                                                                                   | 12 | 80 | 17.90  | 8201   | -.060   | .883     |  |  |
| 86                                                                                                                  | 14 | 0  | 18.22  | 7189   | -.020   | .395     |  |  |
| 76                                                                                                                  | 14 | 10 | 15.98  | 7338   | -.026   | .541     |  |  |
| 66                                                                                                                  | 14 | 20 | 16.31  | 7486   | -.032   | .649     |  |  |
| 56                                                                                                                  | 14 | 30 | 16.64  | 7634   | -.037   | .726     |  |  |
| 46                                                                                                                  | 14 | 40 | 16.96  | 7782   | -.043   | .781     |  |  |
| 36                                                                                                                  | 14 | 50 | 17.29  | 7930   | -.048   | .822     |  |  |
| 26                                                                                                                  | 14 | 60 | 17.95  | 8079   | -.053   | .852     |  |  |
| 16                                                                                                                  | 14 | 70 | 18.28  | 8227   | -.058   | .875     |  |  |
| 6                                                                                                                   | 14 | 80 | 18.61  | 8375   | -.062   | .893     |  |  |
| 84                                                                                                                  | 16 | 0  | 16.36  | 7363   | -.023   | .491     |  |  |
| 74                                                                                                                  | 16 | 10 | 16.69  | 7511   | -.029   | .612     |  |  |
| 64                                                                                                                  | 16 | 20 | 17.02  | 7660   | -.035   | .699     |  |  |
| 54                                                                                                                  | 16 | 30 | 17.35  | 7808   | -.041   | .761     |  |  |
| 44                                                                                                                  | 16 | 40 | 17.68  | 7956   | -.046   | .807     |  |  |
| 34                                                                                                                  | 16 | 50 | 18.01  | 8104   | -.051   | .841     |  |  |
| 24                                                                                                                  | 16 | 60 | 18.34  | 8253   | -.056   | .866     |  |  |
| 14                                                                                                                  | 16 | 70 | 18.67  | 8401   | -.060   | .886     |  |  |
| 4                                                                                                                   | 16 | 80 | 19.00  | 8549   | -.064   | .901     |  |  |
| 82                                                                                                                  | 18 | 0  | 16.75  | 7537   | -.027   | .570     |  |  |
| 72                                                                                                                  | 18 | 10 | 17.08  | 7685   | -.033   | .668     |  |  |
| 62                                                                                                                  | 18 | 20 | 17.41  | 7834   | -.038   | .739     |  |  |
| 52                                                                                                                  | 18 | 30 | 17.74  | 7982   | -.044   | .790     |  |  |
| 42                                                                                                                  | 18 | 40 | 18.07  | 8130   | -.049   | .828     |  |  |
| 32                                                                                                                  | 18 | 50 | 18.40  | 8278   | -.054   | .856     |  |  |
| 22                                                                                                                  | 18 | 60 | 18.73  | 8427   | -.058   | .878     |  |  |
| 12                                                                                                                  | 18 | 70 | 19.06  | 8575   | -.062   | .895     |  |  |
| 2                                                                                                                   | 18 | 80 | 19.38  | 8723   | -.067   | .909     |  |  |
| 80                                                                                                                  | 20 | 0  | 17.14  | 7711   | -.031   | .634     |  |  |
| 70                                                                                                                  | 20 | 10 | 17.47  | 7859   | -.036   | .714     |  |  |
| 60                                                                                                                  | 20 | 20 | 17.79  | 8008   | -.042   | .772     |  |  |
| 50                                                                                                                  | 20 | 30 | 18.12  | 8156   | -.047   | .814     |  |  |
| 40                                                                                                                  | 20 | 40 | 18.45  | 8304   | -.051   | .846     |  |  |
| 30                                                                                                                  | 20 | 50 | 18.78  | 8452   | -.056   | .870     |  |  |
| 20                                                                                                                  | 20 | 60 | 19.11  | 8601   | -.060   | .889     |  |  |
| 10                                                                                                                  | 20 | 70 | 19.44  | 8749   | -.065   | .903     |  |  |
| 0                                                                                                                   | 20 | 80 | 19.77  | 8897   | -.069   | .915     |  |  |

The Table XI the alloy compositions embodying Dy and Gd with neodymium do not provide alloys that meet the desired combination of properties.

TABLE XII

| Magnetization and Temperature Coefficient of $(NdHoTm)_2Fe_{14}B$ Alloys                                            |   |    |        |        |         |          |  |  |
|---------------------------------------------------------------------------------------------------------------------|---|----|--------|--------|---------|----------|--|--|
| <u>W % Ho<sub>2</sub>Fe<sub>14</sub>B + X % Nd<sub>2</sub>Fe<sub>14</sub>B + Y % Tm<sub>2</sub>Fe<sub>14</sub>B</u> |   |    |        |        |         |          |  |  |
| COMPOSITION                                                                                                         |   |    | M(25C) | M(25C) | ALPHA   |          |  |  |
| W                                                                                                                   | X | Y  | MB/FU  | GAUSS  | -50-200 | R SQUARE |  |  |
| 96                                                                                                                  | 4 | 0  | 16.36  | 7364   | .006    | .024     |  |  |
| 86                                                                                                                  | 4 | 10 | 16.97  | 7639   | -.007   | .029     |  |  |
| 76                                                                                                                  | 4 | 20 | 17.59  | 7914   | -.018   | .150     |  |  |
| 66                                                                                                                  | 4 | 30 | 18.20  | 8189   | -.029   | .274     |  |  |
| 56                                                                                                                  | 4 | 40 | 18.81  | 8464   | -.038   | .371     |  |  |
| 46                                                                                                                  | 4 | 50 | 19.42  | 8739   | -.047   | .445     |  |  |
| 36                                                                                                                  | 4 | 60 | 20.03  | 9014   | -.055   | .500     |  |  |
| 26                                                                                                                  | 4 | 70 | 20.64  | 9289   | -.062   | .542     |  |  |

TABLE XII-continued

| Magnetization and Temperature Coefficient of $(NdHoTm)_2Fe_{14}B$ Alloys                                            |    |    |        |        |         |          |      |  |
|---------------------------------------------------------------------------------------------------------------------|----|----|--------|--------|---------|----------|------|--|
| <u>W % Ho<sub>2</sub>Fe<sub>14</sub>B + X % Nd<sub>2</sub>Fe<sub>14</sub>B + Y % Tm<sub>2</sub>Fe<sub>14</sub>B</u> |    |    |        |        |         |          |      |  |
| COMPOSITION                                                                                                         |    |    | M(25C) | M(25C) | ALPHA   |          |      |  |
| W                                                                                                                   | X  | Y  | MB/FU  | GAUSS  | -50-200 | R SQUARE |      |  |
| 16                                                                                                                  | 4  | 80 | 21.25  | 9565   | -.069   | .575     |      |  |
| 6                                                                                                                   | 4  | 90 | 21.87  | 9840   | -.076   | .601     |      |  |
| 94                                                                                                                  | 6  | 0  | 16.70  | 7516   | -.001   | .001     |      |  |
| 10                                                                                                                  | 84 | 6  | 10     | 17.31  | .7791   | -.011    | .074 |  |
| 74                                                                                                                  | 6  | 20 | 17.92  | 8066   | -.022   | .211     |      |  |
| 64                                                                                                                  | 6  | 30 | 18.54  | 8341   | -.032   | .329     |      |  |
| 54                                                                                                                  | 6  | 40 | 19.15  | 8616   | -.041   | .417     |      |  |
| 44                                                                                                                  | 6  | 50 | 19.76  | 8891   | -.050   | .482     |      |  |
| 34                                                                                                                  | 6  | 60 | 20.37  | 9167   | -.057   | .531     |      |  |
| 24                                                                                                                  | 6  | 70 | 20.98  | 9442   | -.065   | .568     |      |  |
| 14                                                                                                                  | 6  | 80 | 21.59  | 9717   | -.071   | .597     |      |  |
| 4                                                                                                                   | 6  | 90 | 22.20  | 9992   | -.078   | .621     |      |  |
| 92                                                                                                                  | 8  | 0  | 17.04  | 7668   | -.003   | .010     |      |  |
| 82                                                                                                                  | 8  | 10 | 17.65  | 7943   | -.015   | .133     |      |  |
| 72                                                                                                                  | 8  | 20 | 18.26  | 8218   | -.025   | .274     |      |  |
| 62                                                                                                                  | 8  | 30 | 18.87  | 8493   | -.035   | .382     |      |  |
| 52                                                                                                                  | 8  | 40 | 19.49  | 8769   | -.044   | .460     |      |  |
| 42                                                                                                                  | 8  | 50 | 20.10  | 9044   | -.052   | .518     |      |  |
| 32                                                                                                                  | 8  | 60 | 20.71  | 9319   | -.060   | .560     |      |  |
| 22                                                                                                                  | 8  | 70 | 21.32  | 9594   | -.067   | .593     |      |  |
| 12                                                                                                                  | 8  | 80 | 21.93  | 9869   | -.073   | .618     |      |  |
| 2                                                                                                                   | 8  | 90 | 22.54  | 10144  | -.080   | .639     |      |  |
| 90                                                                                                                  | 10 | 0  | 17.38  | 7820   | -.008   | .049     |      |  |
| 80                                                                                                                  | 10 | 10 | 17.99  | 8095   | -.019   | .201     |      |  |
| 70                                                                                                                  | 10 | 20 | 18.60  | 8370   | -.029   | .335     |      |  |
| 60                                                                                                                  | 10 | 30 | 19.21  | 8646   | -.038   | .432     |      |  |
| 50                                                                                                                  | 10 | 40 | 19.82  | 8921   | -.047   | .501     |      |  |
| 40                                                                                                                  | 10 | 50 | 20.44  | 9196   | -.055   | .550     |      |  |
| 30                                                                                                                  | 10 | 60 | 21.05  | 9471   | -.062   | .587     |      |  |
| 20                                                                                                                  | 10 | 70 | 21.66  | 9746   | -.069   | .616     |      |  |
| 10                                                                                                                  | 10 | 80 | 22.27  | 10021  | -.075   | .638     |      |  |
| 9                                                                                                                   | 10 | 90 | 22.88  | 10296  | -.081   | .656     |      |  |
| 8                                                                                                                   | 12 | 0  | 20.77  | 9348   | -.057   | .580     |      |  |
| 7                                                                                                                   | 12 | 10 | 18.33  | 8248   | -.022   | .272     |      |  |
| 6                                                                                                                   | 12 | 20 | 18.94  | 8523   | -.032   | .394     |      |  |
| 5                                                                                                                   | 12 | 30 | 19.55  | 8798   | -.041   | .478     |      |  |
| 4                                                                                                                   | 12 | 40 | 20.16  | 9073   | -.049   | .538     |      |  |
| 3                                                                                                                   | 12 | 50 | 20.77  | 9348   | -.057   | .580     |      |  |
| 2                                                                                                                   | 12 | 60 | 21.38  | 9623   | -.064   | .612     |      |  |
| 1                                                                                                                   | 12 | 70 | 22.00  | 9898   | -.071   | .637     |      |  |
| 45                                                                                                                  | 14 | 50 | 21.11  | 9500   | -.059   | .608     |      |  |
| 36                                                                                                                  | 14 | 60 | 21.72  | 9775   | -.066   | .636     |      |  |
| 26                                                                                                                  | 14 | 70 | 22.33  | 10051  | -.073   | .657     |      |  |
| 16                                                                                                                  | 14 | 80 | 22.95  | 10326  | -.079   | .674     |      |  |
| 8                                                                                                                   | 14 | 0  | 18.39  | 8277   | -.019   | .269     |      |  |
| 7                                                                                                                   | 14 | 10 | 19.00  | 8552   | -.029   | .408     |      |  |
| 6                                                                                                                   | 14 | 20 | 19.62  | 8827   | -.038   | .499     |      |  |
| 5                                                                                                                   | 14 | 30 | 20.23  | 9102   | -.047   | .560     |      |  |
| 4                                                                                                                   | 14 | 40 | 20.84  | 9377   | -.054   | .603     |      |  |
| 3                                                                                                                   | 14 | 50 | 21.45  | 9653   | -.062   | .634     |      |  |
| 2                                                                                                                   | 14 | 60 | 22.06  | 9928   | -.069   | .658     |      |  |
| 1                                                                                                                   | 14 | 70 | 22.67  | 10203  | -.075   | .676     |      |  |
| 45                                                                                                                  | 16 | 80 | 23.28  | 10478  | -.081   | .690     |      |  |
| 36                                                                                                                  | 16 | 0  | 18.73  | 8429   | -.023   | .349     |      |  |
| 27                                                                                                                  | 16 | 10 | 19.34  | 8704   | -.032   | .469     |      |  |
| 17                                                                                                                  | 16 | 20 | 19.95  | 8979   | -.041   | .545     |      |  |
| 8                                                                                                                   | 16 | 30 | 20.57  | 9254   | -.049   | .596     |      |  |
| 7                                                                                                                   | 16 | 40 | 21.18  | 9530   | -.057   | .632     |      |  |
| 6                                                                                                                   | 16 | 50 | 21.79  | 9805   | -.064   | .658     |      |  |
| 5                                                                                                                   | 16 | 60 | 22.40  | 10080  | -.071   | .678     |      |  |
| 4                                                                                                                   | 16 | 70 | 23.01  | 10355  | -.077   | .693     |      |  |
| 3                                                                                                                   | 16 | 80 | 23.62  | 10630  | -.082   | .706     |      |  |
| 2                                                                                                                   | 16 | 0  | 19.07  | 8581   | -.026   | .424     |      |  |
| 1                                                                                                                   | 16 | 10 | 19.68  | 8856   | -.035   | .523     |      |  |
| 36                                                                                                                  | 17 | 20 | 20.29  | 9132   | -.044   | .586     |      |  |
| 27                                                                                                                  | 17 | 30 | 20.90  |        |         |          |      |  |

TABLE XII-continued

| Magnetization and Temperature Coefficient of (NdHoTm) <sub>2</sub> Fe <sub>14</sub> B Alloys                             |    |        |        |       |         |          |
|--------------------------------------------------------------------------------------------------------------------------|----|--------|--------|-------|---------|----------|
| W % Ho <sub>2</sub> Fe <sub>14</sub> B + X % Nd <sub>2</sub> Fe <sub>14</sub> B + Y % Tm <sub>2</sub> Fe <sub>14</sub> B |    |        |        |       |         |          |
| COMPOSITION                                                                                                              |    | M(25C) | M(25C) | ALPHA |         |          |
| W                                                                                                                        | X  | Y      | MB/FU  | GAUSS | -50-200 | R SQUARE |
| 0                                                                                                                        | 20 | 80     | 23.96  | 10782 | -.084   | .720     |

As can be seen from the data presented in Table XII with neodymium within the range of 4 to 10%, Tm can be varied from 0 to 13% in combination with Nd and Ho within the range of 83 to 96% to achieve the desired combination of properties.

TABLE XIII

| Magnetization and Temperature Coefficient of (NdHoEr) <sub>2</sub> Fe <sub>14</sub> B Alloys                             |    |        |        |       |         |          |
|--------------------------------------------------------------------------------------------------------------------------|----|--------|--------|-------|---------|----------|
| W % Ho <sub>2</sub> Fe <sub>14</sub> B + X % Nd <sub>2</sub> Fe <sub>14</sub> B + Y % Er <sub>2</sub> Fe <sub>14</sub> B |    |        |        |       |         |          |
| COMPOSITION                                                                                                              |    | M(25C) | M(25C) | ALPHA |         |          |
| W                                                                                                                        | X  | Y      | MB/FU  | GAUSS | -50-200 | R SQUARE |
| 96                                                                                                                       | 4  | 0      | 16.36  | 7364  | .006    | .024     |
| 86                                                                                                                       | 4  | 10     | 16.55  | 7447  | -.001   | .000     |
| 76                                                                                                                       | 4  | 20     | 16.73  | 7530  | -.007   | .024     |
| 66                                                                                                                       | 4  | 30     | 16.92  | 7613  | -.012   | .070     |
| 56                                                                                                                       | 4  | 40     | 17.10  | 8305  | -.018   | .122     |
| 46                                                                                                                       | 4  | 50     | 17.29  | 7780  | -.024   | .173     |
| 36                                                                                                                       | 4  | 60     | 17.47  | 7863  | -.029   | .220     |
| 26                                                                                                                       | 4  | 70     | 17.66  | 7946  | -.034   | .261     |
| 16                                                                                                                       | 4  | 80     | 17.84  | 8029  | -.039   | .297     |
| 6                                                                                                                        | 4  | 90     | 18.03  | 8112  | -.044   | .328     |
| 94                                                                                                                       | 6  | 0      | 16.70  | 7516  | .001    | .001     |
| 84                                                                                                                       | 6  | 10     | 16.89  | 7599  | -.005   | .017     |
| 74                                                                                                                       | 6  | 20     | 17.07  | 7682  | -.011   | .064     |
| 64                                                                                                                       | 6  | 30     | 17.26  | 7765  | -.016   | .120     |
| 54                                                                                                                       | 6  | 40     | 17.44  | 7849  | -.022   | .176     |
| 44                                                                                                                       | 6  | 50     | 17.63  | 7932  | -.027   | .226     |
| 34                                                                                                                       | 6  | 60     | 17.81  | 8015  | -.032   | .269     |
| 24                                                                                                                       | 6  | 70     | 18.00  | 8098  | -.037   | .307     |
| 14                                                                                                                       | 6  | 80     | 18.18  | 8181  | -.042   | .340     |
| 4                                                                                                                        | 6  | 90     | 18.37  | 8265  | -.047   | .368     |
| 92                                                                                                                       | 8  | 0      | 17.04  | 7668  | -.003   | .010     |
| 82                                                                                                                       | 8  | 10     | 17.22  | 7751  | -.009   | .057     |
| 72                                                                                                                       | 8  | 20     | 17.41  | 7834  | -.015   | .118     |
| 62                                                                                                                       | 8  | 30     | 17.59  | 7918  | -.020   | .178     |
| 52                                                                                                                       | 8  | 40     | 17.78  | 8001  | -.026   | .232     |
| 42                                                                                                                       | 8  | 50     | 17.96  | 8084  | -.031   | .279     |
| 32                                                                                                                       | 8  | 60     | 18.15  | 8167  | -.036   | .318     |
| 22                                                                                                                       | 8  | 70     | 18.33  | 8250  | -.041   | .352     |
| 12                                                                                                                       | 8  | 80     | 18.52  | 8334  | -.045   | .381     |
| 2                                                                                                                        | 8  | 90     | 18.70  | 8417  | -.050   | .406     |
| 90                                                                                                                       | 10 | 0      | 17.38  | 7820  | -.008   | .049     |
| 80                                                                                                                       | 10 | 10     | 17.56  | 7903  | -.013   | .115     |
| 70                                                                                                                       | 10 | 20     | 17.75  | 7987  | -.019   | .181     |
| 60                                                                                                                       | 10 | 30     | 17.93  | 8070  | -.024   | .240     |
| 50                                                                                                                       | 10 | 40     | 18.12  | 8153  | -.029   | .289     |
| 40                                                                                                                       | 10 | 50     | 18.30  | 8236  | -.034   | .331     |
| 30                                                                                                                       | 10 | 60     | 18.49  | 8319  | -.039   | .366     |
| 20                                                                                                                       | 10 | 70     | 18.67  | 8403  | -.044   | .396     |
| 10                                                                                                                       | 10 | 80     | 18.86  | 8486  | -.048   | .421     |
| 0                                                                                                                        | 10 | 90     | 19.04  | 8569  | -.053   | .442     |
| 88                                                                                                                       | 12 | 0      | 17.72  | 7972  | -.012   | .111     |
| 78                                                                                                                       | 12 | 10     | 17.90  | 8056  | -.017   | .184     |
| 68                                                                                                                       | 12 | 20     | 18.09  | 8139  | -.022   | .248     |
| 58                                                                                                                       | 12 | 30     | 18.27  | 8222  | -.027   | .302     |
| 48                                                                                                                       | 12 | 40     | 18.46  | 8305  | -.032   | .345     |
| 38                                                                                                                       | 12 | 50     | 18.64  | 8388  | -.037   | .382     |
| 28                                                                                                                       | 12 | 60     | 18.83  | 8472  | -.042   | .412     |
| 18                                                                                                                       | 12 | 70     | 19.01  | 8555  | -.046   | .437     |
| 8                                                                                                                        | 12 | 80     | 19.20  | 8638  | -.051   | .458     |
| 86                                                                                                                       | 14 | 0      | 18.05  | 8125  | -.016   | .187     |
| 76                                                                                                                       | 14 | 10     | 18.24  | 8208  | -.021   | .258     |
| 66                                                                                                                       | 14 | 20     | 18.42  | 8291  | -.026   | .315     |
| 56                                                                                                                       | 14 | 30     | 18.61  | 8374  | -.031   | .362     |
| 46                                                                                                                       | 14 | 40     | 18.79  | 8457  | -.036   | .399     |
| 36                                                                                                                       | 14 | 50     | 18.98  | 8541  | -.040   | .429     |
| 26                                                                                                                       | 14 | 60     | 19.16  | 8624  | -.045   | .454     |
| 16                                                                                                                       | 14 | 70     | 19.35  | 8707  | -.049   | .475     |
| 6                                                                                                                        | 14 | 80     | 19.53  | 8790  | -.054   | .493     |
| 84                                                                                                                       | 16 | 0      | 18.39  | 8277  | -.019   | .269     |

TABLE XIII-continued

| Magnetization and Temperature Coefficient of (NdHoEr) <sub>2</sub> Fe <sub>14</sub> B Alloys                             |    |        |        |       |         |          |
|--------------------------------------------------------------------------------------------------------------------------|----|--------|--------|-------|---------|----------|
| W % Ho <sub>2</sub> Fe <sub>14</sub> B + X % Nd <sub>2</sub> Fe <sub>14</sub> B + Y % Er <sub>2</sub> Fe <sub>14</sub> B |    |        |        |       |         |          |
| COMPOSITION                                                                                                              |    | M(25C) | M(25C) | ALPHA |         |          |
| W                                                                                                                        | X  | Y      | MB/FU  | GAUSS | -50-200 | R SQUARE |
| 74                                                                                                                       | 16 | 10     | 18.58  | 8360  | -.024   | .331     |
| 64                                                                                                                       | 16 | 20     | 18.76  | 8443  | -.029   | .380     |
| 54                                                                                                                       | 16 | 30     | 18.95  | 8527  | -.034   | .418     |
| 44                                                                                                                       | 16 | 40     | 19.13  | 8610  | -.039   | .449     |
| 34                                                                                                                       | 16 | 50     | 19.32  | 8693  | -.043   | .474     |
| 24                                                                                                                       | 16 | 60     | 19.50  | 8776  | -.048   | .494     |
| 14                                                                                                                       | 16 | 70     | 19.69  | 8859  | -.052   | .511     |
| 4                                                                                                                        | 16 | 80     | 19.87  | 8943  | -.056   | .526     |
| 82                                                                                                                       | 18 | 0      | 18.73  | 8429  | -.023   | .349     |
| 72                                                                                                                       | 18 | 10     | 18.92  | 8512  | -.028   | .401     |
| 62                                                                                                                       | 18 | 20     | 19.10  | 8596  | -.032   | .440     |
| 52                                                                                                                       | 18 | 30     | 19.29  | 8679  | -.037   | .471     |
| 42                                                                                                                       | 18 | 40     | 19.47  | 8762  | -.042   | .495     |
| 32                                                                                                                       | 18 | 50     | 19.66  | 8845  | -.046   | .515     |
| 22                                                                                                                       | 18 | 60     | 19.84  | 8928  | -.050   | .531     |
| 12                                                                                                                       | 18 | 70     | 20.03  | 9012  | -.055   | .545     |
| 2                                                                                                                        | 18 | 80     | 20.21  | 9095  | -.059   | .557     |
| 80                                                                                                                       | 20 | 0      | 19.07  | 8581  | -.026   | .424     |
| 70                                                                                                                       | 20 | 10     | 19.25  | 8665  | -.031   | .464     |
| 60                                                                                                                       | 20 | 20     | 19.44  | 8748  | -.036   | .495     |
| 50                                                                                                                       | 20 | 30     | 19.62  | 8831  | -.040   | .519     |
| 40                                                                                                                       | 20 | 40     | 19.81  | 8914  | -.045   | .538     |
| 30                                                                                                                       | 20 | 50     | 19.99  | 8997  | -.049   | .553     |
| 20                                                                                                                       | 20 | 60     | 20.18  | 9081  | -.053   | .565     |
| 10                                                                                                                       | 20 | 70     | 20.36  | 9164  | -.057   | .576     |
| 0                                                                                                                        | 20 | 80     | 20.55  | 9247  | -.061   | .585     |

As may be seen from the data presented in this Table, if Nd varies from 5 to 11%, Er from 0 and Ho from 76 to 94%, the alloys meet the desired combination of properties.

TABLE XIV

| Magnetization and Temperature Coefficient of (NdHoTb) <sub>2</sub> Fe <sub>14</sub> B Alloys                             |    |        |        |       |         |          |
|--------------------------------------------------------------------------------------------------------------------------|----|--------|--------|-------|---------|----------|
| W % Ho <sub>2</sub> Fe <sub>14</sub> B + X % Nd <sub>2</sub> Fe <sub>14</sub> B + Y % Tb <sub>2</sub> Fe <sub>14</sub> B |    |        |        |       |         |          |
| COMPOSITION                                                                                                              |    | M(25C) | M(25C) | ALPHA |         |          |
| W                                                                                                                        | X  | Y      | MB/FU  | GAUSS | -50-200 | R SQUARE |
| 96                                                                                                                       | 4  | 0      | 16.36  | 7364  | .006    | .024     |
| 86                                                                                                                       | 4  | 10     | 16.12  | 7255  | .004    | .011     |
| 76                                                                                                                       | 4  | 20     | 15.88  | 7146  | .002    | .002     |
| 66                                                                                                                       | 4  | 30     | 15.64  | 7037  | -.001   | .000     |
| 56                                                                                                                       | 4  | 40     | 15.40  | 6929  | -.003   | .010     |
| 46                                                                                                                       | 4  | 50     | 15.16  | 6820  | -.005   | .037     |
| 36                                                                                                                       | 4  | 60     | 14.91  | 6711  | -.007   | .087     |
| 26                                                                                                                       | 4  | 70     | 14.67  | 6602  | -.010   | .167     |
| 16                                                                                                                       | 4  | 80     | 14.43  | 6493  | -.012   | .278     |
| 6                                                                                                                        | 4  | 90     | 14.19  | 6385  | -.015   | .414     |
| 94                                                                                                                       | 6  | 0      | 16.70  | 7516  | .001    | .001     |
| 84                                                                                                                       | 6  | 10     | 16.46  | 7407  | -.001   | .001     |
| 74                                                                                                                       | 6  | 20     | 16.22  | 7298  | -.003   | .010     |
| 64                                                                                                                       | 6  | 30     | 15.98  | 7190  | -.005   | .031     |
| 54                                                                                                                       | 6  | 40     | 15.73  | 7081  | -.008   | .069     |
| 44                                                                                                                       | 6  | 50     | 15.49  | 6972  | -.010   | .128     |
| 34                                                                                                                       | 6  | 60     | 15.25  | 6863  | -.012   | .209     |
| 24                                                                                                                       | 6  | 70     | 15.01  | 6754  | -.014   | .314     |
| 14                                                                                                                       | 6  | 80     | 14.77  | 6646  | -.017   | .435     |
| 4                                                                                                                        | 6  | 90     | 14.53  | 6537  | -.019   | .561     |
| 92                                                                                                                       | 8  | 0      | 17.04  | 7668  | -.003   | .010     |
| 82                                                                                                                       | 8  | 10     | 16.80  | 7559  | -.005   | .027     |
| 72                                                                                                                       | 8  | 20     | 16.56  | 7450  | -.008   | .057     |
| 62                                                                                                                       | 8  | 30     | 16.31  | 7342  | -.010   | .102     |
| 52                                                                                                                       | 8  | 40     | 16.07  | 7233  | -.012   | .164     |
| 42                                                                                                                       | 8  | 50     | 15.83  | 7124  | -.014   | .244     |
| 32                                                                                                                       | 8  | 60     | 15.59  | 7015  | -.017   | .341     |
| 22                                                                                                                       | 8  | 70     | 15.35  | 6907  | -.019   | .449     |
| 12                                                                                                                       | 8  | 80     | 15.11  | 6798  | -.021   | .561     |
| 2                                                                                                                        | 8  | 90     | 14.86  | 6689  | -.024   | .668     |
| 90                                                                                                                       | 10 | 0      | 17.38  | 7820  | -.008   | .049     |
| 80                                                                                                                       | 10 | 10     | 17.14  | 7711  | -.010   | .084     |
| 70                                                                                                                       | 10 | 20     | 16.89  | 7603  | -.012   | .133     |
| 60                                                                                                                       | 10 | 30     | 16.65  | 7494  | -.014   | .196     |
| 50                                                                                                                       | 10 | 40     | 16.41  | 7385  | -.016   | .273     |

TABLE XIV-continued

| Magnetization and Temperature Coefficient of $(NdHoTb)_2 Fe_{14}B$ Alloys |    |    |             |        |         |          |
|---------------------------------------------------------------------------|----|----|-------------|--------|---------|----------|
| W % $Ho_2Fe_{14}B + X % Nd_2Fe_{14}B + Y % Tb_2Fe_{14}B$                  |    |    | COMPOSITION |        |         |          |
| W                                                                         | X  | Y  | M(25C)      | M(25C) | ALPHA   |          |
|                                                                           |    |    | MB/FU       | GAUSS  | -50-200 | R SQUARE |
| 40                                                                        | 10 | 50 | 16.17       | 7276   | -.018   | .363     |
| 30                                                                        | 10 | 60 | 15.93       | 7168   | -.021   | .460     |
| 20                                                                        | 10 | 70 | 15.69       | 7059   | -.023   | .560     |
| 10                                                                        | 10 | 80 | 15.44       | 6950   | -.026   | .657     |
| 0                                                                         | 10 | 90 | 15.20       | 6841   | -.028   | .744     |
| 88                                                                        | 12 | 0  | 17.72       | 7972   | -.012   | .111     |
| 78                                                                        | 12 | 10 | 17.47       | 8056   | -.014   | .162     |
| 68                                                                        | 12 | 20 | 17.23       | 7755   | -.016   | .224     |
| 58                                                                        | 12 | 30 | 16.99       | 7646   | -.018   | .297     |
| 48                                                                        | 12 | 40 | 16.75       | 7537   | -.020   | .380     |
| 38                                                                        | 12 | 50 | 16.51       | 7429   | -.022   | .468     |
| 28                                                                        | 12 | 60 | 16.27       | 7320   | -.025   | .559     |
| 18                                                                        | 12 | 70 | 16.02       | 7211   | -.027   | .647     |
| 8                                                                         | 12 | 80 | 15.78       | 7102   | -.030   | .728     |
| 86                                                                        | 14 | 0  | 18.05       | 8125   | -.016   | .187     |
| 76                                                                        | 14 | 10 | 17.81       | 8016   | -.018   | .248     |
| 66                                                                        | 14 | 20 | 17.57       | 7907   | -.020   | .317     |
| 56                                                                        | 14 | 30 | 17.33       | 7798   | -.022   | .394     |
| 46                                                                        | 14 | 40 | 17.09       | 7690   | -.024   | .475     |
| 36                                                                        | 14 | 50 | 16.85       | 7581   | -.026   | .558     |
| 26                                                                        | 14 | 60 | 16.60       | 7472   | -.029   | .638     |
| 16                                                                        | 14 | 70 | 16.36       | 7363   | -.031   | .713     |
| 6                                                                         | 14 | 80 | 16.12       | 7255   | -.033   | .780     |
| 84                                                                        | 16 | 0  | 18.39       | 8277   | -.019   | .269     |
| 74                                                                        | 16 | 10 | 18.15       | 8168   | -.021   | .334     |
| 64                                                                        | 16 | 20 | 17.91       | 8059   | -.023   | .406     |
| 54                                                                        | 16 | 30 | 17.67       | 7951   | -.026   | .480     |
| 44                                                                        | 16 | 40 | 17.43       | 7842   | -.028   | .556     |
| 34                                                                        | 16 | 50 | 17.18       | 7733   | -.030   | .630     |
| 24                                                                        | 16 | 60 | 16.94       | 7624   | -.032   | .700     |
| 14                                                                        | 16 | 70 | 16.70       | 7516   | -.035   | .764     |
| 4                                                                         | 16 | 80 | 16.46       | 7407   | -.037   | .820     |
| 82                                                                        | 18 | 0  | 18.73       | 8429   | -.023   | .349     |
| 72                                                                        | 18 | 10 | 18.49       | 8320   | -.025   | .416     |
| 62                                                                        | 18 | 20 | 18.25       | 8212   | -.027   | .485     |
| 52                                                                        | 18 | 30 | 18.01       | 8103   | -.029   | .555     |
| 42                                                                        | 18 | 40 | 17.76       | 7994   | -.031   | .623     |
| 32                                                                        | 18 | 50 | 17.52       | 7885   | -.033   | .689     |
| 22                                                                        | 18 | 60 | 17.28       | 7777   | -.036   | .749     |
| 12                                                                        | 18 | 70 | 17.04       | 7668   | -.038   | .803     |
| 2                                                                         | 18 | 80 | 16.80       | 7559   | -.040   | .850     |
| 80                                                                        | 20 | 0  | 19.07       | 8581   | -.026   | .424     |
| 70                                                                        | 20 | 10 | 18.83       | 8473   | -.028   | .488     |
| 60                                                                        | 20 | 20 | 18.59       | 8364   | -.030   | .553     |
| 50                                                                        | 20 | 30 | 18.34       | 8255   | -.032   | .617     |
| 40                                                                        | 20 | 40 | 18.10       | 8146   | -.035   | .679     |
| 30                                                                        | 20 | 50 | 17.86       | 8037   | -.037   | .736     |
| 20                                                                        | 20 | 60 | 17.62       | 7929   | -.039   | .787     |
| 10                                                                        | 20 | 70 | 17.38       | 7820   | -.041   | .833     |
| 0                                                                         | 20 | 80 | 17.14       | 7711   | -.044   | .873     |

Table XIV shows that with Nd within the range of 7 to 11% the properties are obtained if Ho is maintained within the range of 78 to 90% and Tb varies 9 to 12%.

TABLE XV

| Magnetization and Temperature Coefficient of $(NdHoDy)_2 Fe_{14}B$ Alloys |   |    |             |        |         |          |
|---------------------------------------------------------------------------|---|----|-------------|--------|---------|----------|
| W % $Ho_2Fe_{14}B + X % Nd_2Fe_{14}B + Y % Dy_2Fe_{14}B$                  |   |    | COMPOSITION |        |         |          |
| W                                                                         | X | Y  | M(25C)      | M(25C) | ALPHA   |          |
|                                                                           |   |    | MB/FU       | GAUSS  | -50-200 | R SQUARE |
| 96                                                                        | 4 | 0  | 16.36       | 7364   | .006    | .024     |
| 86                                                                        | 4 | 10 | 16.12       | 7255   | .005    | .024     |
| 76                                                                        | 4 | 20 | 15.88       | 7146   | .005    | .024     |
| 66                                                                        | 4 | 30 | 15.64       | 7037   | -.005   | .023     |
| 56                                                                        | 4 | 40 | 15.40       | 6929   | -.005   | .023     |
| 46                                                                        | 4 | 50 | 15.16       | 6820   | -.005   | .023     |
| 36                                                                        | 4 | 60 | 14.91       | 6711   | -.005   | .022     |
| 26                                                                        | 4 | 70 | 14.67       | 6602   | -.004   | .022     |
| 16                                                                        | 4 | 80 | 14.43       | 6493   | -.004   | .021     |
| 6                                                                         | 4 | 90 | 14.19       | 6385   | -.004   | .021     |
| 94                                                                        | 6 | 0  | 16.70       | 7516   | .001    | .001     |

TABLE XV-continued

| Magnetization and Temperature Coefficient of $(NdHoDy)_2 Fe_{14}B$ Alloys |    |    |             |        |         |          |
|---------------------------------------------------------------------------|----|----|-------------|--------|---------|----------|
| W % $Ho_2Fe_{14}B + X % Nd_2Fe_{14}B + Y % Dy_2Fe_{14}B$                  |    |    | COMPOSITION |        |         |          |
| W                                                                         | X  | Y  | M(25C)      | M(25C) | ALPHA   |          |
|                                                                           |    |    | MB/FU       | GAUSS  | -50-200 | R SQUARE |
| 84                                                                        | 6  | 10 | 16.46       | 7407   | -.001   | .001     |
| 74                                                                        | 6  | 20 | 16.22       | 7298   | -.001   | .000     |
| 64                                                                        | 6  | 30 | 15.98       | 7190   | -.000   | .000     |
| 54                                                                        | 6  | 40 | 15.73       | 7081   | -.000   | .000     |
| 44                                                                        | 6  | 50 | 15.49       | 6972   | -.000   | .000     |
| 34                                                                        | 6  | 60 | 15.25       | 6863   | -.000   | .000     |
| 24                                                                        | 6  | 70 | 15.01       | 6754   | -.001   | .001     |
| 14                                                                        | 6  | 80 | 14.77       | 6646   | -.001   | .001     |
| 4                                                                         | 6  | 90 | 14.53       | 6537   | -.001   | .003     |
| 92                                                                        | 8  | 0  | 17.04       | 7668   | -.003   | .010     |
| 82                                                                        | 8  | 10 | 16.80       | 7559   | -.004   | .012     |
| 72                                                                        | 8  | 20 | 16.56       | 7450   | -.004   | .018     |
| 62                                                                        | 8  | 30 | 16.31       | 7342   | -.004   | .022     |
| 52                                                                        | 8  | 40 | 16.07       | 7233   | -.005   | .027     |
| 42                                                                        | 8  | 50 | 15.83       | 7124   | -.005   | .033     |
| 32                                                                        | 8  | 60 | 15.59       | 7015   | -.005   | .039     |
| 22                                                                        | 8  | 70 | 15.35       | 6907   | -.006   | .048     |
| 60                                                                        | 10 | 30 | 16.65       | 7494   | -.009   | .083     |
| 50                                                                        | 10 | 40 | 16.41       | 7385   | -.009   | .095     |
| 40                                                                        | 10 | 50 | 16.17       | 7276   | -.009   | .109     |
| 30                                                                        | 10 | 60 | 15.93       | 7168   | -.010   | .125     |
| 20                                                                        | 10 | 70 | 15.69       | 7059   | -.010   | .143     |
| 10                                                                        | 10 | 80 | 15.44       | 6950   | -.011   | .164     |
| 10                                                                        | 10 | 90 | 15.20       | 6841   | -.011   | .111     |
| 88                                                                        | 12 | 0  | 17.72       | 7972   | -.012   | .123     |
| 78                                                                        | 12 | 10 | 17.47       | 8056   | -.012   | .137     |
| 68                                                                        | 12 | 20 | 17.23       | 7755   | -.012   | .152     |
| 58                                                                        | 12 | 30 | 16.99       | 7646   | -.013   | .169     |
| 48                                                                        | 12 | 40 | 16.75       | 7537   | -.013   | .188     |
| 38                                                                        | 12 | 50 | 16.51       | 7429   | -.014   | .210     |
| 28                                                                        | 12 | 60 | 16.27       | 7320   | -.014   | .233     |
| 18                                                                        | 12 | 70 | 16.02       | 7211   | -.014   | .260     |
| 8                                                                         | 12 | 80 | 15.78       | 7102   | -.015   | .280     |
| 86                                                                        | 14 | 0  | 18.05       | 8125   | -.017   | .286     |
| 76                                                                        | 14 | 10 | 17.81       | 8016   | -.017   | .344     |
| 66                                                                        | 14 | 20 | 17.57       | 7907   | -.019   | .375     |
| 56                                                                        | 14 | 30 | 17.33       | 7798   | -.019   | .390     |
| 46                                                                        | 14 | 40 | 17.09       | 7690   | -.017   | .475     |
| 36                                                                        | 14 | 50 | 16.85       | 7581   | -.018   | .290     |
| 26                                                                        | 14 | 60 | 16.60       | 7472   | -.018   | .316     |
| 16                                                                        | 14 | 70 | 16.36       | 7363   | -.019   | .344     |
| 6                                                                         | 14 | 80 | 16.12       | 7255   | -.019   | .375     |
| 84                                                                        | 16 | 0  | 18.39       | 8277   | -.019   | .204     |
| 74                                                                        | 16 | 10 | 18.15       | 8168   | -.016   | .223     |
| 64                                                                        | 16 | 20 | 17.91       | 8059   | -.020   | .312     |
| 54                                                                        | 16 | 30 | 17.67       | 7951   | -.021   | .335     |
| 44                                                                        | 16 | 40 | 17.43       | 7842   | -.021   | .360     |
| 34                                                                        | 16 | 50 | 17.18       | 7733   | -.022   | .387     |
| 24                                                                        | 16 | 60 | 16.94       | 7624   | -.022   | .416     |
| 14                                                                        | 16 | 70 | 16.70       | 7516   | -.023   | .446     |
| 4                                                                         | 16 | 80 | 16.46       | 7407   | -.023   | .478     |
| 82                                                                        | 18 | 0  | 18.73       | 8429   | -.023   | .349     |
| 72                                                                        | 18 | 10 | 18.49       | 8320   | -.023   | .372     |
| 62                                                                        | 18 | 20 | 18.25       | 8212   | -.024   | .396     |
| 52                                                                        | 18 | 30 | 18.01       | 8103   | -.024   | .421     |
| 42                                                                        | 18 | 40 | 17.76       | 7994   | -.025   | .447     |
| 32                                                                        | 18 | 50 | 17.52       | 7885   | -.025   | .475     |
| 22                                                                        | 18 | 60 | 17.28       | 7777   | -.026   | .504     |
| 12                                                                        | 18 | 70 | 17.04       | 7668   | -.026   | .533     |
| 2                                                                         | 18 | 80 | 16.80       | 7559   | -.027   | .564     |
| 60                                                                        | 20 | 0  | 19.07       | 8581   | -.026   | .424     |
| 70                                                                        | 20 | 10 | 18.83       | 8473   | -.027   | .447     |
| 60                                                                        | 20 | 20 | 18.59       | 8364   | -.027   | .472     |
| 50                                                                        | 20 | 30 | 18.34       | 8255   | -.028   | .497     |
| 40                                                                        | 20 | 40 | 18.10       | 8146   | -.028   | .523     |
| 30                                                                        | 20 | 50 | 17.86       | 8037   | -.029   | .550     |
| 20                                                                        | 20 | 60 | 17.62       | 7929   | -.029   | .578     |
| 10                                                                        | 20 | 70 | 17.38       | 7820   | -.030   | .606     |
| 0                                                                         | 20 | 80 | 17.14       | 7711   | -.031   | .634     |

In Table XV the desired combination of properties are achieved with alloys containing the addition of 7 to 11%, Ho 75 to 90%, and Dy within the range of 0 to 15%.

TABLE XVI

| Magnetization and Temperature Coefficient of (NdHoGd) <sub>2</sub> Fe <sub>14</sub> B Alloys                             |    |        |        |       |          |
|--------------------------------------------------------------------------------------------------------------------------|----|--------|--------|-------|----------|
| W % Ho <sub>2</sub> Fe <sub>14</sub> B + X % Nd <sub>2</sub> Fe <sub>14</sub> B + Y % Gd <sub>2</sub> Fe <sub>14</sub> B |    |        |        |       |          |
| COMPOSITION                                                                                                              |    | M(25C) | M(25C) | ALPHA |          |
| W                                                                                                                        | X  | Y      | MB/FU  | GAUSS | -50-200  |
|                                                                                                                          |    |        |        |       | R SQUARE |
| 96                                                                                                                       | 4  | 0      | 16.36  | 7364  | .006     |
| 86                                                                                                                       | 4  | 10     | 16.45  | 7403  | -.002    |
| 76                                                                                                                       | 4  | 20     | 16.54  | 7443  | -.009    |
| 66                                                                                                                       | 4  | 30     | 16.63  | 7482  | -.015    |
| 56                                                                                                                       | 4  | 40     | 16.71  | 7521  | -.022    |
| 46                                                                                                                       | 4  | 50     | 16.80  | 7561  | -.029    |
| 36                                                                                                                       | 4  | 60     | 16.89  | 7600  | -.035    |
| 26                                                                                                                       | 4  | 70     | 16.98  | 7640  | -.041    |
| 16                                                                                                                       | 4  | 80     | 17.07  | 7679  | -.047    |
| 6                                                                                                                        | 4  | 90     | 17.15  | 7719  | -.053    |
| 94                                                                                                                       | 6  | 0      | 16.70  | 7516  | .001     |
| 84                                                                                                                       | 6  | 10     | 16.79  | 7555  | -.006    |
| 74                                                                                                                       | 6  | 20     | 16.88  | 7595  | -.013    |
| 64                                                                                                                       | 6  | 30     | 16.96  | 7634  | -.019    |
| 54                                                                                                                       | 6  | 40     | 17.05  | 7674  | -.026    |
| 44                                                                                                                       | 6  | 50     | 17.14  | 7713  | -.032    |
| 34                                                                                                                       | 6  | 60     | 17.23  | 7753  | -.038    |
| 24                                                                                                                       | 6  | 70     | 17.32  | 7792  | -.045    |
| 14                                                                                                                       | 6  | 80     | 17.40  | 7832  | -.050    |
| 4                                                                                                                        | 6  | 90     | 17.49  | 7871  | -.056    |
| 92                                                                                                                       | 8  | 0      | 17.04  | 7668  | -.003    |
| 82                                                                                                                       | 8  | 10     | 17.13  | 7707  | -.010    |
| 72                                                                                                                       | 8  | 20     | 17.22  | 7747  | -.010    |
| 62                                                                                                                       | 8  | 30     | 17.30  | 7786  | -.017    |
| 52                                                                                                                       | 8  | 40     | 17.39  | 7826  | -.023    |
| 42                                                                                                                       | 8  | 50     | 17.48  | 7865  | -.030    |
| 32                                                                                                                       | 8  | 60     | 17.57  | 7905  | -.036    |
| 22                                                                                                                       | 8  | 70     | 17.65  | 7944  | -.042    |
| 12                                                                                                                       | 8  | 80     | 17.74  | 7984  | -.048    |
| 2                                                                                                                        | 8  | 90     | 17.83  | 8023  | -.053    |
| 90                                                                                                                       | 10 | 0      | 17.38  | 7820  | -.059    |
| 80                                                                                                                       | 10 | 10     | 17.47  | 7860  | -.062    |
| 70                                                                                                                       | 10 | 20     | 17.55  | 7899  | -.066    |
| 60                                                                                                                       | 10 | 30     | 17.64  | 7939  | -.070    |
| 50                                                                                                                       | 10 | 40     | 17.73  | 7978  | -.073    |
| 40                                                                                                                       | 10 | 50     | 17.82  | 8018  | -.076    |
| 30                                                                                                                       | 10 | 60     | 17.90  | 8057  | -.079    |
| 20                                                                                                                       | 10 | 70     | 17.99  | 8096  | -.082    |
| 10                                                                                                                       | 10 | 80     | 18.08  | 8136  | -.085    |
| 0                                                                                                                        | 10 | 90     | 18.17  | 8175  | -.088    |
| 88                                                                                                                       | 12 | 0      | 17.72  | 7972  | -.092    |
| 78                                                                                                                       | 12 | 10     | 17.80  | 8012  | -.095    |
| 68                                                                                                                       | 12 | 20     | 17.89  | 8051  | -.098    |
| 58                                                                                                                       | 12 | 30     | 17.98  | 8091  | -.101    |
| 48                                                                                                                       | 12 | 40     | 18.07  | 8130  | -.104    |
| 38                                                                                                                       | 12 | 50     | 18.16  | 8170  | -.107    |
| 28                                                                                                                       | 12 | 60     | 18.24  | 8209  | -.110    |
| 18                                                                                                                       | 12 | 70     | 18.33  | 8249  | -.113    |
| 8                                                                                                                        | 12 | 80     | 18.42  | 8288  | -.116    |
| 86                                                                                                                       | 14 | 0      | 18.05  | 8125  | -.119    |
| 76                                                                                                                       | 14 | 10     | 18.14  | 8164  | -.122    |
| 66                                                                                                                       | 14 | 20     | 18.23  | 8204  | -.125    |
| 56                                                                                                                       | 14 | 30     | 18.32  | 8243  | -.128    |
| 46                                                                                                                       | 14 | 40     | 18.41  | 8283  | -.131    |
| 36                                                                                                                       | 14 | 50     | 18.49  | 8322  | -.134    |
| 26                                                                                                                       | 14 | 60     | 18.58  | 8361  | -.137    |
| 16                                                                                                                       | 14 | 70     | 18.67  | 8401  | -.140    |
| 6                                                                                                                        | 14 | 80     | 18.76  | 8440  | -.143    |
| 84                                                                                                                       | 16 | 0      | 18.39  | 8277  | -.146    |
| 74                                                                                                                       | 16 | 10     | 18.48  | 8316  | -.149    |
| 64                                                                                                                       | 16 | 20     | 18.57  | 8356  | -.152    |
| 54                                                                                                                       | 16 | 30     | 18.66  | 8395  | -.155    |
| 44                                                                                                                       | 16 | 40     | 18.74  | 8435  | -.158    |
| 34                                                                                                                       | 16 | 50     | 18.83  | 8474  | -.161    |
| 24                                                                                                                       | 16 | 60     | 18.92  | 8514  | -.164    |
| 14                                                                                                                       | 16 | 70     | 19.01  | 8553  | -.167    |
| 4                                                                                                                        | 16 | 80     | 19.09  | 8593  | -.170    |
| 82                                                                                                                       | 18 | 0      | 18.73  | 8429  | -.173    |
| 72                                                                                                                       | 18 | 10     | 18.82  | 8469  | -.176    |
| 62                                                                                                                       | 18 | 20     | 18.91  | 8508  | -.179    |
| 52                                                                                                                       | 18 | 30     | 18.99  | 8547  | -.182    |

TABLE XVI-continued

| Magnetization and Temperature Coefficient of (NdHoGd) <sub>2</sub> Fe <sub>14</sub> B Alloys                             |    |        |        |       |          |
|--------------------------------------------------------------------------------------------------------------------------|----|--------|--------|-------|----------|
| W % Ho <sub>2</sub> Fe <sub>14</sub> B + X % Nd <sub>2</sub> Fe <sub>14</sub> B + Y % Gd <sub>2</sub> Fe <sub>14</sub> B |    |        |        |       |          |
| COMPOSITION                                                                                                              |    | M(25C) | M(25C) | ALPHA |          |
| W                                                                                                                        | X  | Y      | MB/FU  | GAUSS | -50-200  |
|                                                                                                                          |    |        |        |       | R SQUARE |
| 42                                                                                                                       | 18 | 40     | 19.08  | 8587  | -.045    |
| 32                                                                                                                       | 18 | 50     | 19.17  | 8626  | -.051    |
| 22                                                                                                                       | 18 | 60     | 19.26  | 8666  | -.056    |
| 12                                                                                                                       | 18 | 70     | 19.35  | 8705  | -.061    |
| 2                                                                                                                        | 18 | 80     | 19.43  | 8745  | -.066    |
| 80                                                                                                                       | 20 | 0      | 19.07  | 8581  | -.026    |
| 70                                                                                                                       | 20 | 10     | 19.16  | 8621  | -.032    |
| 60                                                                                                                       | 20 | 20     | 19.25  | 8660  | -.037    |
| 50                                                                                                                       | 20 | 30     | 19.33  | 8700  | -.043    |
| 40                                                                                                                       | 20 | 40     | 19.42  | 8739  | -.048    |
| 30                                                                                                                       | 20 | 50     | 19.51  | 8779  | -.054    |
| 20                                                                                                                       | 20 | 60     | 19.60  | 8818  | -.059    |
| 10                                                                                                                       | 20 | 70     | 19.68  | 8858  | -.064    |
| 0                                                                                                                        | 20 | 80     | 19.77  | 8897  | -.069    |

  

| Magnetization and Temperature Coefficient of (NdTbGdHo) <sub>2</sub> Fe <sub>14</sub> B Alloys                                                                  |   |        |        |       |          |
|-----------------------------------------------------------------------------------------------------------------------------------------------------------------|---|--------|--------|-------|----------|
| W % Tb <sub>2</sub> Fe <sub>14</sub> B + X % Nd <sub>2</sub> Fe <sub>14</sub> B + Y % Ho <sub>2</sub> Fe <sub>14</sub> B Z % Gd <sub>2</sub> Fe <sub>14</sub> B |   |        |        |       |          |
| COMPOSITION                                                                                                                                                     |   | M(25C) | M(25C) | ALPHA |          |
| W                                                                                                                                                               | X | Y      | Z      | MB/FU | GAUSS    |
|                                                                                                                                                                 |   |        |        |       | R SQUARE |
| 38                                                                                                                                                              | 2 | 0      | 60     | 15.11 | 6798     |
| 28                                                                                                                                                              | 2 | 0      | 70     | 15.35 | 6907     |
| 18                                                                                                                                                              | 2 | 0      | 80     | 15.59 | 7016     |
| 8                                                                                                                                                               | 2 | 0      | 90     | 15.83 | 7124     |
| 34                                                                                                                                                              | 2 | 4      | 60     | 15.24 | 6857     |
| 24                                                                                                                                                              | 2 | 4      | 70     | 15.48 | 6966     |
| 14                                                                                                                                                              | 2 | 4      | 80     | 15.72 | 7075     |
| 4                                                                                                                                                               | 2 | 4      | 90     | 15.96 | 7184     |
| 30                                                                                                                                                              | 2 | 8      | 60     | 15.37 | 6917     |
| 20                                                                                                                                                              | 2 | 8      | 70     | 15.61 | 7025     |
| 10                                                                                                                                                              | 2 | 8      | 80     | 15.85 | 7134     |
| 0                                                                                                                                                               | 2 | 8      | 90     | 16.10 | 7243     |
| 26                                                                                                                                                              | 2 | 12     | 60     | 15.50 | 6976     |
| 16                                                                                                                                                              | 2 | 12     | 70     | 15.74 | 7085     |
| 6                                                                                                                                                               | 2 | 12     | 80     | 15.99 | 7193     |
| 22                                                                                                                                                              | 2 | 16     | 60     | 15.63 | 7035     |
| 12                                                                                                                                                              | 2 | 16     | 70     | 15.88 | 7144     |
| 2                                                                                                                                                               | 2 | 16     | 80     | 16.12 | 7253     |
| 18                                                                                                                                                              | 2 | 20     | 60     | 15.77 | 7095     |
| 8                                                                                                                                                               | 2 | 20     | 70     | 16.01 | 7203     |
| 36                                                                                                                                                              | 4 | 0      | 60     | 15.49 | 6972     |
| 26                                                                                                                                                              | 4 | 0      | 70     | 15.74 | 7081     |
| 16                                                                                                                                                              | 4 | 0      | 80     | 15.98 | 7190     |
| 6                                                                                                                                                               | 4 | 0      | 90     | 16.22 | 7298     |
| 32                                                                                                                                                              | 4 | 4      | 60     | 15.63 | 7031     |
| 22                                                                                                                                                              | 4 | 4      | 70     | 15.87 | 7140     |
| 12                                                                                                                                                              | 4 | 4      | 80     | 16.11 | 7249     |
| 2                                                                                                                                                               | 4 | 4      | 90     | 16.35 | 7358     |
| 28                                                                                                                                                              | 4 | 8      | 60     | 15.76 | 7091     |
| 18                                                                                                                                                              | 4 | 8      | 70     | 16.00 | 7199     |
| 8                                                                                                                                                               | 4 | 8      | 80     | 16.24 | 7308     |
| 14                                                                                                                                                              | 4 | 12     | 60     | 15.89 | 7150     |
| 14                                                                                                                                                              | 4 | 12     | 70     | 16.13 | 7259     |
| 4                                                                                                                                                               | 4 | 12     | 80     | 16.37 | 7367     |
| 20                                                                                                                                                              | 4 | 16     | 60     | 16.02 | 7209     |
| 16                                                                                                                                                              | 4 | 20     | 60     | 16.15 | 7268     |
| 6                                                                                                                                                               | 4 | 20     | 70     | 16.39 | 7377     |
| 34                                                                                                                                                              | 6 | 0      | 60     | 15.88 | 7146     |
| 24                                                                                                                                                              | 6 | 0      | 70     | 16.12 | 7255     |
| 14                                                                                                                                                              | 6 | 0      | 80     | 16.36 | 7364     |
| 4                                                                                                                                                               | 6 | 0      | 90     | 16.61 | 7472     |
| 30                                                                                                                                                              | 6 | 4      | 60     | 16.01 | 7205     |

Table XVI shows that the desired combination of properties may be achieved with 7 to 11% Nd, 82 to 90% Ho, and 0 to 10% Gd.

It was further determined experimentally that the desired range of rare earth elements may be increased while achieving the desired combination of properties if three heavy rare earth elements are used in combination with Nd.

TABLE XVII

| Magnetization and Temperature Coefficient of (NdTbGdHo) <sub>2</sub> Fe <sub>14</sub> B Alloys                                                                  |   |        |        |       |          |
|-----------------------------------------------------------------------------------------------------------------------------------------------------------------|---|--------|--------|-------|----------|
| W % Tb <sub>2</sub> Fe <sub>14</sub> B + X % Nd <sub>2</sub> Fe <sub>14</sub> B + Y % Ho <sub>2</sub> Fe <sub>14</sub> B Z % Gd <sub>2</sub> Fe <sub>14</sub> B |   |        |        |       |          |
| COMPOSITION                                                                                                                                                     |   | M(25C) | M(25C) | ALPHA |          |
| W                                                                                                                                                               | X | Y      | Z      | MB/FU | GAUSS    |
|                                                                                                                                                                 |   |        |        |       | R SQUARE |
| 38                                                                                                                                                              | 2 | 0      | 60     | 15.11 | 6798     |
| 28                                                                                                                                                              | 2 | 0      | 70     | 15.35 | 6907     |
| 18                                                                                                                                                              | 2 | 0      | 80     | 15.59 | 7016     |
| 8                                                                                                                                                               | 2 | 0      | 90     | 15.83 | 7124     |
| 34                                                                                                                                                              | 2 | 4      | 60     | 15.24 | 6857     |
| 24                                                                                                                                                              | 2 | 4      | 70     | 15.48 | 6966     |
| 14                                                                                                                                                              | 2 | 4      | 80     | 15.72 | 7075     |
| 4                                                                                                                                                               | 2 | 4      | 90     | 15.96 | 7184     |
| 30                                                                                                                                                              | 2 | 8      | 60     | 15.37 | 6917     |
| 20                                                                                                                                                              | 2 | 8      | 70     | 15.61 | 7025     |
| 10                                                                                                                                                              | 2 | 8      | 80     | 15.85 | 7134     |
| 0                                                                                                                                                               | 2 | 8      | 90     | 16.10 | 7243     |
| 26                                                                                                                                                              | 2 | 12     | 60     | 15.50 | 6976     |
| 16                                                                                                                                                              | 2 | 12     | 70     | 15.74 | 7081     |
| 6                                                                                                                                                               | 2 | 12     | 80     | 15.98 | 7190     |
| 32                                                                                                                                                              | 2 | 16     | 60     | 16.22 | 7298     |
| 22                                                                                                                                                              | 2 | 16     | 70     | 16.37 | 7367     |
| 12                                                                                                                                                              | 2 | 16     | 80     | 16.63 | 7309     |
| 2                                                                                                                                                               | 2 | 16     | 90     | 16.87 | 7377     |
| 36                                                                                                                                                              | 4 | 0      | 60     | 15.49 | 6972     |
| 26                                                                                                                                                              | 4 | 0      | 70     | 15.74 | 7081     |
| 16                                                                                                                                                              | 4 | 0      | 80     | 15.98 | 7190     |
| 6                                                                                                                                                               | 4 | 0      | 90     | 16.22 | 7298     |
| 32                                                                                                                                                              | 4 | 4      | 60     | 15.63 | 7031     |
| 22                                                                                                                                                              | 4 | 4      | 70     | 15.87 | 7140     |
| 12                                                                                                                                                              | 4 | 4      | 80     | 16.11 | 7249     |
| 2                                                                                                                                                               | 4 | 4      | 90     | 16.35 | 7358     |
| 30                                                                                                                                                              | 4 | 8      | 60     | 15.76 | 7091     |
| 20                                                                                                                                                              |   |        |        |       |          |

TABLE XVII-continued

| Magnetization and Temperature Coefficient of (NdTbGdHo) <sub>2</sub> Fe <sub>14</sub> B Alloys |    |        |        |       |                                                                                                                                                   |         |          |
|------------------------------------------------------------------------------------------------|----|--------|--------|-------|---------------------------------------------------------------------------------------------------------------------------------------------------|---------|----------|
| COMPOSITION                                                                                    |    | M(25C) | M(25C) | ALPHA | W % Tb <sub>2</sub> Fe <sub>14</sub> B + X % Nd <sub>2</sub> Fe <sub>14</sub> B + Y % Ho <sub>2</sub> Fe <sub>14</sub> B Z % HoFe <sub>14</sub> B |         |          |
| W                                                                                              | X  | Y      | Z      | MB/FU | GAUSS                                                                                                                                             | -50-200 | R SQUARE |
| 20                                                                                             | 6  | 4      | 70     | 16.25 | 7314                                                                                                                                              | -.006   | .036     |
| 10                                                                                             | 6  | 4      | 80     | 16.50 | 7423                                                                                                                                              | -.004   | .014     |
| 0                                                                                              | 6  | 4      | 90     | 16.74 | 7532                                                                                                                                              | -.002   | .003     |
| 26                                                                                             | 6  | 8      | 60     | 16.14 | 7265                                                                                                                                              | -.010   | .109     |
| 16                                                                                             | 6  | 8      | 70     | 16.39 | 7373                                                                                                                                              | -.008   | .062     |
| 6                                                                                              | 6  | 8      | 80     | 16.63 | 7482                                                                                                                                              | -.006   | .031     |
| 22                                                                                             | 6  | 12     | 60     | 16.28 | 7324                                                                                                                                              | -.012   | .146     |
| 12                                                                                             | 6  | 12     | 70     | 16.52 | 7433                                                                                                                                              | -.010   | .092     |
| 2                                                                                              | 6  | 12     | 80     | 16.76 | 7541                                                                                                                                              | -.008   | .052     |
| 18                                                                                             | 6  | 16     | 60     | 16.41 | 7383                                                                                                                                              | -.014   | .185     |
| 8                                                                                              | 6  | 16     | 70     | 16.65 | 7492                                                                                                                                              | -.012   | .125     |
| 14                                                                                             | 6  | 20     | 60     | 16.54 | 7442                                                                                                                                              | -.016   | .223     |
| 4                                                                                              | 6  | 20     | 70     | 16.78 | 7551                                                                                                                                              | -.014   | .159     |
| 32                                                                                             | 8  | 0      | 60     | 16.27 | 7320                                                                                                                                              | -.010   | .113     |
| 22                                                                                             | 8  | 0      | 70     | 16.51 | 7429                                                                                                                                              | -.008   | .065     |
| 12                                                                                             | 8  | 0      | 80     | 16.75 | 7538                                                                                                                                              | -.006   | .032     |
| 2                                                                                              | 8  | 0      | 90     | 16.99 | 7646                                                                                                                                              | -.004   | .012     |
| 28                                                                                             | 8  | 4      | 60     | 16.40 | 7379                                                                                                                                              | -.012   | .151     |
| 18                                                                                             | 8  | 4      | 70     | 16.64 | 7488                                                                                                                                              | -.010   | .095     |
| 8                                                                                              | 8  | 4      | 80     | 16.88 | 7597                                                                                                                                              | -.008   | .055     |
| 24                                                                                             | 8  | 8      | 60     | 16.53 | 7439                                                                                                                                              | -.014   | .190     |
| 14                                                                                             | 8  | 8      | 70     | 16.77 | 7547                                                                                                                                              | -.012   | .129     |
| 4                                                                                              | 8  | 8      | 80     | 17.01 | 7656                                                                                                                                              | -.010   | .081     |
| 20                                                                                             | 8  | 12     | 60     | 16.66 | 7498                                                                                                                                              | -.016   | .230     |
| 10                                                                                             | 8  | 12     | 70     | 16.90 | 7607                                                                                                                                              | -.014   | .164     |
| 0                                                                                              | 8  | 12     | 80     | 17.15 | 7715                                                                                                                                              | -.011   | .111     |
| 16                                                                                             | 8  | 16     | 60     | 16.79 | 7557                                                                                                                                              | -.018   | .268     |
| 6                                                                                              | 8  | 16     | 70     | 17.04 | 7666                                                                                                                                              | -.015   | .200     |
| 12                                                                                             | 8  | 20     | 60     | 16.93 | 7616                                                                                                                                              | -.019   | .306     |
| 2                                                                                              | 8  | 20     | 70     | 17.17 | 7725                                                                                                                                              | -.017   | .235     |
| 30                                                                                             | 10 | 0      | 60     | 16.65 | 7494                                                                                                                                              | -.014   | .196     |
| 20                                                                                             | 10 | 0      | 70     | 16.89 | 7603                                                                                                                                              | -.012   | .133     |
| 10                                                                                             | 10 | 0      | 80     | 17.14 | 7711                                                                                                                                              | -.010   | .084     |
| 26                                                                                             | 10 | 4      | 60     | 16.78 | 7553                                                                                                                                              | -.016   | .236     |
| 16                                                                                             | 10 | 4      | 70     | 17.03 | 7662                                                                                                                                              | -.014   | .169     |
| 6                                                                                              | 10 | 4      | 80     | 17.27 | 7771                                                                                                                                              | -.012   | .114     |
| 22                                                                                             | 10 | 8      | 60     | 16.92 | 7613                                                                                                                                              | -.018   | .275     |
| 12                                                                                             | 10 | 8      | 70     | 17.16 | 7721                                                                                                                                              | -.015   | .205     |
| 2                                                                                              | 10 | 8      | 80     | 17.40 | 7830                                                                                                                                              | -.013   | .146     |
| 18                                                                                             | 10 | 12     | 60     | 17.05 | 7672                                                                                                                                              | -.019   | .313     |
| 8                                                                                              | 10 | 12     | 70     | 17.29 | 7781                                                                                                                                              | -.017   | .241     |
| 14                                                                                             | 10 | 16     | 60     | 17.18 | 7731                                                                                                                                              | -.021   | .348     |
| 4                                                                                              | 10 | 16     | 70     | 17.42 | 7840                                                                                                                                              | -.019   | .276     |
| 10                                                                                             | 10 | 20     | 60     | 17.31 | 7790                                                                                                                                              | -.023   | .382     |
| 0                                                                                              | 10 | 20     | 70     | 17.55 | 7899                                                                                                                                              | -.021   | .310     |
| 28                                                                                             | 12 | 0      | 60     | 17.04 | 7668                                                                                                                                              | -.018   | .282     |
| 18                                                                                             | 12 | 0      | 70     | 17.28 | 7777                                                                                                                                              | -.015   | .211     |
| 8                                                                                              | 12 | 0      | 80     | 17.52 | 7885                                                                                                                                              | -.013   | .151     |
| 24                                                                                             | 12 | 4      | 60     | 17.17 | 7727                                                                                                                                              | -.019   | .320     |
| 14                                                                                             | 12 | 4      | 70     | 17.41 | 7836                                                                                                                                              | -.017   | .247     |
| 4                                                                                              | 12 | 4      | 80     | 17.65 | 7945                                                                                                                                              | -.015   | .184     |
| 20                                                                                             | 12 | 8      | 60     | 17.30 | 7786                                                                                                                                              | -.021   | .355     |
| 10                                                                                             | 12 | 8      | 70     | 17.55 | 7895                                                                                                                                              | -.019   | .282     |
| 0                                                                                              | 12 | 8      | 80     | 17.79 | 8004                                                                                                                                              | -.017   | .217     |
| 16                                                                                             | 12 | 12     | 60     | 17.44 | 7846                                                                                                                                              | -.023   | .389     |
| 6                                                                                              | 12 | 12     | 70     | 17.68 | 7955                                                                                                                                              | -.021   | .317     |
| 12                                                                                             | 12 | 16     | 60     | 17.57 | 7905                                                                                                                                              | -.024   | .421     |
| 2                                                                                              | 12 | 16     | 70     | 17.81 | 8014                                                                                                                                              | -.022   | .349     |
| 8                                                                                              | 12 | 20     | 60     | 17.70 | 7964                                                                                                                                              | -.026   | .450     |

TABLE XIX

| Magnetization and Temperature Coefficient of (NdErDyHo) <sub>2</sub> Fe <sub>14</sub> B Alloys |    |        |        |       |                                                                                                                                                   |         |          |
|------------------------------------------------------------------------------------------------|----|--------|--------|-------|---------------------------------------------------------------------------------------------------------------------------------------------------|---------|----------|
| COMPOSITION                                                                                    |    | M(25C) | M(25C) | ALPHA | W % Er <sub>2</sub> Fe <sub>14</sub> B + X % Nd <sub>2</sub> Fe <sub>14</sub> B + Y % Dy <sub>2</sub> Fe <sub>14</sub> B Z % HoFe <sub>14</sub> B |         |          |
| W                                                                                              | X  | Y      | Z      | MB/FU | GAUSS                                                                                                                                             | -50-200 | R SQUARE |
| 38                                                                                             | 2  | 0      | 60     | 16.73 | 7528                                                                                                                                              | -.013   | .065     |
| 28                                                                                             | 2  | 0      | 70     | 16.54 | 7444                                                                                                                                              | -.007   | .023     |
| 10                                                                                             | 18 | 2      | 0      | 80    | 16.36                                                                                                                                             | -.001   | .001     |
|                                                                                                | 8  | 2      | 0      | 90    | 16.17                                                                                                                                             | 7278    | .005     |
|                                                                                                | 34 | 2      | 4      | 60    | 16.56                                                                                                                                             | 7451    | -.011    |
|                                                                                                | 24 | 2      | 4      | 70    | 16.37                                                                                                                                             | 7368    | -.005    |
| 15                                                                                             | 14 | 2      | 4      | 80    | 16.19                                                                                                                                             | 7284    | .001     |
|                                                                                                | 4  | 2      | 4      | 90    | 16.00                                                                                                                                             | 7201    | .008     |
|                                                                                                | 30 | 2      | 8      | 60    | 16.39                                                                                                                                             | 7374    | -.009    |
|                                                                                                | 20 | 2      | 8      | 70    | 16.20                                                                                                                                             | 7291    | -.002    |
|                                                                                                | 10 | 2      | 8      | 80    | 16.02                                                                                                                                             | 7208    | .004     |
|                                                                                                | 0  | 2      | 8      | 90    | 15.83                                                                                                                                             | 7124    | .010     |
|                                                                                                | 26 | 2      | 12     | 60    | 16.22                                                                                                                                             | 7297    | -.006    |
|                                                                                                | 16 | 2      | 12     | 70    | 16.03                                                                                                                                             | 7214    | -.000    |
| 20                                                                                             | 6  | 2      | 12     | 80    | 15.85                                                                                                                                             | 7131    | .006     |
|                                                                                                | 22 | 2      | 16     | 60    | 16.05                                                                                                                                             | 7220    | -.004    |
|                                                                                                | 12 | 2      | 16     | 70    | 15.86                                                                                                                                             | 7137    | .002     |
|                                                                                                | 2  | 2      | 16     | 80    | 15.68                                                                                                                                             | 7054    | .009     |
|                                                                                                | 18 | 2      | 20     | 60    | 15.87                                                                                                                                             | 7144    | -.002    |
|                                                                                                | 8  | 2      | 20     | 70    | 15.69                                                                                                                                             | 7060    | .005     |
| 25                                                                                             | 36 | 4      | 0      | 60    | 17.03                                                                                                                                             | 7663    | -.016    |
|                                                                                                | 26 | 4      | 0      | 70    | 16.84                                                                                                                                             | 7580    | -.010    |
|                                                                                                | 16 | 4      | 0      | 80    | 16.66                                                                                                                                             | 7497    | -.004    |
|                                                                                                | 6  | 4      | 0      | 90    | 16.47                                                                                                                                             | 7414    | .002     |
|                                                                                                | 32 | 4      | 4      | 60    | 16.86                                                                                                                                             | 7586    | -.014    |
|                                                                                                | 22 | 4      | 4      | 70    | 16.67                                                                                                                                             | 7503    | -.008    |
|                                                                                                | 12 | 4      | 4      | 80    | 16.49                                                                                                                                             | 7420    | -.002    |
|                                                                                                | 2  | 4      | 4      | 90    | 16.30                                                                                                                                             | 7337    | .004     |
| 30                                                                                             | 28 | 4      | 8      | 60    | 16.69                                                                                                                                             | 7510    | -.012    |
|                                                                                                | 18 | 4      | 8      | 70    | 16.50                                                                                                                                             | 7426    | -.006    |
|                                                                                                | 8  | 4      | 8      | 80    | 16.32                                                                                                                                             | 7343    | .000     |
|                                                                                                | 24 | 4      | 12     | 60    | 16.52                                                                                                                                             | 7433    | -.009    |
|                                                                                                | 14 | 4      | 12     | 70    | 16.33                                                                                                                                             | 7350    | -.003    |
|                                                                                                | 4  | 4      | 12     | 80    | 16.15                                                                                                                                             | 7266    | .003     |
|                                                                                                | 20 | 4      | 16     | 60    | 16.35                                                                                                                                             | 7356    | -.007    |
|                                                                                                | 10 | 4      | 16     | 70    | 16.16                                                                                                                                             | 7273    | -.001    |
|                                                                                                | 0  | 4      | 16     | 80    | 15.98                                                                                                                                             | 7190    | .005     |
|                                                                                                | 16 | 4      | 20     | 60    | 16.18                                                                                                                                             | 7279    | -.005    |
|                                                                                                | 6  | 4      | 20     | 70    | 15.99                                                                                                                                             | 7196    | .001     |
| 40                                                                                             | 34 | 6      | 0      | 60    | 17.33                                                                                                                                             | 7799    | -.019    |
|                                                                                                | 24 | 6      | 0      | 70    | 17.15                                                                                                                                             | 7715    | -.013    |
|                                                                                                | 14 | 6      | 0      | 80    | 16.96                                                                                                                                             | 7632    | -.007    |
|                                                                                                | 4  | 6      | 0      | 90    | 16.78                                                                                                                                             | 7549    | -.001    |
|                                                                                                | 30 | 6      | 4      | 60    | 17.16                                                                                                                                             | 7722    | -.017    |
|                                                                                                | 20 | 6      | 4      | 70    | 16.97                                                                                                                                             | 7639    | -.011    |
|                                                                                                | 10 | 6      | 4      | 80    | 16.79                                                                                                                                             | 7556    | -.005    |
|                                                                                                | 0  | 6      | 4      | 90    | 16.61                                                                                                                                             | 7472    | .001     |
|                                                                                                | 26 | 6      | 8      | 60    | 16.99                                                                                                                                             | 7645    | -.015    |
|                                                                                                | 16 | 6      | 8      | 70    | 16.80                                                                                                                                             | 7562    | -.009    |
|                                                                                                | 6  | 6      | 8      | 80    | 16.62                                                                                                                                             | 7479    | -.003    |
|                                                                                                | 2  | 6      | 12     | 60    | 16.82                                                                                                                                             | 7568    | -.012    |
| 50                                                                                             | 12 | 6      | 12     | 70    | 16.63                                                                                                                                             | 7485    | -.007    |
|                                                                                                | 2  | 6      | 12     | 80    | 16.45                                                                                                                                             | 7402    | -.001    |
|                                                                                                | 18 | 6      | 16     | 60    | 16.65                                                                                                                                             | 7492    | -.010    |
|                                                                                                | 8  | 6      | 16     | 70    | 16.46                                                                                                                                             | 7408    | -.004    |
|                                                                                                | 14 | 6      | 20     | 60    | 16.48                                                                                                                                             | 7415    | -.008    |
|                                                                                                | 4  | 6      | 20     | 70    | 16.29                                                                                                                                             | 7332    | -.002    |
|                                                                                                | 32 | 8      | 0      | 60    | 17.63                                                                                                                                             | 7934    | -.021    |
|                                                                                                | 22 | 8      | 0      | 70    | 17.45                                                                                                                                             | 7851    | -.016    |
|                                                                                                | 12 | 8      | 0      | 80    | 17.26                                                                                                                                             | 7768    | -.010    |
|                                                                                                | 2  | 8      | 0      | 90    | 17.08                                                                                                                                             | 7685    | -.005    |
|                                                                                                | 28 | 8      | 4      | 60    | 17.46                                                                                                                                             | 7857    | -.019    |
|                                                                                                | 18 | 8      | 4      | 70    | 17.28                                                                                                                                             | 7774    | -.014    |
|                                                                                                | 8  | 8      | 4      | 80    | 17.09                                                                                                                                             | 7691    | -.008    |
|                                                                                                | 24 | 8      | 8      | 60    | 17.29                                                                                                                                             | 7781    | -.017    |
|                                                                                                | 14 | 8      | 8      | 70    | 17.11                                                                                                                                             | 7697    | -.012    |
|                                                                                                | 4  | 8      | 8      | 80    | 16.92                                                                                                                                             | 7614    | -.006    |
|                                                                                                | 20 | 8      | 12     | 60    | 17.12                                                                                                                                             | 7704    | -.015    |
|                                                                                                | 10 | 8      | 12     | 70    | 16.93                                                                                                                                             | 7621    | -.010    |
|                                                                                                | 0  | 8      | 12     | 80    | 16.75                                                                                                                                             | 7538    | -.004    |
|                                                                                                | 16 | 8      | 16     | 60    | 16.95                                                                                                                                             | 7627    | -.013    |
|                                                                                                | 6  | 8      | 16     | 70    | 16.76                                                                                                                                             | 7544    | -.007    |
|                                                                                                | 12 | 8      | 20     | 60    | 16.78                                                                                                                                             | 7550    | -.011    |
|                                                                                                | 2  | 8      | 20     | 70    | 16.59                                                                                                                                             | 7467    | -.005    |
| 55                                                                                             | 30 | 10     | 0      | 60    | 17.93                                                                                                                                             | 8070    | -.024    |

It was further determined experimentally that the desired range of rare earth elements may be increased while achieving the desired combination of properties if 60 three heavy rare earth elements are used in combination with Nd.

In Table XVII Nd is combined with Tb, Gd and Ho. Specifically, the data show that if Nd varies from 1 to 10%, Tb 0 to 10%, and Gd 0 to 4% with Ho within the 65 range of 80 to 90% the desired combination of properties is achieved.

TABLE XIX-continued

| Magnetization and Temperature Coefficient<br>of (NdErDyHo) <sub>2</sub> Fe <sub>14</sub> B Alloys                                                    |    |        |    |        |       |         |        |
|------------------------------------------------------------------------------------------------------------------------------------------------------|----|--------|----|--------|-------|---------|--------|
| W % Er <sub>2</sub> Fe <sub>14</sub> B + X % Nd <sub>2</sub> Fe <sub>14</sub> B + Y % Dy <sub>2</sub> Fe <sub>14</sub> B Z %<br>HoFe <sub>14</sub> B |    |        |    |        |       |         |        |
| COMPOSITION                                                                                                                                          |    | M(25C) |    | M(25C) |       | ALPHA   | R      |
| W                                                                                                                                                    | X  | Y      | Z  | MB/FU  | GAUSS | -50-200 | SQUARE |
| 20                                                                                                                                                   | 10 | 0      | 70 | 17.75  | 7987  | -.019   | .181   |
| 10                                                                                                                                                   | 10 | 0      | 80 | 17.56  | 7903  | -.013   | .115   |
| 0                                                                                                                                                    | 10 | 0      | 90 | 17.38  | 7820  | -.008   | .049   |
| 26                                                                                                                                                   | 10 | 4      | 60 | 17.76  | 7993  | -.022   | .223   |
| 16                                                                                                                                                   | 10 | 4      | 70 | 17.58  | 7910  | -.017   | .160   |
| 6                                                                                                                                                    | 10 | 4      | 80 | 17.39  | 7827  | -.011   | .092   |
| 22                                                                                                                                                   | 10 | 8      | 60 | 17.59  | 7916  | -.020   | .205   |
| 12                                                                                                                                                   | 10 | 8      | 70 | 17.41  | 7833  | -.015   | .138   |
| 2                                                                                                                                                    | 10 | 8      | 80 | 17.22  | 7750  | -.009   | .068   |
| 18                                                                                                                                                   | 10 | 12     | 60 | 17.42  | 7839  | -.018   | .184   |
| 8                                                                                                                                                    | 10 | 12     | 70 | 17.24  | 7756  | -.013   | .114   |
| 14                                                                                                                                                   | 10 | 16     | 60 | 17.25  | 7763  | -.016   | .163   |
| 4                                                                                                                                                    | 10 | 16     | 70 | 17.07  | 7679  | -.010   | .089   |
| 10                                                                                                                                                   | 10 | 20     | 60 | 17.08  | 7686  | -.014   | .139   |
| 0                                                                                                                                                    | 10 | 20     | 70 | 16.89  | 7603  | -.008   | .064   |
| 28                                                                                                                                                   | 12 | 0      | 60 | 18.23  | 8205  | -.026   | .292   |
| 18                                                                                                                                                   | 12 | 0      | 70 | 18.05  | 8122  | -.021   | .236   |
| 8                                                                                                                                                    | 12 | 0      | 80 | 17.86  | 8039  | -.016   | .170   |
| 24                                                                                                                                                   | 12 | 4      | 60 | 18.06  | 8129  | -.025   | .277   |
| 14                                                                                                                                                   | 12 | 4      | 70 | 17.88  | 8045  | -.019   | .217   |
| 4                                                                                                                                                    | 12 | 4      | 80 | 17.69  | 7962  | -.014   | .146   |
| 20                                                                                                                                                   | 12 | 8      | 60 | 17.89  | 8052  | -.023   | .261   |
| 10                                                                                                                                                   | 12 | 8      | 70 | 17.71  | 7969  | -.017   | .196   |
| 0                                                                                                                                                    | 12 | 8      | 80 | 17.52  | 7885  | -.012   | .121   |
| 16                                                                                                                                                   | 12 | 12     | 60 | 17.72  | 7975  | -.021   | .243   |
| 6                                                                                                                                                    | 12 | 12     | 70 | 17.54  | 7892  | -.015   | .173   |
| 12                                                                                                                                                   | 12 | 16     | 60 | 17.55  | 7898  | -.019   | .223   |
| 2                                                                                                                                                    | 12 | 16     | 70 | 17.37  | 7815  | -.013   | .148   |
| 8                                                                                                                                                    | 12 | 20     | 60 | 17.38  | 7821  | -.017   | .201   |

TABLE XXI

| Magnetization and Temperature Coefficient<br>of (NdErTmHo) <sub>2</sub> Fe <sub>14</sub> B Alloys                                                    |   |        |    |        |       |         |        |
|------------------------------------------------------------------------------------------------------------------------------------------------------|---|--------|----|--------|-------|---------|--------|
| W % Er <sub>2</sub> Fe <sub>14</sub> B + X % Nd <sub>2</sub> Fe <sub>14</sub> B + Y % Tm <sub>2</sub> Fe <sub>14</sub> B Z %<br>HoFe <sub>14</sub> B |   |        |    |        |       |         |        |
| COMPOSITION                                                                                                                                          |   | M(25C) |    | M(25C) |       | ALPHA   | R      |
| W                                                                                                                                                    | X | Y      | Z  | MB/FU  | GAUSS | -50-200 | SQUARE |
| 38                                                                                                                                                   | 2 | 0      | 60 | 16.73  | 7528  | -.013   | .065   |
| 28                                                                                                                                                   | 2 | 0      | 70 | 16.54  | 7444  | -.007   | .023   |
| 18                                                                                                                                                   | 2 | 0      | 80 | 16.36  | 7361  | -.001   | .001   |
| 8                                                                                                                                                    | 2 | 0      | 90 | 16.17  | 7278  | .005    | .018   |
| 34                                                                                                                                                   | 2 | 4      | 60 | 16.90  | 7604  | -.015   | .088   |
| 24                                                                                                                                                   | 2 | 4      | 70 | 16.71  | 7521  | -.010   | .041   |
| 14                                                                                                                                                   | 2 | 4      | 80 | 16.53  | 7438  | -.004   | .007   |
| 4                                                                                                                                                    | 2 | 4      | 90 | 16.34  | 7355  | .003    | .004   |
| 30                                                                                                                                                   | 2 | 8      | 60 | 17.07  | 7681  | -.018   | .113   |
| 20                                                                                                                                                   | 2 | 8      | 70 | 16.88  | 7598  | -.012   | .062   |
| 10                                                                                                                                                   | 2 | 8      | 80 | 16.70  | 7515  | -.006   | .019   |
| 0                                                                                                                                                    | 2 | 8      | 90 | 16.51  | 7431  | .000    | .000   |
| 26                                                                                                                                                   | 2 | 12     | 60 | 17.24  | 7758  | -.020   | .138   |
| 16                                                                                                                                                   | 2 | 12     | 70 | 17.05  | 7675  | -.014   | .086   |
| 6                                                                                                                                                    | 2 | 12     | 80 | 16.37  | 7591  | -.008   | .037   |
| 22                                                                                                                                                   | 2 | 16     | 60 | 17.41  | 7835  | -.022   | .165   |
| 12                                                                                                                                                   | 2 | 16     | 70 | 17.23  | 7751  | -.016   | .112   |
| 2                                                                                                                                                    | 2 | 16     | 80 | 17.04  | 7668  | -.011   | .059   |
| 18                                                                                                                                                   | 2 | 20     | 60 | 17.58  | 7911  | -.024   | .191   |
| 8                                                                                                                                                    | 2 | 20     | 70 | 17.40  | 7828  | -.019   | .139   |
| 36                                                                                                                                                   | 4 | 0      | 60 | 17.03  | 7663  | -.016   | .101   |
| 26                                                                                                                                                   | 4 | 0      | 70 | 16.84  | 7580  | -.010   | .050   |
| 16                                                                                                                                                   | 4 | 0      | 80 | 16.66  | 7497  | -.004   | .010   |
| 6                                                                                                                                                    | 4 | 0      | 90 | 16.47  | 7414  | .002    | .002   |
| 32                                                                                                                                                   | 4 | 4      | 60 | 17.20  | 7740  | -.018   | .127   |
| 22                                                                                                                                                   | 4 | 4      | 70 | 17.01  | 7657  | -.012   | .073   |
| 12                                                                                                                                                   | 4 | 4      | 80 | 16.83  | 7573  | -.007   | .026   |
| 2                                                                                                                                                    | 4 | 4      | 90 | 16.65  | 7490  | -.001   | .000   |
| 28                                                                                                                                                   | 4 | 8      | 60 | 17.37  | 7817  | -.020   | .154   |
| 18                                                                                                                                                   | 4 | 8      | 70 | 17.19  | 7733  | -.015   | .099   |
| 8                                                                                                                                                    | 4 | 8      | 80 | 17.00  | 7650  | -.009   | .046   |
| 24                                                                                                                                                   | 4 | 12     | 60 | 17.54  | 7893  | -.022   | .181   |
| 14                                                                                                                                                   | 4 | 12     | 70 | 17.36  | 7810  | -.017   | .127   |
| 4                                                                                                                                                    | 4 | 12     | 80 | 17.17  | 7727  | -.011   | .070   |
| 20                                                                                                                                                   | 4 | 16     | 60 | 17.71  | 7970  | -.025   | .209   |

TABLE XXI-continued

| Magnetization and Temperature Coefficient<br>of (NdErTmHo) <sub>2</sub> Fe <sub>14</sub> B Alloys                                                    |    |        |    |        |       |           |        |      |
|------------------------------------------------------------------------------------------------------------------------------------------------------|----|--------|----|--------|-------|-----------|--------|------|
| W % Er <sub>2</sub> Fe <sub>14</sub> B + X % Nd <sub>2</sub> Fe <sub>14</sub> B + Y % Tm <sub>2</sub> Fe <sub>14</sub> B Z %<br>HoFe <sub>14</sub> B |    |        |    |        |       |           |        |      |
| COMPOSITION                                                                                                                                          |    | M(25C) |    | M(25C) |       | ALPHA     | R      |      |
| W                                                                                                                                                    | X  | Y      | Z  | MB/FU  | GAUSS | -50-200   | SQUARE |      |
| 10                                                                                                                                                   | 4  | 16     | 70 | 17.53  | 7887  | -.019     | .155   |      |
| 0                                                                                                                                                    | 4  | 16     | 80 | 17.34  | 7804  | -.014     | .097   |      |
| 10                                                                                                                                                   | 16 | 4      | 20 | 17.88  | 8047  | -.027     | .236   |      |
| 6                                                                                                                                                    | 4  | 20     | 70 | 17.70  | 7964  | -.021     | .184   |      |
| 34                                                                                                                                                   | 6  | 0      | 60 | 17.33  | 7799  | -.019     | .143   |      |
| 24                                                                                                                                                   | 6  | 0      | 70 | 17.15  | 7715  | -.013     | .086   |      |
| 14                                                                                                                                                   | 6  | 0      | 80 | 16.96  | 7632  | -.007     | .033   |      |
| 4                                                                                                                                                    | 6  | 0      | 90 | 16.78  | 7549  | -.001     | .002   |      |
| 15                                                                                                                                                   | 30 | 6      | 4  | 60     | 17.50 | 7875      | -.021  | .171 |
| 20                                                                                                                                                   | 6  | 4      | 70 | 17.32  | 7792  | -.015     | .114   |      |
| 10                                                                                                                                                   | 6  | 4      | 80 | 17.13  | 7709  | -.010     | .056   |      |
| 0                                                                                                                                                    | 6  | 4      | 90 | 16.95  | 7626  | -.004     | .011   |      |
| 26                                                                                                                                                   | 6  | 8      | 60 | 17.67  | 7952  | -.023     | .200   |      |
| 16                                                                                                                                                   | 6  | 8      | 70 | 17.49  | 7869  | -.018     | .143   |      |
| 22                                                                                                                                                   | 6  | 12     | 60 | 17.84  | 8029  | -.025     | .228   |      |
| 12                                                                                                                                                   | 6  | 12     | 70 | 17.66  | 7946  | -.020     | .173   |      |
| 2                                                                                                                                                    | 6  | 12     | 80 | 17.47  | 7863  | -.014     | .113   |      |
| 18                                                                                                                                                   | 6  | 16     | 60 | 18.01  | 8106  | -.027     | .255   |      |
| 8                                                                                                                                                    | 6  | 16     | 70 | 17.83  | 8023  | -.022     | .203   |      |
| 25                                                                                                                                                   | 14 | 6      | 20 | 60     | 18.18 | 8183      | -.029  | .282 |
| 4                                                                                                                                                    | 6  | 20     | 70 | 18.00  | 8099  | -.024     | .233   |      |
| 32                                                                                                                                                   | 8  | 0      | 60 | 17.63  | 7934  | -.021     | .190   |      |
| 22                                                                                                                                                   | 8  | 0      | 70 | 17.45  | 7851  | -.016     | .130   |      |
| 12                                                                                                                                                   | 8  | 0      | 80 | 17.26  | 7768  | -.010     | .069   |      |
| 6                                                                                                                                                    | 8  | 16     | 70 | 17.08  | 7685  | -.005     | .017   |      |
| 30                                                                                                                                                   | 28 | 8      | 4  | 60     | 17.80 | 8011      | -.023  | .219 |
| 18                                                                                                                                                   | 8  | 4      | 70 | 17.62  | 7928  | -.018     | .161   |      |
| 8                                                                                                                                                    | 8  | 4      | 80 | 17.43  | 7845  | -.013     | .098   |      |
| 24                                                                                                                                                   | 8  | 8      | 60 | 17.97  | 8088  | -.026     | .248   |      |
| 14                                                                                                                                                   | 8  | 8      | 70 | 17.79  | 8005  | -.020     | .193   |      |
| 4                                                                                                                                                    | 8  | 8      | 80 | 17.60  | 7921  | -.015     | .130   |      |
| 20                                                                                                                                                   | 8  | 12     | 60 | 18.14  | 8165  | -.028     | .276   |      |
| 10                                                                                                                                                   | 8  | 12     | 70 | 17.96  | 8081  | -.022     | .224   |      |
| 0                                                                                                                                                    | 8  | 12     | 80 | 17.77  | 7998  | -.017     | .163   |      |
| 16                                                                                                                                                   | 8  | 16     | 60 | 18.31  | 8241  | -.029     | .303   |      |
| 6                                                                                                                                                    | 8  | 16     | 70 | 18.13  | 8158  | -.024     | .254   |      |
| 12                                                                                                                                                   | 8  | 20     | 60 | 18.48  | 8318  | -.031     | .329   |      |
| .2                                                                                                                                                   | 8  | 20     | 70 | 18.30  | 8235  | -.026     | .284   |      |
| 30                                                                                                                                                   | 10 | 0      | 60 | 17.93  | 8070  | -.024     | .240   |      |
| 20                                                                                                                                                   | 10 | 0      | 70 | 17.75  | 7987  | -.019     | .181   |      |
| 10                                                                                                                                                   | 10 | 0      | 80 | 17.56  | 7903  | -.013     | .115   |      |
| 0                                                                                                                                                    | 10 | 0      | 90 | 17.38  | 7820  | -.008     | .049   |      |
| 26                                                                                                                                                   | 10 | 4      | 60 | 18.10  | 8147  | -.026     | .269   |      |
| 16                                                                                                                                                   | 10 | 4      | 70 | 17.92  | 8063  | -.021     | .214   |      |
| 6                                                                                                                                                    | 10 | 4      | 80 | 17.73  | 7980  | -.015     | .149   |      |
| 22                                                                                                                                                   | 10 | 8      | 60 | 18.27  | 8223  | -.028     | .298   |      |
| 12                                                                                                                                                   | 10 | 8      | 70 | 18.09  | 8140  | -.023     | .246   |      |
| 2                                                                                                                                                    | 10 | 8      | 80 | 17.90  | 8057  | -.018     | .184   |      |
| 18                                                                                                                                                   | 10 | 12     | 60 | 18.44  | 8300  | -.030     | .325   |      |
| 8                                                                                                                                                    | 10 | 12     | 70 | 18.26  | 8217  | -.025     | .277   |      |
| 14                                                                                                                                                   | 10 | 16     | 60 | 18.62  | 8377  | -.032     | .351   |      |
| 4                                                                                                                                                    | 10 | 16     | 70 | 18.43  | 8294  | -.027     | .307   |      |
| 10                                                                                                                                                   | 10 | 20     | 60 | 18.79  | 8454  | -.034     | .376   |      |
| 0                                                                                                                                                    | 10 | 20     | 70 | 18.60  | 8370  | -.029     | .335   |      |
| 28                                                                                                                                                   | 12 | 0      | 60 | 18.23  | 8205  | -.026     | .292   |      |
| 18                                                                                                                                                   | 12 | 0      | 70 | 18.05  | 8122  | -.021     | .236   |      |
| 8                                                                                                                                                    | 12 | 0      | 80 | 17.86  | 8039  | -.016     | .170   |      |
| 24                                                                                                                                                   | 12 | 4      | 60 | 18.40  | 8282  | -.028     | .321   |      |
| 14                                                                                                                                                   | 12 | 4      | 79 | 18.22  | 8199  | -.023     | .269   |      |
| 4                                                                                                                                                    | 12 | 4      | 80 | 18.04  | 8116  | -.018     | .207   |      |
| 20                                                                                                                                                   | 12 | 8      | 60 | 18.58  | 8359  | -.030     | .348   |      |
| 10                                                                                                                                                   | 12 | 8      | 70 | 18.39  | 8276  | -.025     | .301   |      |
| 0                                                                                                                                                    | 12 | 8      | 80 | 18.21  | 8193  | -.020     | .243   |      |
| 16                                                                                                                                                   | 12 | 12     | 60 | 18.75  | 8436  | -.032     | .374   |      |
| 6                                                                                                                                                    | 12 | 12     | 70 | 18.56  | 8353  | -.027     | .331   |      |
| 12                                                                                                                                                   | 12 | 16     | 60 | 18.92  | 8513  | -.034     | .399   |      |
| 2                                                                                                                                                    | 12 | 16     | 70 | 18.73  | 8429  | -.029</td |        |      |

Tm from 0 to 12%, Er from 0 to 18%, and Ho from 76 to 92%.

TABLE XXIII

| Magnetization and Temperature Coefficient of $(\text{NdTbDyHo})_2 \text{Fe}_{14}\text{B}$ Alloys |   |                                                                                                                                     |    |       |       |        |
|--------------------------------------------------------------------------------------------------|---|-------------------------------------------------------------------------------------------------------------------------------------|----|-------|-------|--------|
| W %                                                                                              |   | $\text{Tb}_2\text{Fe}_{14}\text{B} + \text{X} \% \text{Nd}_2\text{Fe}_{14}\text{B} + \text{Y} \% \text{Dy}_2\text{Fe}_{14}\text{B}$ |    | Z %   |       |        |
| Ho <sub>2</sub> Fe <sub>14</sub> B                                                               |   |                                                                                                                                     |    |       |       |        |
| COMPOSITION                                                                                      |   | M(25C)                                                                                                                              |    | ALPHA |       | R      |
| W                                                                                                | X | Y                                                                                                                                   | Z  | MB/FU | GAUSS | SQUARE |
| 38                                                                                               | 2 | 0                                                                                                                                   | 60 | 15.11 | 6798  | .002   |
| 28                                                                                               | 2 | 0                                                                                                                                   | 70 | 15.35 | 6907  | .005   |
| 18                                                                                               | 2 | 0                                                                                                                                   | 80 | 15.59 | 7016  | .007   |
| 8                                                                                                | 2 | 0                                                                                                                                   | 90 | 15.83 | 7124  | .009   |
| 34                                                                                               | 2 | 4                                                                                                                                   | 60 | 15.11 | 6798  | .003   |
| 24                                                                                               | 2 | 4                                                                                                                                   | 70 | 15.35 | 6907  | .005   |
| 14                                                                                               | 2 | 4                                                                                                                                   | 80 | 15.59 | 7016  | .008   |
| 4                                                                                                | 2 | 4                                                                                                                                   | 90 | 15.83 | 7124  | .010   |
| 30                                                                                               | 2 | 8                                                                                                                                   | 60 | 15.11 | 6798  | .004   |
| 20                                                                                               | 2 | 8                                                                                                                                   | 70 | 15.35 | 6907  | .006   |
| 10                                                                                               | 2 | 8                                                                                                                                   | 80 | 15.59 | 7016  | .008   |
| 0                                                                                                | 2 | 8                                                                                                                                   | 90 | 15.83 | 7124  | .010   |
| 26                                                                                               | 2 | 12                                                                                                                                  | 60 | 15.11 | 6798  | .005   |
| 16                                                                                               | 2 | 12                                                                                                                                  | 70 | 15.35 | 6907  | .007   |
| 6                                                                                                | 2 | 12                                                                                                                                  | 80 | 15.59 | 7016  | .009   |
| 22                                                                                               | 2 | 16                                                                                                                                  | 60 | 15.11 | 6798  | .006   |
| 12                                                                                               | 2 | 16                                                                                                                                  | 70 | 15.35 | 6907  | .008   |
| 2                                                                                                | 2 | 16                                                                                                                                  | 80 | 15.59 | 7016  | .010   |
| 18                                                                                               | 2 | 20                                                                                                                                  | 60 | 15.11 | 6798  | .006   |
| 8                                                                                                | 2 | 20                                                                                                                                  | 70 | 15.35 | 6907  | .009   |
| 36                                                                                               | 4 | 0                                                                                                                                   | 60 | 15.49 | 6972  | -.002  |
| 26                                                                                               | 4 | 0                                                                                                                                   | 70 | 15.74 | 7081  | .000   |
| 16                                                                                               | 4 | 0                                                                                                                                   | 80 | 15.98 | 7190  | .002   |
| 6                                                                                                | 4 | 0                                                                                                                                   | 90 | 16.22 | 7298  | .004   |
| 32                                                                                               | 4 | 4                                                                                                                                   | 60 | 15.49 | 6972  | -.001  |
| 22                                                                                               | 4 | 4                                                                                                                                   | 70 | 15.74 | 7081  | .001   |
| 12                                                                                               | 4 | 4                                                                                                                                   | 80 | 15.98 | 7190  | .003   |
| 2                                                                                                | 4 | 4                                                                                                                                   | 90 | 16.22 | 7298  | .005   |
| 28                                                                                               | 4 | 8                                                                                                                                   | 60 | 15.49 | 6972  | -.000  |
| 18                                                                                               | 4 | 8                                                                                                                                   | 70 | 15.74 | 7081  | .002   |
| 8                                                                                                | 4 | 8                                                                                                                                   | 80 | 15.98 | 7190  | .004   |
| 24                                                                                               | 4 | 12                                                                                                                                  | 60 | 15.49 | 6972  | .000   |
| 14                                                                                               | 4 | 12                                                                                                                                  | 70 | 15.74 | 7081  | .003   |
| 4                                                                                                | 4 | 12                                                                                                                                  | 80 | 15.98 | 7190  | .006   |
| 20                                                                                               | 4 | 16                                                                                                                                  | 60 | 15.49 | 6972  | .001   |
| 10                                                                                               | 4 | 16                                                                                                                                  | 70 | 15.74 | 7081  | .003   |
| 0                                                                                                | 4 | 16                                                                                                                                  | 80 | 15.98 | 7190  | .005   |
| 16                                                                                               | 4 | 20                                                                                                                                  | 60 | 15.49 | 6972  | .002   |
| 6                                                                                                | 4 | 20                                                                                                                                  | 70 | 15.74 | 7081  | .004   |
| 34                                                                                               | 6 | 0                                                                                                                                   | 60 | 15.88 | 7146  | -.006  |
| 24                                                                                               | 6 | 0                                                                                                                                   | 70 | 16.12 | 7255  | -.004  |
| 14                                                                                               | 6 | 0                                                                                                                                   | 80 | 16.36 | 7364  | -.002  |
| 4                                                                                                | 6 | 0                                                                                                                                   | 90 | 16.61 | 7472  | .000   |
| 30                                                                                               | 6 | 4                                                                                                                                   | 60 | 15.88 | 7146  | -.005  |
| 20                                                                                               | 6 | 4                                                                                                                                   | 70 | 16.12 | 7255  | -.003  |
| 10                                                                                               | 6 | 4                                                                                                                                   | 80 | 16.36 | 7364  | -.001  |
| 0                                                                                                | 6 | 4                                                                                                                                   | 90 | 16.61 | 7472  | .001   |
| 26                                                                                               | 6 | 8                                                                                                                                   | 60 | 15.88 | 7146  | -.005  |
| 16                                                                                               | 6 | 8                                                                                                                                   | 70 | 16.12 | 7255  | -.003  |
| 6                                                                                                | 6 | 8                                                                                                                                   | 80 | 16.36 | 7364  | -.000  |
| 22                                                                                               | 6 | 12                                                                                                                                  | 60 | 15.88 | 7146  | -.004  |
| 12                                                                                               | 6 | 12                                                                                                                                  | 70 | 16.12 | 7255  | -.002  |
| 2                                                                                                | 6 | 12                                                                                                                                  | 80 | 16.36 | 7364  | .000   |
| 18                                                                                               | 6 | 16                                                                                                                                  | 60 | 15.88 | 7146  | -.003  |
| 8                                                                                                | 6 | 16                                                                                                                                  | 70 | 16.12 | 7255  | -.001  |
| 14                                                                                               | 6 | 20                                                                                                                                  | 60 | 15.88 | 7146  | -.002  |
| 4                                                                                                | 6 | 20                                                                                                                                  | 70 | 16.12 | 7255  | -.000  |
| 32                                                                                               | 8 | 0                                                                                                                                   | 60 | 16.27 | 7320  | -.000  |
| 22                                                                                               | 8 | 0                                                                                                                                   | 70 | 16.51 | 7429  | -.008  |
| 12                                                                                               | 8 | 0                                                                                                                                   | 80 | 16.75 | 7538  | -.006  |
| 2                                                                                                | 8 | 0                                                                                                                                   | 90 | 16.99 | 7646  | -.004  |
| 28                                                                                               | 8 | 4                                                                                                                                   | 60 | 16.27 | 7320  | -.009  |
| 18                                                                                               | 8 | 4                                                                                                                                   | 70 | 16.51 | 7429  | -.007  |
| 8                                                                                                | 8 | 4                                                                                                                                   | 80 | 16.75 | 7538  | -.005  |
| 24                                                                                               | 8 | 8                                                                                                                                   | 60 | 16.27 | 7320  | -.009  |
| 14                                                                                               | 8 | 8                                                                                                                                   | 70 | 16.51 | 7429  | -.007  |
| 4                                                                                                | 8 | 8                                                                                                                                   | 80 | 16.75 | 7538  | -.004  |
| 20                                                                                               | 8 | 12                                                                                                                                  | 60 | 16.27 | 7320  | -.008  |
| 10                                                                                               | 8 | 12                                                                                                                                  | 70 | 16.51 | 7429  | -.006  |
| 0                                                                                                | 8 | 12                                                                                                                                  | 80 | 16.75 | 7538  | -.004  |
| 16                                                                                               | 8 | 16                                                                                                                                  | 60 | 16.27 | 7320  | -.007  |
| 6                                                                                                | 8 | 16                                                                                                                                  | 70 | 16.51 | 7429  | -.005  |
| 12                                                                                               | 8 | 20                                                                                                                                  | 60 | 16.27 | 7320  | -.007  |

TABLE XXIII-continued

| Magnetization and Temperature Coefficient<br>of $(NdTbDyHo)_2 Fe_{14}B$ Alloys |                                                              |    |    |    |                    |        |         |        |  |
|--------------------------------------------------------------------------------|--------------------------------------------------------------|----|----|----|--------------------|--------|---------|--------|--|
| 5                                                                              | W % $Tb_2Fe_{14}B$ + X % $Nd_2Fe_{14}B$ + Y % $Dy_2Fe_{14}B$ |    |    |    | Z % $Ho_2Fe_{14}B$ |        |         |        |  |
|                                                                                | COMPOSITION                                                  |    |    |    | M(25C)             | M(25C) | ALPHA   | R      |  |
|                                                                                | W                                                            | X  | Y  | Z  | MB/FU              | GAUSS  | -50-200 | SQUARE |  |
| 10                                                                             | 2                                                            | 8  | 20 | 70 | 16.51              | 7429   | -.004   | .018   |  |
|                                                                                | 30                                                           | 10 | 0  | 60 | 16.65              | 7494   | -.014   | .196   |  |
|                                                                                | 20                                                           | 10 | 0  | 70 | 16.89              | 7603   | -.012   | .133   |  |
|                                                                                | 10                                                           | 10 | 0  | 80 | 17.14              | 7711   | -.010   | .084   |  |
|                                                                                | 0                                                            | 10 | 0  | 90 | 17.38              | 7820   | -.008   | .049   |  |
|                                                                                | 26                                                           | 10 | 4  | 60 | 16.65              | 7494   | -.013   | .177   |  |
| 15                                                                             | 16                                                           | 10 | 4  | 70 | 16.89              | 7603   | -.011   | .117   |  |
|                                                                                | 6                                                            | 10 | 4  | 80 | 17.14              | 7711   | -.009   | .072   |  |
|                                                                                | 22                                                           | 10 | 8  | 60 | 16.65              | 7494   | -.013   | .158   |  |
|                                                                                | 12                                                           | 10 | 8  | 70 | 16.89              | 7603   | -.010   | .102   |  |
|                                                                                | 2                                                            | 10 | 8  | 80 | 17.14              | 7711   | -.008   | .061   |  |
|                                                                                | 18                                                           | 10 | 12 | 60 | 16.65              | 7494   | -.012   | .140   |  |
| 20                                                                             | 8                                                            | 10 | 12 | 70 | 16.89              | 7603   | -.010   | .088   |  |
|                                                                                | 14                                                           | 10 | 16 | 60 | 16.65              | 7494   | -.011   | .123   |  |
|                                                                                | 4                                                            | 10 | 16 | 70 | 16.89              | 7603   | -.009   | .075   |  |
|                                                                                | 10                                                           | 10 | 20 | 60 | 16.65              | 7494   | -.010   | .108   |  |
|                                                                                | 0                                                            | 10 | 20 | 70 | 16.89              | 7603   | -.008   | .064   |  |
|                                                                                | 28                                                           | 12 | 0  | 60 | 17.04              | 7668   | -.018   | .282   |  |
| 25                                                                             | 18                                                           | 12 | 0  | 70 | 17.28              | 7777   | -.015   | .211   |  |
|                                                                                | 8                                                            | 12 | 0  | 80 | 17.52              | 7885   | -.013   | .151   |  |
|                                                                                | 24                                                           | 12 | 4  | 60 | 17.04              | 7668   | -.017   | .261   |  |
|                                                                                | 14                                                           | 12 | 4  | 70 | 17.28              | 7777   | -.015   | .192   |  |
|                                                                                | 4                                                            | 12 | 4  | 80 | 17.52              | 7885   | -.013   | .135   |  |
|                                                                                | 20                                                           | 12 | 8  | 60 | 17.04              | 7668   | -.016   | .241   |  |
| 30                                                                             | 10                                                           | 12 | 8  | 70 | 17.28              | 7777   | -.014   | .175   |  |
|                                                                                | 0                                                            | 12 | 8  | 80 | 17.52              | 7885   | -.012   | .121   |  |
|                                                                                | 16                                                           | 12 | 12 | 60 | 17.04              | 7668   | -.015   | .221   |  |
|                                                                                | 6                                                            | 12 | 12 | 70 | 17.28              | 7777   | -.013   | .158   |  |
|                                                                                | 12                                                           | 12 | 16 | 60 | 17.04              | 7668   | -.015   | .202   |  |
|                                                                                | 2                                                            | 12 | 16 | 70 | 17.28              | 7777   | -.013   | .142   |  |
|                                                                                | 8                                                            | 12 | 20 | 60 | 17.04              | 7668   | -.014   | .184   |  |

35 Table XXIII shows alloys wherein the Nd is combined with Tb, Dy and Ho. The desired combination of properties is achieved if Nd varies from 9 to 11, Dy varies from 0 to 15, Tb from 0 to 12 and Ho is within the range from 75 to 88%.

TABLE XXV

| Magnetization and Temperature Coefficient<br>of $(NdGdDyHo)_2Fe_{14}B$ Alloys |                                                                                 |   |    |        |        |       |         |        |
|-------------------------------------------------------------------------------|---------------------------------------------------------------------------------|---|----|--------|--------|-------|---------|--------|
|                                                                               | W % $Gd_2Fe_{14}B$ + X % $Nd_2Fe_{14}B$ + Y % $Dy_2Fe_{14}B$ + Z % $HoFe_{14}B$ |   |    |        |        |       |         |        |
| 45                                                                            | COMPOSITION                                                                     |   |    | M(25C) | M(25C) | ALPHA | R       |        |
|                                                                               | W                                                                               | X | Y  | Z      | MB/FU  | GAUSS | -50-200 | SQUARE |
| 50                                                                            | 38                                                                              | 2 | 0  | 60     | 16.36  | 7361  | -.017   | .230   |
|                                                                               | 28                                                                              | 2 | 0  | 70     | 16.27  | 7322  | -.010   | .085   |
|                                                                               | 18                                                                              | 2 | 0  | 80     | 16.18  | 7282  | -.003   | .006   |
|                                                                               | 8                                                                               | 2 | 0  | 90     | 16.10  | 7243  | .005    | .016   |
|                                                                               | 34                                                                              | 2 | 4  | 60     | 16.23  | 7302  | -.014   | .174   |
|                                                                               | 24                                                                              | 2 | 4  | 70     | 16.14  | 7263  | -.007   | .046   |
|                                                                               | 14                                                                              | 2 | 4  | 80     | 16.05  | 7223  | .000    | .000   |
|                                                                               | 4                                                                               | 2 | 4  | 90     | 15.96  | 7184  | .007    | .042   |
| 55                                                                            | 30                                                                              | 2 | 8  | 60     | 16.10  | 7243  | -.012   | .121   |
|                                                                               | 20                                                                              | 2 | 8  | 70     | 16.01  | 7203  | -.004   | .018   |
|                                                                               | 10                                                                              | 2 | 8  | 80     | 15.92  | 7164  | .003    | .007   |
|                                                                               | 0                                                                               | 2 | 8  | 90     | 15.83  | 7124  | .010    | .077   |
|                                                                               | 26                                                                              | 2 | 12 | 60     | 15.96  | 7183  | -.009   | .074   |
|                                                                               | 16                                                                              | 2 | 12 | 70     | 15.88  | 7144  | -.002   | .002   |
|                                                                               | 6                                                                               | 2 | 12 | 80     | 15.79  | 7105  | .006    | .027   |
|                                                                               | 22                                                                              | 2 | 16 | 60     | 15.83  | 7124  | -.006   | .036   |
| 60                                                                            | 12                                                                              | 2 | 16 | 70     | 15.74  | 7085  | .001    | .001   |
|                                                                               | 2                                                                               | 2 | 16 | 80     | 15.66  | 7045  | .009    | .060   |
|                                                                               | 18                                                                              | 2 | 20 | 60     | 15.70  | 7065  | -.003   | .011   |
|                                                                               | 8                                                                               | 2 | 20 | 70     | 15.61  | 7025  | .004    | .015   |
|                                                                               | 36                                                                              | 4 | 0  | 60     | 16.68  | 7506  | -.019   | .292   |
|                                                                               | 26                                                                              | 4 | 0  | 70     | 16.59  | 7466  | -.013   | .137   |
|                                                                               | 16                                                                              | 4 | 0  | 80     | 16.50  | 7427  | -.006   | .029   |
|                                                                               | 6                                                                               | 4 | 0  | 90     | 16.42  | 7387  | .001    | .001   |
| 65                                                                            | 32                                                                              | 4 | 4  | 60     | 16.55  | 7446  | -.017   | .236   |
|                                                                               | 22                                                                              | 4 | 4  | 70     | 16.46  | 7407  | -.010   | .090   |
|                                                                               | 12                                                                              | 4 | 4  | 80     | 16.37  | 7367  | -.003   | .008   |

TABLE XXV-continued

| Magnetization and Temperature Coefficient of $(\text{NdGdDyHo})_2 \text{Fe}_{14}\text{B}$ Alloys                                                             |    |    |    |             |        |         |
|--------------------------------------------------------------------------------------------------------------------------------------------------------------|----|----|----|-------------|--------|---------|
| W % $\text{Gd}_2\text{Fe}_{14}\text{B}$ + X % $\text{Nd}_2\text{Fe}_{14}\text{B}$ + Y % $\text{Dy}_2\text{Fe}_{14}\text{B}$ + Z % $\text{HoFe}_{14}\text{B}$ |    |    |    | COMPOSITION |        |         |
| W                                                                                                                                                            | X  | Y  | Z  | M(25C)      | M(25C) | ALPHA   |
|                                                                                                                                                              |    |    |    | MB/FU       | GAUSS  | -50-200 |
|                                                                                                                                                              |    |    |    |             |        | SQUARE  |
| 2                                                                                                                                                            | 4  | 4  | 90 | 16.28       | 7328   | .004    |
| 28                                                                                                                                                           | 4  | 8  | 60 | 16.42       | 7387   | -.014   |
| 18                                                                                                                                                           | 4  | 8  | 70 | 16.33       | 7348   | -.007   |
| 8                                                                                                                                                            | 4  | 8  | 80 | 16.24       | 7308   | -.000   |
| 24                                                                                                                                                           | 4  | 12 | 60 | 16.28       | 7328   | -.012   |
| 14                                                                                                                                                           | 4  | 12 | 70 | 16.20       | 7288   | -.005   |
| 4                                                                                                                                                            | 4  | 12 | 80 | 16.11       | 7249   | .002    |
| 20                                                                                                                                                           | 4  | 16 | 60 | 16.15       | 7268   | -.009   |
| 10                                                                                                                                                           | 4  | 16 | 70 | 16.06       | 7229   | -.002   |
| 0                                                                                                                                                            | 4  | 16 | 80 | 15.98       | 7190   | .005    |
| 16                                                                                                                                                           | 4  | 20 | 60 | 16.02       | 7209   | -.006   |
| 6                                                                                                                                                            | 4  | 20 | 70 | 15.93       | 7170   | .001    |
| 34                                                                                                                                                           | 6  | 0  | 60 | 17.00       | 7650   | -.022   |
| 24                                                                                                                                                           | 6  | 0  | 70 | 16.91       | 7611   | -.015   |
| 14                                                                                                                                                           | 6  | 0  | 80 | 16.82       | 7571   | -.009   |
| 4                                                                                                                                                            | 6  | 0  | 90 | 16.74       | 7532   | -.002   |
| 30                                                                                                                                                           | 6  | 4  | 60 | 16.87       | 7591   | -.020   |
| 20                                                                                                                                                           | 6  | 4  | 70 | 16.78       | 7551   | -.013   |
| 10                                                                                                                                                           | 6  | 4  | 80 | 16.69       | 7512   | -.006   |
| 0                                                                                                                                                            | 6  | 4  | 90 | 16.61       | 7472   | .001    |
| 26                                                                                                                                                           | 6  | 8  | 60 | 16.74       | 7531   | -.017   |
| 16                                                                                                                                                           | 6  | 8  | 70 | 16.65       | 7492   | -.010   |
| 6                                                                                                                                                            | 6  | 8  | 80 | 16.56       | 7452   | -.003   |
| 22                                                                                                                                                           | 6  | 12 | 60 | 16.60       | 7472   | -.015   |
| 12                                                                                                                                                           | 6  | 12 | 70 | 16.52       | 7433   | -.008   |
| 2                                                                                                                                                            | 6  | 12 | 80 | 16.43       | 7393   | -.001   |
| 18                                                                                                                                                           | 6  | 16 | 60 | 16.47       | 7413   | -.012   |
| 8                                                                                                                                                            | 6  | 16 | 70 | 16.39       | 7373   | -.005   |
| 14                                                                                                                                                           | 6  | 20 | 60 | 16.34       | 7354   | -.009   |
| 4                                                                                                                                                            | 6  | 20 | 70 | 16.25       | 7314   | -.002   |
| 32                                                                                                                                                           | 8  | 0  | 60 | 17.32       | 7794   | -.024   |
| 22                                                                                                                                                           | 8  | 0  | 70 | 17.23       | 7755   | -.018   |
| 12                                                                                                                                                           | 8  | 0  | 80 | 17.15       | 7715   | -.011   |
| 2                                                                                                                                                            | 8  | 0  | 90 | 17.06       | 7676   | -.005   |
| 28                                                                                                                                                           | 8  | 4  | 60 | 17.19       | 7735   | -.022   |
| 18                                                                                                                                                           | 8  | 4  | 70 | 17.10       | 7696   | -.016   |
| 8                                                                                                                                                            | 8  | 4  | 80 | 17.01       | 7656   | -.009   |
| 24                                                                                                                                                           | 8  | 8  | 60 | 17.06       | 7676   | -.020   |
| 14                                                                                                                                                           | 8  | 8  | 70 | 16.97       | 7636   | -.013   |
| 4                                                                                                                                                            | 8  | 8  | 80 | 16.88       | 7597   | -.066   |
| 20                                                                                                                                                           | 8  | 12 | 60 | 16.93       | 7616   | -.017   |
| 10                                                                                                                                                           | 8  | 12 | 70 | 16.84       | 7577   | -.011   |
| 0                                                                                                                                                            | 8  | 12 | 80 | 16.75       | 7538   | -.004   |
| 16                                                                                                                                                           | 8  | 16 | 60 | 16.79       | 7557   | -.015   |
| 6                                                                                                                                                            | 8  | 16 | 70 | 16.71       | 7518   | -.008   |
| 12                                                                                                                                                           | 8  | 20 | 60 | 16.66       | 7498   | -.012   |
| 2                                                                                                                                                            | 8  | 20 | 70 | 16.57       | 7458   | -.005   |
| 30                                                                                                                                                           | 10 | 0  | 60 | 17.64       | 7939   | -.027   |
| 20                                                                                                                                                           | 10 | 0  | 70 | 17.55       | 7899   | -.021   |
| 10                                                                                                                                                           | 10 | 0  | 80 | 17.47       | 7860   | -.014   |
| 0                                                                                                                                                            | 10 | 0  | 90 | 17.38       | 7820   | -.008   |
| 26                                                                                                                                                           | 10 | 4  | 60 | 17.51       | 7879   | -.025   |
| 16                                                                                                                                                           | 10 | 4  | 70 | 17.42       | 7840   | -.018   |
| 6                                                                                                                                                            | 10 | 4  | 80 | 17.33       | 7800   | -.012   |
| 22                                                                                                                                                           | 10 | 8  | 60 | 17.38       | 7820   | -.022   |
| 12                                                                                                                                                           | 10 | 8  | 70 | 17.29       | 7781   | -.016   |
| 2                                                                                                                                                            | 10 | 8  | 80 | 17.20       | 7741   | -.009   |
| 18                                                                                                                                                           | 10 | 12 | 60 | 17.25       | 7761   | -.020   |
| 8                                                                                                                                                            | 10 | 12 | 70 | 17.16       | 7721   | -.013   |
| 14                                                                                                                                                           | 10 | 16 | 60 | 17.11       | 7701   | -.017   |
| 4                                                                                                                                                            | 10 | 16 | 70 | 17.03       | 7662   | -.011   |
| 10                                                                                                                                                           | 10 | 20 | 60 | 16.98       | 7642   | -.015   |
| 0                                                                                                                                                            | 10 | 20 | 70 | 16.89       | 7603   | -.008   |
| 28                                                                                                                                                           | 12 | 0  | 60 | 17.96       | 8083   | -.029   |
| 18                                                                                                                                                           | 12 | 0  | 70 | 17.87       | 8043   | -.023   |
| 8                                                                                                                                                            | 12 | 0  | 80 | 17.79       | 8004   | -.017   |
| 24                                                                                                                                                           | 12 | 4  | 60 | 17.83       | 8024   | -.277   |
| 14                                                                                                                                                           | 12 | 4  | 70 | 17.74       | 7984   | -.021   |
| 4                                                                                                                                                            | 12 | 4  | 80 | 17.65       | 7945   | -.014   |
| 20                                                                                                                                                           | 12 | 8  | 60 | 17.70       | 7964   | -.025   |
| 10                                                                                                                                                           | 12 | 8  | 70 | 17.61       | 7925   | -.018   |
| 0                                                                                                                                                            | 12 | 8  | 80 | 17.52       | 7885   | -.012   |
| 16                                                                                                                                                           | 12 | 12 | 60 | 17.57       | 7905   | -.022   |
| 6                                                                                                                                                            | 12 | 12 | 70 | 17.48       | 7866   | -.016   |
| 12                                                                                                                                                           | 12 | 16 | 60 | 17.44       | 7846   | -.020   |

TABLE XXV-continued

| Magnetization and Temperature Coefficient of $(\text{NdGdDyHo})_2 \text{Fe}_{14}\text{B}$ Alloys                                                             |    |    |    |             |        |         |
|--------------------------------------------------------------------------------------------------------------------------------------------------------------|----|----|----|-------------|--------|---------|
| W % $\text{Gd}_2\text{Fe}_{14}\text{B}$ + X % $\text{Nd}_2\text{Fe}_{14}\text{B}$ + Y % $\text{Dy}_2\text{Fe}_{14}\text{B}$ + Z % $\text{HoFe}_{14}\text{B}$ |    |    |    | COMPOSITION |        |         |
| W                                                                                                                                                            | X  | Y  | Z  | M(25C)      | M(25C) | ALPHA   |
|                                                                                                                                                              |    |    |    | MB/FU       | GAUSS  | -50-200 |
|                                                                                                                                                              |    |    |    |             |        | SQUARE  |
| 2                                                                                                                                                            | 12 | 16 | 70 | 17.35       | 7806   | -.014   |
| 8                                                                                                                                                            | 12 | 20 | 60 | 17.30       | 7786   | -.018   |

Table XXV shows alloy compositions of Nd with Gd, Dy and Ho if Nd varies from 8 to 12%, Dy from 0 to 15%, Gd from 0 to 8%, and Ho is within the range from 72 to 88%, the alloys exhibit the desired combination of properties.

What is claimed is:

1. A permanent magnet alloy consisting essentially of  $\text{R}_2\text{Fe}_{14}\text{B}$ , wherein R is a combination of rare earth elements consisting essentially of, in atomic percent, Nd 3 to 11 and balance Ho, said alloy exhibiting in combination  $\alpha$  less than  $-0.01\%$  per  $^{\circ}\text{C}$ . over the temperature range of  $-50^{\circ}\text{C}$ . to  $250^{\circ}\text{C}$ . and  $M_s$  greater than 7500 Gauss at room temperature.
2. The alloy of claim 1 wherein R includes up to 10% Gd.
3. The alloy of claim 1 wherein R includes up to 15% Tb.
4. The alloy of claim 1 wherein R includes up to 10% Dy.
5. The alloy of claim 1 wherein R includes up to 18% Er.
6. The alloy of claim 1 wherein R includes up to 12% Tm.
7. A permanent magnet alloy consisting essentially of  $\text{R}_2\text{Fe}_{14}\text{B}$ , wherein R is a combination of rare earth elements consisting essentially of, in atomic percent, Nd 3 to 11, at least one optional heavy rare earth element selected from the group consisting of Gd up to 10, Tb up to 15, Dy up to 16, Er up to 18 and Tm up to 12 and balance Ho, said alloy exhibiting in combination  $\alpha$  less than  $-0.01\%$  per  $^{\circ}\text{C}$ . over the temperature range of  $-50^{\circ}\text{C}$ . to  $250^{\circ}\text{C}$ . and  $M_s$  greater than 7500 Gauss at room temperature.
8. The alloy of claim 1, or claim 2, or claim 3, or claim 4, or claim 5, or claim 6 or claim 7 wherein Ho is 75 to 92%.
9. A permanent magnet alloy consisting essentially of  $\text{R}_2\text{Fe}_{14}\text{B}$ , wherein R is a combination of rare elements consisting essentially of, in atomic percent, Nd 4 to 10, Tm 0 to 13 and Ho 83 to 96, said alloy exhibiting in combination alpha less than  $-0.01\%$  per  $^{\circ}\text{C}$ . over the temperature range of  $-50^{\circ}\text{C}$ . to  $250^{\circ}\text{C}$ . and  $M_s$  greater than 7500 Gauss at room temperature.
10. A permanent magnet alloy consisting essentially of  $\text{R}_2\text{Fe}_{14}\text{B}$  wherein R is a combination of rare earth elements consisting essentially of, in atomic percent, Nd 5 to 11, Er 0 to 18, Ho 76 to 94, said alloy exhibiting in combination alpha less than  $-0.01\%$  per  $^{\circ}\text{C}$ . over the temperature range of  $-50^{\circ}\text{C}$ . to  $250^{\circ}\text{C}$ . and  $M_s$  greater than 7500 Gauss at room temperature.
11. A permanent magnet alloy consisting essentially of  $\text{R}_2\text{Fe}_{14}\text{B}$  wherein R is a combination of rare earth elements consisting essentially of, in atomic percent, Nd 7 to 11, Tb 9 to 12 and Ho 78 to 90, said alloy exhibiting in combination alpha less than  $-0.01\%$  per  $^{\circ}\text{C}$ . over the temperature range of  $-50^{\circ}\text{C}$ . to  $250^{\circ}\text{C}$ . and  $M_s$  greater than 7500 Gauss at room temperature.

12. A permanent magnet alloy consisting essentially of  $R_2Fe_{14}B$  wherein R is a combination of rare earth elements consisting essentially of, atomic percent Nd 7 to 11, Dy 0 to 15 and Ho 75 to 90, said alloy exhibiting in combination alpha less than  $-0.01\%$  per  $^{\circ}C$ . over the temperature range of  $-50^{\circ}C$ . to  $250^{\circ}C$ . and  $M_s$  greater than 7500 Gauss at room temperature.

13. A permanent magnet alloy consisting essentially of  $R_2Fe_{14}B$  wherein R is a combination of a rare earth elements consisting essentially of, in atomic percent, Nd 7 to 11, Gd 0 to 10, and Ho 82 to 92, said alloy exhibiting in combination alpha less than  $-0.01\%$  per  $^{\circ}C$ . over the temperature range of  $-50^{\circ}C$ . to  $250^{\circ}C$ . and  $M_s$  greater than 7500 Gauss at room temperature.

14. A permanent magnet alloy consisting essentially of  $R_2Fe_{14}B$  wherein R is a combination of rare earth elements consisting essentially of, in atomic percent, Nd 7 to 11, Gd 0 to 10, and Ho 82 to 92, said alloy exhibiting in combination alpha less than  $-0.01\%$  per  $^{\circ}C$ . over the temperature range of  $-50^{\circ}C$ . to  $250^{\circ}C$ . and  $M_s$  greater than 7500 Gauss at room temperature.

15. A permanent magnet alloy consisting essentially of  $R_2Fe_{14}B$  wherein R is a combination of rare earth elements consisting essentially of, in atomic percent, Nd 6 to 10, Dy 0 to 8, Er 0 to 14, Ho 76 to 96, said alloy 25

exhibiting in combination alpha less than  $-0.01\%$  per  $^{\circ}C$ . over the temperature range of  $-50^{\circ}C$ . to  $250^{\circ}C$ . and  $M_s$  greater than 7500 Gauss at room temperature.

16. A permanent magnet alloy consisting essentially of  $R_2Fe_{14}B$  wherein R is a combination of rare earth elements consisting essentially of, in atomic percent, Nd 3 to 11, Tm 0 to 12, Er 0 to 18, and Ho 76 to 92, said alloy exhibiting in combination alpha less than  $-0.01\%$  per  $^{\circ}C$ . over the temperature range of  $-50^{\circ}C$ . to  $250^{\circ}C$ . and  $M_s$  greater than 7500 Gauss at room temperature.

17. A permanent magnet alloy consisting essentially of  $R_2Fe_{14}B$  wherein R is a combination of rare earth elements consisting essentially of, in atomic percent, Nd 9 to 11, Dy 9 to 15, Tb 0 to 12, and Ho 75 to 88, said alloy exhibiting in combination alpha less than  $-0.01\%$  per  $^{\circ}C$ . over the temperature range of  $-50^{\circ}C$ . to  $250^{\circ}C$ . and  $M_s$  greater than 7500 Gauss at room temperature.

18. A permanent magnet alloy consisting essentially of  $R_2Fe_{14}B$  wherein R is a combination of rare earth elements consisting essentially of, in atomic percent, Nd 8 to 12, Dy 0 to 15, Gd 0 to 8, and Ho 72 to 88, said alloy exhibiting in combination alpha less than  $-0.01\%$  per  $^{\circ}C$ . over the temperature range of  $-50^{\circ}C$ . to  $250^{\circ}C$ . and  $M_s$  greater than 7500 Gauss at room temperature.

\* \* \* \* \*